



US006291144B1

(12) **United States Patent**  
**Aylward et al.**

(10) **Patent No.:** **US 6,291,144 B1**  
(b4) **Date of Patent:** **Sep. 18, 2001**

(54) **DAY/NIGHT IMAGING MEMBER WITH EXPANDED COLOR GAMUT**

(75) Inventors: **Peter T. Aylward**, Hilton; **Robert P. Bourdelais**, Pittsford; **James L. Edwards**; **Alphonse D. Camp**, both of Rochester, all of NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/664,517**

(22) Filed: **Sep. 18, 2000**

(51) **Int. Cl.<sup>7</sup>** ..... **G03C 7/18**; G03C 7/22; G03C 7/26; G03C 7/30

(52) **U.S. Cl.** ..... **430/359**; 430/364; 430/363; 430/383; 430/504; 430/506; 430/508

(58) **Field of Search** ..... 430/504, 506, 430/508, 359, 364, 533, 536, 503, 363, 383

(56) **References Cited**

U.S. PATENT DOCUMENTS

- |           |   |         |                  |       |          |
|-----------|---|---------|------------------|-------|----------|
| 2,927,024 | * | 3/1960  | Woodward et al.  | ..... | 430/506  |
| 4,705,745 | * | 11/1987 | Kitchen et al.   | ..... | 430/508  |
| 4,746,599 |   | 5/1988  | Deguchi et al.   | ..... | 430/504  |
| 4,816,378 | * | 3/1989  | Powers et al.    | ..... | 430/508  |
| 5,436,116 |   | 7/1995  | Hoshino et al.   | ..... | 430/505  |
| 5,437,969 |   | 8/1995  | Schmuck et al.   | ..... | 430/504  |
| 5,445,928 |   | 8/1995  | Schmuck et al.   | ..... | 430/504  |
| 5,447,831 |   | 9/1995  | Singer et al.    | ..... | 430/504  |
| 5,455,150 |   | 10/1995 | Mooberry et al.  | ..... | 430/504  |
| 5,486,450 |   | 1/1996  | Tosaka et al.    | ..... | 430/538  |
| 5,563,026 |   | 10/1996 | Singer           | ..... | 430/504  |
| 5,679,139 |   | 10/1997 | McInerney et al. | ..... | 106/20 D |

- |           |   |         |                   |       |          |
|-----------|---|---------|-------------------|-------|----------|
| 5,679,140 |   | 10/1997 | McInerney et al.  | ..... | 106/20 D |
| 5,679,141 |   | 10/1997 | McInerney et al.  | ..... | 106/20 D |
| 5,679,142 |   | 10/1997 | McInerney et al.  | ..... | 106/20 D |
| 5,723,263 |   | 3/1998  | Singer et al.     | ..... | 430/374  |
| 5,866,282 |   | 2/1999  | Bourdelaïs et al. | ..... | 430/536  |
| 6,017,685 | * | 1/2000  | Bourdelaïs et al. | ..... | 430/536  |
| 6,030,742 |   | 2/2000  | Bourdelaïs et al. | ..... | 430/207  |
| 6,030,756 | * | 2/2000  | Bourdelaïs et al. | ..... | 430/533  |
| 6,071,654 | * | 6/2000  | Camp et al.       | ..... | 430/533  |
| 6,080,532 |   | 6/2000  | Camp et al.       | ..... | 430/536  |
| 6,083,669 | * | 7/2000  | Bourdelaïs et al. | ..... | 430/533  |
| 6,093,521 | * | 7/2000  | Laney et al.      | ..... | 430/533  |
| 6,153,351 |   | 11/2000 | Gula et al.       | ..... | 430/536  |
| 6,159,674 |   | 12/2000 | Edwards           | ..... | 430/383  |

FOREIGN PATENT DOCUMENTS

- |              |  |        |        |
|--------------|--|--------|--------|
| 0 825 488 A1 |  | 2/1998 | (EP) . |
| 0 915 374 A1 |  | 5/1999 | (EP) . |

\* cited by examiner

Primary Examiner—Richard L. Schilling

(74) Attorney, Agent, or Firm—Paul A. Leipold

(57) **ABSTRACT**

This invention relates to an imaging element comprising a translucent polymer sheet, and at least three photosensitive dye forming coupler containing layers on the face side of said sheet, wherein said at least three photosensitive forming coupler containing layers comprise a cyan dye forming layer comprising a cyan dye forming coupler in combination with a red sensitized photosensitive emulsion, a yellow dye forming layer comprising a yellow dye forming coupler in combination with a blue light sensitive photosensitive emulsion, a magenta dye forming layer comprising a magenta dye forming coupler and a green light sensitive photosensitive emulsion, and on the backside of said translucent polymer sheet at least one dye forming coupler that forms at least one dye that is spectrally distinct from the dyes on the face side of said translucent sheet.

**17 Claims, 2 Drawing Sheets**







FIG. 3

## DAY/NIGHT IMAGING MEMBER WITH EXPANDED COLOR GAMUT

## FIELD OF THE INVENTION

This invention relates to an improved silver halide display element. More specifically, it relates to a preferred display element comprising at least five separately sensitized light-sensitive silver halide emulsion layers containing, in addition to the three conventional cyan, magenta, and yellow dye-forming layers, a fourth image dye-forming layer comprising a coupler wherein the dye formed by that coupler has a CIELAB  $h_{ab}$  hue angle in the range of from not less than 355° to not more than 75°, and a fifth image dye-forming layer comprising a coupler wherein the dye formed by that coupler has a hue angle in the range of from not less than 225° to not more than 310°, which increases the gamut of colors possible

## BACKGROUND OF THE INVENTION

It is known in the art that photographic display materials are utilized for advertising, as well as decorative displays of photographic images. Since these display materials are used in advertising, the image quality of the display material is critical in expressing the quality message of the product or service being advertised. Further, a photographic display image needs to be high impact, as it attempts to draw consumer attention to the display material and the desired message being conveyed. Typical applications for display material include product and service advertising in public places such as airports, buses and sports stadiums, movie posters and fine art photography. The desired attributes of a quality, high impact photographic display material are a slight blue density minimum, durability, sharpness and flatness. Cost is also important as display materials tend to be expensive compared with alternative display material technology mainly lithographic images on paper. For display materials, traditional color paper is undesirable as it suffers from a lack of durability for the handling, photoprocessing and display of large format images.

Prior art silver halide display materials typically utilize yellow, magenta and cyan dyes to create an image. In a typical yellow, magenta and cyan imaging system the color gamut is limited compared to printing of color inks. Color gamut is an important feature of color printing and imaging systems. It is a measure of the range of colors that can be produced using a given combination of colorants. It is desirable for the color gamut to be as large as possible. The color gamut of the imaging system is controlled primarily by the absorption characteristics of the set of colorants used to produce the image. Silver halide imaging systems typically employ three colorants, typically including cyan, magenta, and yellow in the conventional subtractive imaging system

The ability to produce an image containing any particular color is limited by the color gamut of the system and materials used to produce the image. Thus, the range of colors available for image reproduction is limited by the color gamut that the system and materials can produce.

Color gamut is often thought to be maximized by the use of so-called "block dyes". In *The Reproduction of Color* 4th ed., R. W. G. Hunt, pp 135-144, it has been suggested that the optimum gamut could be obtained with a subtractive three-color system using three theoretical block dyes where the blocks are separated at approximately 490 nm and 580 nm. This proposal is interesting but cannot be implemented for various reasons. In particular, there are no real organic based couplers, which produce dyes corresponding to the proposed block dyes.

Variations in the block dye concept are advanced by Clarkson, M. E. and Vickerstaff, T. in "Brightness and Hue of Present-Day Dyes in Relation to Color Photography," Photo. J. 88b, 26 (1948). Three example spectral shapes are given by Clarkson and Vickerstaff: Block, Trapezoidal, and Triangular. The authors conclude, contrary to the teachings of Hunt, that trapezoidal absorption spectra may be preferred to a vertical sided block dye. Again, dyes having these trapezoidal spectra shapes are theoretical and are not available in practice.

Both commercially available dyes and theoretical dyes were investigated in "The Color Gamut Obtainable by the Combination of Subtractive Color Dyes. Optimum Absorption Bands as Defined by Nonlinear Optimization Technique," J. Imaging Science, 30, 9-12. The author, N. Ohta, deals with the subject of real colorants and notes that the existing curve for a typical cyan dye, as shown in the publication, is the optimum absorption curve for cyan dyes from a gamut standpoint.

20 Bourdelais et al in U.S. Pat. No. 6,030,756 discusses imaging layers containing silver halide and dye forming couplers applied to both sides of a translucent base for a display material. While the display material in U.S. Pat. No. 6,030,756 provides an excellent image that can be displayed 25 without the need for a backlight source, the image is only capable of reproducing 56% of Pantone color space.

McInerney et al in U.S. Pat. Nos. 5,679,139; 5,679,140; 5,679,141; and 5,679,142 teach the shape of preferred 30 subtractive dye absorption shapes for use in four color, C,M,Y,K based ink-jet prints.

McInerney et al in EP 0 825 488 teaches the shape of preferred subtractive cyan dye absorption shape for use in silver halide based color prints.

35 Kitchin et al in U.S. Pat. No. 4,705,745 teaches the preparation of a photographic element for preparing half-tone color proofs comprising four separate imaging layers capable of producing cyan, magenta, yellow, and black images.

40 Powers et al in U.S. Pat. No. 4,816,378 teaches an imaging process for the preparation of color half-tone images that contain cyan, magenta, yellow, and black images. The use of the black dye does little to improve the gamut of color reproduction.

45 Haraga et al in EP 0 915 374 A1 teaches a method for improving image clarity by mixing 'invisible' information in the original scene with a color print and reproducing it as an infrared dye, magenta dye, or as a mixture of cyan magenta and yellow dyes to achieve improved color tone and realism. 50 The addition of the resulting infrared, magenta, or black dye does little to improve the gamut.

In spite of the foregoing teachings relative to color gamut, the coupler sets which have been employed in silver halide color imaging have not provided the range of gamut desired for modern digital imaging; especially for so-called 'spot colors', or 'HiFi colors'.

55 It is, therefore, a problem to be solved by providing a coupler set which provides an increase in color gamut compared to coupler sets comprised of cyan, magenta, and yellow dye forming couplers by further incorporating red dye and blue dye forming couplers.

60 It has been proposed in U.S. Pat. No. 5,866,282 (Bourdelais et al) to utilize a composite support material with laminated biaxially oriented polyolefin sheets as a photographic imaging material. In U.S. Pat. No. 5,866,282, biaxially oriented polyolefin sheets are extrusion laminated

to cellulose paper to create a support for silver halide imaging layers. The biaxially oriented sheets described in U.S. Pat. No. 5,866,282 have a microvoided layer in combination with coextruded layers that contain white pigments such as TiO<sub>2</sub> above and below the microvoided layer. In the composite imaging support structure described in U.S. Pat. No. 5,866,282 the silver halide imaging layers are applied to the white, reflecting side of the base that has a spectral transmission less than 15%.

Prior art photographic display materials historically have been classified as either reflection or transmission. Reflection display material typically is highly pigmented image supports with a light sensitive silver halide coating applied. Reflection display materials are typically used in commercial applications where an image is used to convey an idea or message. An application example of a reflection display material is product advertisement in a public area. Prior art reflection display materials have been optimized to provide a pleasing image using reflective light. Transmission display materials are used in commercial imaging applications and are typically backlit with a light source. Transmission display materials are typically a clear support with a light sensitive silver halide and an incorporated diffuser (to hide the "show through" of the lamps used to provide viewing illumination) or a substantially transparent support coated with a light sensitive silver halide emulsion which requires a diffusing screen to be placed behind the material as a means to obscure the "show through" of the lamps used to provide illumination to the media. Prior art transmission display materials have been optimized to provide a pleasing image when the image is backlit with a variety of light sources. Because prior art reflection and transmission products have been optimized to be either a reflection display image or a transmission display image, two separate product designs must exist in manufacturing, and two inventories of display materials must be maintained at the photofinishing printing site. Further, when the quality of the backlighting for transmission display material is diminished when, for example, a backlight burns out or the output of the backlight decreases with the age, the transmission image will appear dark and reduce the commercial value of the image. It would be desirable if an image support could function both as a reflection and transmission display material.

Prior art transmission display materials use a high coverage of light sensitive silver halide emulsion to increase the density of the image compared to photographic reflection print materials. While increasing the coverage does increase the density of the image in transmission space, the time to image development is also increased as the coverage increases. Typically, a high-density transmission display material has a developer time of at least 110 seconds compared to a developer time of 45 seconds or less for photographic print materials. Prior art high-density transmission display materials, when processed, reduce the productivity of the development lab. Further, coating a high coverage of emulsion requires additional drying of the emulsion in manufacturing, which reduces the productivity of emulsion coating machines. It would be desirable if a transmission display material was high in density and had a developer time less than 50 seconds.

Prior art photographic display material uses polyester as a base for the support. Typically the polyester support is from 150 to 250 micrometers thick to provide the required stiffness. Prior art photographic display materials are typically coated with light sensitive silver halide imaging layers on one side of the support. Exposure devices have been built to expose only one side of prior art display materials thus

there is little concern for print platen design. For example, exposure devices that use a vacuum roll for holding the media during exposing typically employ slots for vacuum. These slots act as "black traps" (areas where exposing energy will be lost and have little secondary reflection) which in a duplitized emulsion system will result in insufficient density for the back side image.

In U.S. Pat. No. 6,030,756 duplitized silver halide imaging layers are discussed for use as a display material. In U.S. Pat. No. 6,030,756, both the top and bottom images are exposed by exposing the topside silver halide imaging layers. While the display material in U.S. Pat. No. 6,030,756 does form an excellent image capable of an exceptional reflection and transmission image, the display material in U.S. Pat. No. 6,030,756 does suffer from sufficient backside image density when placed against a non-uniform reflecting platen.

It has been found that the prior art structure disclosed in U.S. Pat. Nos. 6,030,756 and 6,017,685 is plagued with uneven density variations as a result of uncontrolled back scatter in certain printers in the absence of an antihalation layer. As is obvious, this undesirable exposure can be effectively controlled by the addition of an antihalation layer. However, the presence of an antihalation layer was found to give greatly diminished imaging efficiency, particularly in the backside imaging layer. In this case, the curve shape of an exposure versus density plot reveals a significant break at the mid-scale that leads to significantly lower shoulder and maximum density, as compared to an element without the antihalation layer. Although in principle, it may be possible to recover this density with the addition of silver and coupler to the backside imaging layers, this would be very undesirable on a material cost basis and also due to the desire to keep the required photo processing time to a minimum.

#### PROBLEM TO BE SOLVED BY THE INVENTION

There is a need for a display imaging material that provides an expanded color gamut while maintaining processing efficiency and that will present a bright reflective image when viewed directly and also provide a sharp bright image of sufficient dye density when backlit.

#### SUMMARY OF THE INVENTION

It is an object of the invention to provide improved imaging layers.

It is another object to provide imaging material that has an expanded color gamut.

It is a further object to maintain processing efficiency of the silver halide image.

It is another object to provide a backside image of sufficient dye density when the only exposing light is on the front side of the display element.

These and other objects of the invention are accomplished by an imaging element comprising a translucent polymer sheet, and at least three photosensitive dye forming coupler containing layers on the face side of said sheet, wherein said at least three photosensitive forming coupler containing layers comprise a cyan dye forming layer comprising a cyan dye forming coupler in combination with a red sensitized photosensitive emulsion, a yellow dye forming layer comprising a yellow dye forming coupler in combination with a blue light sensitive photosensitive emulsion, a magenta dye forming layer comprising a magenta dye forming coupler

and a green light sensitive photosensitive emulsion, and on the backside of said translucent polymer sheet at least one dye forming coupler that forms at least one dye that is spectrally distinct from the dyes on the face side of said translucent sheet.

#### ADVANTAGEOUS EFFECT OF THE INVENTION

The invention provides a display imaging material with an improved color gamut while maintaining typical the 45 second color development that will, when imaged and developed, result in a bright sharp reflective image, when viewed in ambient front surface lighting conditions, as well as allowing for a pleasing image of sufficient dye density when illuminated with a transmission light source. In a preferred form the invention provides a product that may be provided with a silver halide image on each side but still retain a single exposure step and short processing time.

#### BRIEF DESCRIPTION OF THE DRAWINGS

FIG. 1 is a cross-sectional drawing of the imaging material with expanded color gamut utilizing a red dye forming coupler.

FIG. 2 is a cross-sectional drawing of the imaging material with expanded color gamut utilizing a blue dye forming coupler.

FIG. 3 is a cross-sectional drawing of the imaging material with expanded color gamut utilizing a red and blue dye forming coupler.

#### DETAILED DESCRIPTION OF THE INVENTION

The invention has numerous advantages over prior practices in the art. The photographic element of the invention employs subtractive, additive, or a combination of subtractive and additive color imaging to form a day/night display material. In such imaging, a viewable digital print color image is formed by generating a combination of cyan, magenta, yellow, red, and blue or black colorants in proportion to the amounts of exposure of up to six different digitally controlled light sources respectively. The object is to provide a reproduction that is pleasing to the observer, but also has the improved capability to specifically reproduce the so-called 'spot colors', Pantone® colors or Hi-Fi colors. Color in the reproduced image is composed of one or a combination of the cyan, magenta, yellow, red, blue, and black image colorants. The silver halide reproduction of Pantone colors allows the invention to better match the performance of printed pigmented inks. The relationship of the original color to the reproduced color is a combination of many factors. It is, however, limited by the color gamut achievable by the multitude of combinations of cyan, magenta, yellow, red, blue and black colorants used to generate the final image.

Illustrated in FIG. 1 is a cross section of the day/night imaging element 11 with expanded color gamut utilizing a red dye forming coupler. Cyan dye forming layer 2, magenta dye forming layer 4, and yellow dye forming layer 6 are applied to translucent support 8. On the backside of translucent support 8, red dye forming layer 10 is applied.

Illustrated in FIG. 2 is a cross section of the day/night imaging element 29 with expanded color gamut utilizing a blue dye forming coupler. Cyan dye forming layer 20, magenta dye forming layer 22, and yellow dye forming layer 24 are applied to translucent support 26. On the backside of translucent support 26, blue dye forming layer 28 is applied.

Illustrated in FIG. 3 is a cross section of the day/night imaging element 41 with expanded color gamut utilizing a red and blue dye forming coupler. Cyan dye forming layer 30, magenta dye forming layer 32, and yellow dye forming layer 34 are applied to translucent support 36. On the backside of translucent support 36, red dye forming layer 38 and blue dye forming layer 40 are applied.

In addition to the individual colorant characteristics, it is necessary to have cyan, magenta and yellow, red and blue colorants that have preferred absorption maxima relative to one another and that have absorption band shapes which function together to provide an optimum overall color gamut. The imaging element of the invention can be processed in 45 seconds, as the additional dyes and couplers required to expand the color gamut are applied to the backside of the transparent polymer sheet, as an additional fourth or fifth layer applied to one side of the support is difficult to process in 45 seconds as the development chemistry does not have enough time to develop the bottommost layers.

FIG. 1 is a cross-sectional drawing of the imaging material with expanded color gamut utilizing a red dye forming coupler. FIG. 2 is a cross-sectional drawing of the imaging material with expanded color gamut utilizing a blue dye forming coupler. FIG. 3 is a cross-sectional drawing of the imaging material with expanded color gamut utilizing a red and blue dye forming coupler.

The developed silver halide imaging element with expanded color gamut is applied to a translucent support material containing an incorporated diffuser thus allowing silver halide images with expanded color gamut to be utilized for illuminated and reflective display. The base materials of the invention allows a greater amount of illuminating light to actually be utilized as display illumination, while at the same time very effectively diffusing the light sources such that they are not apparent to the observer. The display material of the invention will appear whiter to the observer than prior art materials which have a tendency to appear somewhat yellow as they require a high amount of light scattering pigments to prevent the viewing of individual light sources. These high concentrations of pigments appear yellow to the observer and result in an image that is darker than desirable.

The material, as it contains in its preferred form silver halide imaging layers on both sides of a translucent sheet, may be imaged by a collimated beam exposure device in a single exposure. As there are two relatively thin layers of silver halide image materials, the developing of the invention element may be carried out rapidly as the penetration of the developing solution is rapid through the thin layers of imaging material allowing greater productivity in a commercial printing lab. The material of the invention is robust to exposure devices as the chemistry added to the bottom-most layers allows for different exposure devices to be utilized for the formation of quality images. The invention material allows for the simultaneous exposure of both the top and bottom imaging layers while preventing the effects of printer back scatter which would significantly degrade the quality of the image. The structure of the media allows for a pleasing reflection image when the image is captured in a light box containing an air gap from the illumination lamps used for transmission viewing, while also providing uniform diffusion of the transmission illumination source to provide a pleasing transmission image. The invention material ensures that the speed of the front side and back side formed dye density after processing results in a differential speed of the two such that when measured by Status A transmission densitometry there is presented a continuous and uninterrupted curve shape substantially free from non-uniformities caused by an incorrect speed offset of the front side and back side emulsions. These and other advantages will be apparent from the detailed description below.

An imaging element comprising a translucent polymer sheet, and at least three photosensitive dye forming coupler

containing layers on the face side of said sheet, wherein said at least three photosensitive forming coupler containing layers comprise a cyan dye forming layer comprising a cyan dye forming coupler in combination with a red sensitized photosensitive emulsion, a yellow dye forming layer comprising a yellow dye forming coupler in combination with a blue light sensitive photosensitive emulsion, a magenta dye forming layer comprising a magenta dye forming coupler and a green light sensitive photosensitive emulsion, and on the back side of said translucent polymer sheet at least one dye forming coupler that forms at least one dye that is spectrally distinct from the dyes on the face side of said translucent sheet is preferred. By applying at least one of the photosensitive dye forming couplers containing layers on the opposite side of the translucent polymer sheet, during the processing step of image creation, the additional layer of the invention is in contact with the development chemistry, thereby allowing for 45 second development time.

The front image is separated from the back image using a translucent sheet such that utilizing reflected light only, an observer can only see the front image. When the image of the invention is viewed in transmission, the back image is combined with the front image to provide an image that provides expanded color gamut. The translucent polymer sheet of the invention allows a greater amount of illuminating light to actually be utilized as display illumination, while at the same time very effectively diffusing the light sources such that they are not apparent to the observer.

For the silver halide day/night display materials with expanded color gamut, the layers of the biaxially oriented translucent polymer sheet have levels of microvoiding voiding,  $TiO_2$  and colorants adjusted to provide optimum light transmission properties. The functional optical properties for the transmission day/night display materials have been incorporated into the translucent polymer sheet. Microvoiding the polymer sheet in combination with low levels of  $TiO_2$  provides a very effective diffuser of backlighting sources that are used to illuminate transmission display images. Colorants and optical brighteners are added to the translucent polymer sheet of this invention to offset the native yellowness of the photographic imaging layers. The translucent polymer sheet of the invention may be laminated to a transparent polymer base for stiffness for efficient image processing as well as product handling and display. An important aspect of this invention is the elimination of  $TiO_2$  from the base material and the emulsion layers that is typical with prior art transmission materials. Elimination of  $TiO_2$  from the base and emulsion layers allows for a lower cost silver halide transmission display material.

The imaging element wherein said at least four spectrally distinct colors comprise magenta, yellow, cyan, red, and black, wherein said red has a CIELAB hue angle,  $h_{ab}$ , from not less than 355 to not more than 75 degrees is preferred. The possible combinations of cyan, magenta and yellow colorants limit the color saturation and color gamut of red, green, and blue colors that a subtractive color photographic system can reproduce. We have found that the color gamut of a photographic system can be expanded by the use of additional colorants. Red in combination with magenta, yellow, cyan, and black is preferred because red as defined as CIELAB hue angle,  $h_{ab}$ , from not less than 355 to not more than 75 degrees, improves color reproduction possible working in silver halide color space. The red improves a color deficiency in the current silver halide color space, thus allowing an improved color gamut, especially red. The black also provides additional density that is difficult to obtain using balanced amounts of yellow, magenta, and cyan,

providing a deeper, more saturated black. An improved black is more perceptually preferred compared to blacks created using balanced amounts of magenta, cyan, and yellow.

The imaging element wherein at least four spectrally distinct colors comprise magenta, yellow, cyan, blue and black, wherein said blue has a CIELAB hue angle,  $h_{ab}$ , from 225 to 310 degrees is preferred. The possible combinations of cyan, magenta, and yellow colorants limit the color saturation and color gamut of red, green, and blue colors that a subtractive color photographic system can reproduce. We have found that the color gamut of a photographic system can be expanded by the use of additional colorants. Blue, in combination with magenta, yellow, cyan, and black is preferred because blue as defined as CIELAB hue angle,  $h_{ab}$ , from 225 to 310 degrees improves color reproduction possible working in silver halide color space. The blue improves a color deficiency in the current silver halide color space, thus allowing an improved color gamut, especially in the blue. The black also provides additional density that is difficult to obtain using balanced amounts of yellow, magenta, and cyan providing a deeper, more saturated black. An improved black is more perceptually preferred compared to blacks created using balanced amounts of magenta, cyan, and yellow.

The imaging element wherein at least four spectrally distinct colors comprise magenta, yellow, cyan and red, wherein said red has a CIELAB hue angle,  $h_{ab}$ , from not less than 355 to not more than 75 degrees is preferred. The possible combinations of cyan, magenta, and yellow colorants limit the color saturation and color gamut of red, green, and blue colors that a subtractive color photographic system can reproduce. We have found that the color gamut of a photographic system can be expanded by the use of additional colorants. Red, in combination with magenta, yellow, and cyan is preferred because red as defined as CIELAB hue angle,  $h_{ab}$ , from not less than 355 to not more than 75 degrees, improves color reproduction possible working in silver halide color space. The red improves a color deficiency in the current silver halide color space, thus allowing an improved color gamut, especially in the red.

One preferred imaging element has at least four spectrally distinct colors comprise magenta, yellow, cyan, and blue wherein the blue has a CIELAB hue angle,  $h_{ab}$ , from 225 to 310 degrees. The possible combinations of cyan, magenta, and yellow colorants limit the color saturation and color gamut of red, green, and blue colors that a subtractive color photographic system can reproduce. We have found that the color gamut of a photographic system can be expanded by the use of additional colorants. Blue, in combination with magenta, yellow, and cyan is preferred because blue as defined as CIELAB hue angle,  $h_{ab}$ , from 225 to 310 degrees improves color reproduction possible working in silver halide color space. The blue improves a color deficiency in the current silver halide color space, thus allowing an improved color gamut, especially in the blue.

In one preferred imaging element of the invention the spectrally distinct colors comprise magenta, yellow, cyan, red, and blue wherein said blue has a CIELAB hue angle,  $h_{ab}$ , from 225 to 310 degrees and wherein said red has a CIELAB hue angle,  $h_{ab}$ , from not less than 355 to not more than 75 degrees. The possible combinations of cyan, magenta, and yellow colorants limit the color saturation and color gamut of red, green, and blue colors that a subtractive color photographic system can reproduce. We have found that the color gamut of a photographic system can be expanded by the use of additional colorants. Blue and red in

combination with magenta, yellow, and cyan is preferred because blue and red improves color reproduction possible working in silver halide color space. The blue and red improves a color deficiency in the current silver halide color space, thus allowing an improved color gamut of the image.

In another preferred imaging element of the invention the spectrally distinct colors comprise magenta, yellow, cyan, red, black, and blue, wherein said blue has a CIELAB hue angle,  $h_{ab}$ , from 225 to 310 degrees and wherein said red has a CIELAB hue angle,  $h_{ab}$ , from not less than 355 to not more than 75 degrees. The possible combinations of cyan, magenta, and yellow colorants limit the color saturation and color gamut of red, green, and blue colors that a subtractive color photographic system can reproduce. We have found that the color gamut of a photographic system can be expanded by the use of additional colorants. Blue, black, and red in combination with magenta, yellow, and cyan is preferred because blue and red improves color reproduction possible working in silver halide color space. The blue, black, and red improves a color deficiency in the current silver halide color space, thus allowing an improved color gamut of the image. Further, by combining red, blue and black, the image not only has improved color gamut, but also the black provides additional density that is difficult to obtain using equal yellow, magenta and cyan providing a deeper, more saturated black. An improved black is more perceptually preferred compared to blacks created using equal amounts of magenta, cyan, and yellow.

The term as used herein, "transparent" means the ability to pass radiation without significant deviation or absorption. For this invention, "transparent" material is defined as a material that has a spectral transmission greater than 90%. The term as used herein, "translucent" is a property of the optical base materials in which parallel entering light rays exit in a disorderly path. For this invention, "translucent" material is defined as a material having a spectral transmission between 30% and 80%. For a photographic element, spectral transmission is the ratio of the transmitted power to the incident power and is expressed as a percentage as follows:  $T_{RGB}=10^{-D}*100$  where D is the average of the red, green, and blue Status A transmission density response measured by an X-Rite model 310 (or comparable) photographic transmission densitometer.

The terms as used herein, "top", "upper", and "face" relate to the side that is facing the exposure source. The terms "bottom", "lower", and "back" mean the side that is farther from the exposure source.

The imaging element of the invention typically is captured in frames and illumination light boxes. The stiffness of the translucent sheet, on to which the light sensitive silver halide imaging layers are applied, must be stiff for placement into the light boxes and frames. A translucent sheet that has a stiffness of at least 100 millinewtons is preferred, as image stiffness less than 80 millinewtons has been shown to be perceived as low in quality as the consumer associates high quality with a stiff image. Further, image stiffness less than 80 millinewtons is difficult to insert into display frames. Stiffness between 100 millinewtons and 450 millinewtons is most preferred, as stiffness greater than 500 millinewtons is too stiff and encumbers viewing and storage of images by consumers especially in photographic albums and frames.

A translucent sheet that has an  $L^*$  greater than 92.0 is preferred as translucent sheet with  $L^*$  less than 85.0 are not bright enough for a high quality display image. A white translucent sheet is preferred as the white content or density minimum areas in an image are created by the whiteness of

the base because silver halide imaging systems can not as of yet create the color "white".

A preferred translucent sheet comprises a polyester or polyolefin. It has been found that incorporating a voided layer into the translucent sheet provides diffusion of a variety of illuminating back light sources. "Void" is used herein to mean devoid of added solid and liquid matter, although it is likely the "voids" contain gas. The void-initiating particles which remain in the finished packaging sheet core should be from 0.1 to 10 micrometers in diameter, preferably round in shape, to produce voids of the desired shape and size. The size of the void is also dependent on the degree of orientation in the machine and transverse directions. Ideally, the void would assume a shape which is defined by two opposed and edge contacting concave disks. In other words, the voids tend to have a lens-like or biconvex shape. The voids are oriented so that the two major dimensions are aligned with the machine and transverse directions of the sheet. The Z-direction axis is a minor dimension and is roughly the size of the cross diameter of the voiding particle. The voids generally tend to be closed cells, and thus there is virtually no path open from one side of the voided-core to the other side through which gas or liquid can traverse. Voided polymer sheets are preferred as they provide diffusion of the illuminating back light sources without scattering or absorbing back light energy.

A polymer translucent sheet is typically smooth resulting in a high quality glossy image. Further, addenda may be added to the polymer translucent sheet to improve the sharpness and whiteness of the image. Addenda such as white pigments to improve the density minimum areas of the image, optical brightener to prove a blue tint to the density minimum areas and blue tint to offset the native yellowness of the gelatin utilized in the silver halide imaging members. Examples of suitable polymers for a translucent sheet are those disclosed in U.S. Pat. Nos. 4,912,333; 4,994,312; 5,055,371; and 4,187,133. Voided polyester white reflective sheets are preferred as white pigment content in polyester can approach 70% by weight of polymer producing a exceptionally white density minimum area. Voided polyolefin sheets are preferred as they tend to be low in cost and high in mechanical modulus which results in a stiff imaging element.

The polyester film will typically contain an undercoat or primer layer on both sides of the polyester film. Subbing layers used to promote adhesion of coating compositions to the support are well known in the art and any such material can be employed. Some useful compositions for this purpose include interpolymers of vinylidene chloride such as vinylidene chloride/methyl acrylate/itaconic acid terpolymers or vinylidene chloride/acrylonitrile/acrylic acid terpolymers, and the like. These and other suitable compositions are described, for example, in U.S. Pat. Nos. 2,627,088; 2,698,240; 2,943,937; 3,143,421; 3,201,249; 3,271,178; 3,443,950; and 3,501,301. The polymeric subbing layer is usually overcoated with a second subbing layer comprised of gelatin, typically referred to as gel sub. The base also may be a microvoided polyethylene terephthalate such as disclosed in U.S. Pat. Nos. 4,912,333; 4,994,312; 5,055,371; and 6,048,606.

Another preferred translucent sheet comprises a composite structure that includes both a cellulose paper and polymer coatings and/or sheets applied to the surface of the cellulose paper. A composite structure consisting of a cellulose paper base and a polymer for the translucent sheet allows for a low cost, high quality translucent sheet, as this combination allows for the use of low cost of cellulose paper to be used

## 11

in combination with the desirable performance characteristics of a polymer coating or sheet. Examples of suitable cellulose paper, polymer combinations for a translucent sheet are those disclosed in U.S. Pat. Nos. 5,866,282; 5,74,205; 5,888,681; and 5,466,519.

Another preferred translucent sheet comprises a composite structure that includes a polyolefin voided polymer sheet adhesively adhered to a transparent polyester sheet. A composite structure consisting of a transmissive polyolefin sheet and transparent polyester sheet allows for a low cost, high quality translucent sheet, as this combination allows for the use of low cost of polyolefin to be used in combination with the desirable performance characteristics of a polyester sheet. Examples of transmissive polyolefin sheets in combination with polyester sheets are those disclosed in U.S. Pat. Nos. 6,017,685; 6,030,756; and 6,063,552.

Surprisingly, it has also been found that polymer chemistry can be added to the translucent sheet to provide ultraviolet protection to the color couplers used in the developed image layers. Traditionally, this protection for prior art materials has been provided in the gelatin overcoat layer. The incorporation of the ultraviolet protection materials in the biaxially oriented polymer sheet of this invention provides better ultraviolet protection to the imaging couplers and is lower in cost as less ultraviolet filter materials are required in the biaxially oriented sheet than in a gelatin overcoat. Further, the most ultraviolet sensitive color couplers can be applied to the imaging layers that are applied to the back side.

Duplication display materials with expanded color gamut possessing both reflection properties, as well as sufficient dye formed on the backside as a means to present pleasing densities when backlit would be highly desired for display applications. The media would present eye-catching and aesthetically pleasing reflection images, as well as being able to provide pleasing images of sufficient dye densities during nighttime or in low ambient light levels when illuminated from the back side. In addition, the dual property of the formed image (both reflection and transmissive) would allow for pleasing images in outdoor applications or those cases subject to non-controllable high ambient reflection surface lighting (man made or natural) by the property of the formed front side image. In this invention, the face side image formed and backed by the translucent substrate and illuminated by front surface lighting would not appear "washed out" as conventional transmission only display media would.

The inability to predict the future with regard to printer design and expected wear of existing printers can cause serious deficiencies in correct latent image formation. Specifically, a backside light sensitive layer, when exposed against a backing platen of non-uniform reflectivity (due to either wear or design), can adversely affect both the quality of the formed backside latent image, as well as the subsequently processed image resulting in localized non-uniform dye density. The obvious use of an antihalation layer below and adjacent to the bottommost light sensitive layer in the back side structure would clearly resolve the problem of non-uniform reflectivity of any backing apparatus in the printer, but presents its own set of issues. This inclusion of an antihalation layer will solve the problem of backlight scatter by non-uniform reflectivity of media backing in the printer, but will also remove the benefit of any secondary exposure of the backside light sensitive layers.

For this invention, both a "primary first exposure" and an automatic "secondary exposure" of the backside emulsion

## 12

occurs when exposed from only the front side. This is caused by the designed back scatter of the media and compensates for the initial loss of the imaging radiation caused by imaging through the front side of the media and passing through both front side absorber dyes, as well as the translucent support prior to reaching the backside light sensitive layers. In this fashion, a mirror image of the front side image of sufficient sharpness and sufficient dye density is formed on the backside. This allows for both proper image registration (low to no flare of the backside image), as well as sufficient dye density to survive backlighting. In the presence of an antihalation layer on the backside necessitated by uncontrolled back scatter in the printer, the practical result will be a very low density formation of the backside image, and any attempt to increase the front side exposure to improve the back side density will result in overexposure of the face side light sensitive layers, thus degrading the front side image.

This obstacle was solved by the invention whereby a tone enhancing layer was added to the backside adjacent to the bottommost light sensitive layer to provide a tunable "secondary exposure" capability, while also allowing for the application of an antihalation layer to defeat any non-uniform reflectivity resulting from any backing platen or stray back light in the printer. It has been found that these problems can be solved by the addition of a tone enhancing layer between the bottommost light sensitive layer and an antihalation layer. This tone enhancing layer is comprised of a component capable of reflecting light with minimal scatter. Suitable materials include, but are not limited to, titanium dioxide, barium sulfate, clay, calcium carbonate, or suitable polymeric materials. Suitable polymeric materials include hollow polystyrene beads such as Ropaque™ beads (HP-1055, Rohm & Haas). Most preferred is TiO<sub>2</sub>, which may be either of the anatase or rutile type.

The use of this tone enhancing layer also allows for even further improvement of the backside image sharpness, as well as an overall and pleasing increase in transmission maximum density, while not adversely affecting the quality of the face side image.

The developed silver halide image layers preferably contain an environmental protection layer or EPL to protect the delicate silver halide formed image on each side of the translucent sheet from handling damage and damage caused from exposure to liquids. Protection of the silver halide imaging layers is an important attribute of display materials since display materials, because they are often exposed to greater amounts of environmental exposure, need to have the image protected to preserve the quality of the image. Examples of liquids that can damage the silver halide formed image include water, coffee, soda, and the like. Preferred EPLs include UV curable polymers, latex, acrylic, and laminated polymer sheets. Because the EPL layer is critical to conveyance and forming in automated equipment, the EPL layer may require modification. Conveyed products commonly use a variety of lubricants to provide abrasion resistance and slip characteristics. Lubricants used in substrates, printing inks, and coatings include natural waxes, synthetic waxes, fatty acid amides, polytetrafluoroethylene (PTFE), as well as silicone-based compounds.

Natural waxes include vegetable waxes such as carnauba, candelilla, and ouricury. Carnuba, for example, has a molecular weight range of 340–820 with a melting point range of 80–86° C. It has a specific gravity similar to water. Animal and insect waxes include beeswax, shellac, and lanolin. Natural mineral waxes include montan and ozokerite. Natural petroleum waxes include paraffin and micro-

rystalline waxes. Montan is very similar to carnauba wax and has similar molecular weight and melting point characteristics.

Fatty acid amides include euricimide, stearamides, and other primary amides. Fatty acid amides behave like waxes. They have similar molecular weight ranges (275–350) and melting point ranges (68–108° C.).

Synthetic waxes used in packaging include Fisher-Tropsch waxes, PE and PP waxes, and PTFE. PE waxes are used extensively in inks and coatings. They improve abrasion resistance and easily disperse in most common solvents. PTFE waxes used in the ink and coating industries are chemically related to Teflon but have lower molecular weight (10,000–100,000). These waxes have melting points above 300° C. and specific gravity greater than 2. Because they have much higher specific gravity than other waxes, they can be more difficult to handle in low-viscosity systems, such as water-based inks and coatings.

PTFE waxes can be produced in particle sizes ranging from submicrometers to 20  $\mu\text{m}$ . These particles are extremely hard, and the PTFE has lower surface tension than any of the comparable hydrocarbon-based waxes. Use of PTFE is very effective in reducing COF in printing inks and coatings. Since PTFEs do not dissolve or “bloom to the surface,” they are effective in providing lower COF at press. PTFE is chemically inert. It is thermally and oxidatively stable to temperature of 320° C. It is UV-resistant and nonflammable, and it can be used as a release additive.

Silicon-based products are used extensively in inks and coatings to provide slip, abrasion, and mar resistance, as well as release characteristics. Although silicon-based products are used for many of the same purposes as waxes and PTFEs, they are different in performance. Silanes are used when clarity is a priority.

Particle size is a critical parameter for optimum performance of wax. The particle size best suited for given applications should be similar to the thickness of that application of the applied ink film. Lithography applies a very thin ink film in the range of 2–3  $\mu\text{m}$ . Wax particles that are much higher than 5  $\mu\text{m}$  will have difficulty passing through the nip, which may have a gap of only 6  $\mu\text{m}$ . If larger particles are used, “piling” can occur. At the same time, if a coating is applied by rotogravure, the coating process can tolerate much higher particle size wax constituents. In general, for an ink film in the range of 3  $\mu\text{m}$ , a particle size range of 4–6  $\mu\text{m}$  offers the best compromise of rub resistance and performance.

Since the transparent polymer sheet is coated with silver halide imaging layers that are oxygen and moisture sensitive, the transparent sheet of the invention preferably contains oxygen and moisture barrier properties to improve, for example, gelatin hardening which depends the moisture gradient between the machine dryer and the gelatin imaging layers. The preferred water transmission rate of the transparent polymer sheet is between 5 and 500 grams/m<sup>2</sup>/day utilizing test method ASTM F1249. Below 1 gram/m<sup>2</sup>/day, expensive auxiliary coatings are required to reduce water transmission. Above 600 grams/m<sup>2</sup>/day, little improvement in gelatin hardening has been observed. The preferred oxygen transmission rate of the transparent polymer sheet is between 2 and 120 cc/m<sup>2</sup>/day utilizing test method D3985. Below 1 cc/m<sup>2</sup>/day, expensive coatings are required to reduce the oxygen transmission rate. Above 150 cc/m<sup>2</sup>/day, little improvement in dye fade, which is known in the art to be accelerated in the presence of oxygen, has been observed.

The CIELAB metrics, a\*, b\*, and L\*, when specified in combination, describe the color of an object, (under fixed

viewing conditions, etc). The measurement of a\*, b\*, and L\* are well documented and now represent an international standard of color measurement. (The well-known CIE system of color measurement was established by the International Commission on Illumination in 1931 and was further revised in 1971. For a more complete description of color measurement, refer to “Principles of Color Technology, 2nd Edition by F. Billmeyer, Jr. and M. Saltzman, published by J. Wiley and Sons, 1981).

L\* is a measure of how light or dark a color is. L\*=100 is white. L\*=0 is black. The value of L\* is a function of the Tristimulus value Y, thus

$$L^* = 116(Y/Y_n)^{1/3} - 16$$

Simply stated, a\* is a measure of how green or magenta the color is (since they are color opposites), and b\* is a measure of how blue or yellow a color is. From a mathematical perspective, a\* and b\* are determined as follows:

$$a^* = 500 \{ (X/X_n)^{1/3} - (Y/Y_n)^{1/3} \}$$

$$b^* = 200 \{ (Y/Y_n)^{1/3} - (Z/Z_n)^{1/3} \}$$

where X, Y and Z are the Tristimulus values obtained from the combination of the visible reflectance spectrum of the object, the illuminant source (i.e. 5000° K), and the standard observer function.

The a\* and b\* functions determined above may also be used to better define the color of an object. By calculating the arctangent of the ratio of b\*/a\*, the hue-angle of the specific color can be stated in degrees.

$$h_{ab} = \arctan(b^*/a^*)$$

The nomenclature convention for this definition differs from that of the geographic compass heading where 0° or 360° represents north and the angle increases in a clockwise direction. As defined in colorimetric usage, the 0° hue angle is the geographic equivalent of 90° or east, and hue angle increases in a counterclockwise direction. A hue-angle of 0° is broadly defined as magenta. It's complement, 180°, is green. The hue-angle compass between 0° and 360° then includes and describes the hue of all colors. Hue angle does not define lightness or darkness, which is defined by L\*; nor color saturation, C\* which is defined as

$$C^* = (a^{*2} + b^{*2})^{1/2}$$

While it may be convenient to refer to a color as a specific color, for example, ‘red’, in reality, the perception of ‘red’ may encompass a range of hue-angles. This is also true for any other color. In color photographic systems, it is convenient to form cyan, magenta and yellow dyes as the primary subtractive dye set. Subsequently, to reproduce, for example, ‘red’, various combinations of yellow and magenta dyes are formed and the combination of these colorants is perceived by the viewer as ‘red’. Similarly, to form ‘blue’, combinations of magenta and cyan dyes are formed, and to form ‘green’, combinations of cyan and yellow dyes are formed.

For example, a ‘red’ color formed by combining magenta and yellow dyes is limited to the color saturation C\*, of the combination of magenta and yellow. As the relative ratios of the two dyes is varied, the hue angle of the combination changes in proportion. As the amounts of the two dyes change, the color saturation, C\*, and the lightness L\* change. The color saturation, also referred to as color purity is limited by the inherent spectral characteristics of the

15

combinant dyes. The color saturation is a function of the shape of the adsorption band of each dye, the  $\lambda$ -max of each dye, the bandwidth of each dye and other system related factors such as the image viewing conditions, the color and lightness,  $L^*$ , of the reflective support and many related other factors.

The possible combinations of cyan, magenta, and yellow colorants then limit the color saturation and color gamut of red, green, and blue colors that a subtractive color photographic system can reproduce.

We have found that the color gamut of a photographic system can be expanded by the use of additional colorants. Preferred additional colorants are dyes that appear red, blue, or black in color. The red or blue dyes are formed from couplers that have a chemical composition that produces dyes that appear blue or red. Dyes formed by red dye forming couplers have adsorption maxima between that of the magenta and yellow dyes; typically around 500 nm. Dyes formed by blue dye forming couplers have adsorption maxima between that of the magenta and cyan dyes; typically around 600 nm.

Surprisingly, the addition of a green colorant does not significantly increase the color gamut beyond the addition of the red, blue and black colorants.

In some C,M,Y printing systems, such as ink jet or lithographic printing, a 4<sup>th</sup> colorant, K, is added. The 4<sup>th</sup> colorant is black and, therefore, by definition, cannot change the color or hue-angle of a color to which it has been added. The addition of black to a color has two effects: The first to darken the color, thus reducing its  $L^*$  value and the second to desaturate the color (lower  $C^*$ ) which gives the impression that it is less pure.

The addition of K as a colorant has a small positive effect on the available color gamut as it makes dark colors (low  $L^*$ ) more easily achieved.

As used herein, the color gamut of a colorant set is the sum total of the nine slices of color space represented as the sum of  $a^* \times b^*$  areas of 9- $L^*$  slices ( $L^* = 10, 20, 30, 40, 50, 60, 70, 80, \text{ and } 90$ ) for the dye set being tested. Color gamut may be obtained through measurement and estimation from a large sample of color patches (very tedious and time-consuming) or, as herein, calculated from the measured and blue absorption characteristics of the individual colorants using the techniques described in *J. Photographic Science*, 38, 163 (1990).

The absorption characteristics of a given colorant will vary to some extent with a change in colorant amount (transferred and blue density). This is due to factors such as a measurement flare, colorant-colorant interactions, colorant-receiver interactions, colorant concentration effects, and the presence of color impurities in the media. However, by using characteristic vector analysis (sometimes referred to as principal component analysis or eigen-vector analysis), one can determine a characteristic absorption curve that is representative of the absorption characteristics of the colorant over the complete wavelength and density ranges of interest. The characteristic vector for each colorant is, thus, a two-dimensional array of optical transmission density and wavelength. This technique is described by Albert J. Sant in *Photographic Science and Engineering*, 5(3), May-June 1961 and by J. L. Simonds in the *Journal of the Optical Society of America*, 53(8), 968-974 (1963).

The characteristic vector for each colorant is a two-dimensional array of optical transmission density and wavelength normalized to a peak height of 1.0. The characteristic vector is obtained by first measuring the reflection spectra of test images comprising patches of varying densities of the

16

colorant, including fully exposed development yielding a  $D_{max}$  and no exposure ( $D_{min}$ ). The spectral reflection density of the  $D_{min}$  is then subtracted from the spectral reflection density of each color patch. The resulting  $D_{min}$  subtracted reflection densities are then converted to transmission density by passing the density data through the  $Dr/Dt$  curve as defined by Clapper and Williams, *J. Opt. Soc. Am.*, 43, 595 (1953). Characteristic vector analysis is then used to find one transmission density curve for each colorant which, when scaled in transmission density space, converted to reflection density, and added to the  $D_{min}$  of the reflection element, gives a best fit to the measured and blue spectral reflectance data. This characteristic vector is used herein to both specify the spectral absorption characteristics of the colorant and to calculate the color gamut of each imaging system employing the colorant.

Imaging couplers are nominally termed yellow, magenta and cyan if the spectra of their dyes generally absorb in the ranges of 400-500 nm, 500-600 nm, and 600-700 nm, respectively. The image dye-forming couplers in a given color record, typically comprised of one or more light sensitive silver halide emulsion layers, produce image dyes of similar spectral absorption (e.g.  $\lambda_{max} + 20\text{nm}$ ). Image dye-forming couplers are sufficient in type and coverage, considering all of the layers of a given color record, to provide a  $D_{max}$  of at least 1.0. They may thereby be distinguished from functional PUG (photographically useful group) releasing couplers as known in the art, which form a very small portion of the resulting image dye. Thus, after coupling with oxidized developer, the image dye-forming couplers form a predominant portion of the image dye of a particular color record at maximum density. An imaging layer or layer(s) is a layer that is sensitized to light of a particular color range, suitably at least 30 nm apart from such layers sensitized to other color ranges. The absorption curve shape of a colorant is a function of many factors and is not merely a result of the selection of a particular colorant compound. The couplers conventionally employed in silver halide photography form dyes that include yellow ( $h_{ab} = 80-100^\circ$ ); cyan ( $h_{ab} = 200-220^\circ$ ); magenta ( $h_{ab} = 320-350^\circ$ ). Further, the spectral curve may represent the composite absorbance of two or more compounds. For example, if one particular compound provides the desired spectral curve, the addition of further compounds of the same color may provide a composite curve, which remains within the desired range. Thus, when two or more dyes of a particular color are employed, the spectral curve for the "magenta", "yellow", "blue", "red", or "cyan" colorant, for purposes of this invention, means the composite curve obtained from these two or more colorants.

Besides the chemical constitution of the dyes, the spectral curve of a given dye can be affected by other system components (solvents, surfactants, etc.). These parameters are selected to provide the desired spectral curve.

As noted above, the red dye forming coupler forms a dye that has a hue-angle,  $h_{ab}$ , of not less than  $355^\circ$  and not more than  $75^\circ$ , and the blue coupler forms a dye that has a hue-angle from  $225$  to  $310^\circ$ . The dyes are formed upon reaction of the coupler with a suitable developing agent such as a p-phenylenediamine color developing agent. Suitably, the agent is CD-3 as disclosed for use in the RA-4 process of Eastman Kodak Company as described in the British Journal of Photography Annual of 1988, pp 198-199 and described in detail below.

The hue angle of the red dye is from not less than  $355^\circ$  to not more than  $75^\circ$ , suitably from  $5-75^\circ$ , and preferably from  $15-75^\circ$ . and in this coupler combination, desirably from  $25-45^\circ$ .

**17**

Examples of 'red' dyes useful in the invention are:

**18**

-continued



The hue angle of the blue dye is from 225 to 310°, suitably from 228–305°, and preferably from 230–290°. Examples of blue dyes useful in the invention are:

19

-continued



IB-3



IB-4



IB-5



Since the effect of the red and blue dye-forming couplers of the invention is optical rather than chemical, the invention is not limited to a particular compound or class of compounds. Further, more than one coupler of a particular color may be employed in combination which together produce a composite density curve which may satisfy the requirements of the invention.

20

Black Image Couplers

Black image dye forming couplers are well known in the art. Black dyes are those which lack any specific recognizable color and appear as various shades of gray. They are generally formed from m- or p-aminophenols (U.S. Pat. No. 3,622,629); hydroxypyrazoles (U.S. Pat. No. 2,333,106); or resorcinols (U.S. Pat. Nos. 4,126,461 and 5,821,039). The dye is formed upon reaction with a suitable developing agent such as a p-phenylenediamine color-developing agent. Suitably the agent is CD-3, 4-amino-3-methyl-N-ethyl-N-(2-methanesulfonamido-ethyl)aniline sesquisulfate hydrate, as disclosed for use in the RA-4 process of Eastman Kodak Company as described in the British Journal of Photography Annual of 1988, pp. 198-199.

Examples of resorcinol based black dye forming couplers particularly useful in the invention are in issued patents: Suitable black dye forming couplers are disclosed in U.S. Pat. No. 4,126,461 at columns 6-14. The black dye forming couplers in U.S. Pat. No. 5,821,039 at columns 3-5 compounds also are suitable.

It is also possible to have a black dye forming layer that consists of a mixture of cyan, magenta and yellow dyes. Preferred combinations of dye mixtures are given in U.S. Pat. Nos. 5,362,616; 5,364,747; and 5,939,247. The emulsions associated with a black dye forming layer can be singly, ortho- or para-spectrally sensitized.

Cyan Image Couplers

The cyan coupler forms a dye that generally absorbs in the range between 600 nm and 700 nm. The dye is formed upon reaction with a suitable developing agent such as a p-phenylenediamine color-developing agent. Suitably the agent is CD-3, 4-amino-3-methyl-N-ethyl-N-(2-methanesulfonamido-ethyl)aniline sesquisulfate hydrate, as disclosed for use in the RA-4 process of Eastman Kodak Company as described in the British Journal of Photography Annual of 1988, pp. 198-199.



55 wherein

R<sub>1</sub> represents hydrogen or an alkyl group;R<sub>2</sub> represents an alkyl group or an aryl group;

n represents 1, 2, or 3;

each X is a substituent; and

Z represents a hydrogen atom or a group which can be split off by the reaction of the coupler with an oxidized color developing agent.

Coupler (I) is a 2,5-diacylaminophenol cyan coupler in which the S-acylamino moiety is an amide of a carboxylic acid which is substituted in the alpha position by a particular sulfone ( $-\text{SO}_2-$ ) group. The sulfone moiety is an arylsul-

fone. In addition, the 2-acylamino moiety must be an amide ( $-\text{NHCO}-$ ) of a carboxylic acid, and cannot be a ureido ( $-\text{NHCONH}-$ ) group. The result of this unique combination of sulfone-containing amide group at the 5-position and amide group at the 2-position is a class of cyan dye-forming 5 couplers which form H-aggregated image dyes having very sharp-cutting dye hues on the short wavelength side of the absorption curves and absorption maxima ( $\lambda_{\text{max}}$ ) generally in the range of 620–645 nanometers, which is ideally suited for producing excellent color reproduction and high color 10 saturation in color photographic papers.

Referring to formula (I),  $R_1$  represents hydrogen or an alkyl group including linear or branched cyclic or acyclic alkyl group of 1 to 10 carbon atoms, suitably a methyl, ethyl, n-propyl, isopropyl or butyl group, and most suitably an 15 ethyl group.

$R_2$  represents an aryl group or an alkyl group such as a perfluoroalkyl group. Such alkyl groups typically have 1 to 20 carbon atoms, usually 1 to 4 carbon atoms, and include groups such as methyl, propyl, and dodecyl; a perfluoroalkyl group having 1 to 20 carbon atoms, typically 3 to 8 carbon atoms, such as trifluoromethyl or perfluorotetradecyl, heptafluoropropyl or heptadecylfluoroctyl; a substituted or unsubstituted aryl group typically having 6 to 30 carbon atoms, which may be substituted by, for example, 1 to 4 halogen atoms, a cyano group, a carbonyl group, a carbonamido group, a sulfonamido group, a carboxy group, a sulfo group, an alkyl group, an aryl group, an alkoxy group, an aryloxy group, an alkylthio group, an arylthio group, an alkylsulfonyl group or an arylsulfonyl group. Suitably,  $R_2$  represents a heptafluoropropyl group, a 4-chlorophenyl group, a 3,4-dichlorophenyl group, a 4-cyanophenyl group, a 3-chloro-4-cyanophenyl group, a pentafluorophenyl group, a 4-carbonamidophenyl group, a 4-sulfonamidophenyl group, or an alkylsulfonylphenyl group.

Examples of a suitable  $X$  substituent is one located at a position of the phenyl ring meta or para to the sulfonyl group and is independently selected from the group consisting of alkyl, alkenyl, alkoxy, aryloxy, acyloxy, acylamino, sulfonyloxy, sulfamoylamino, sulfonamido, ureido, 40 oxy carbonyl, oxycarbonylamino, and carbamoyl groups.

In formula (I), each  $X$  is preferably located at the meta or para position of the phenyl ring, and each independently represents a linear or branched, saturated or unsaturated alkyl or alkenyl group such as methyl, t-butyl, dodecyl, 45 pentadecyl or octadecyl; an alkoxy group such as methoxy, t-butoxy or tetradecyloxy; an aryloxy group such as phenoxy, 4-t-butylphenoxy or 4-dodecylphenoxy; an alkyl or aryl acyloxy group such as acetoxy or dodecanoxyloxy; an alkyl or aryl acylamino group such as acetamido, 50 benzamido, or hexadecanamido; an alkyl or aryl sulfonyloxy group such as methylsulfonyloxy, dodecylsulfonyloxy, or 4-methylphenylsulfonyloxy; an alkyl or aryl sulfamoylamino group such as N-butylsulfamoylamino, or N-4-t-butylphenylsulfamoylamino; an alkyl or aryl sulfonamido 55 group such as methanesulfonamido, 4-chlorophenylsulfonamido or hexadecanesulfonamido; a ureido group such as methylureido or phenylureido; an alkoxy carbonyl or aryloxy carbonylamino group such as methoxycarbonylamino or phenoxy carbonylamino; a carbamoyl group such as N-butylcarbamoyl or N-methyl-N- 60 dodecylcarbamoyl; or a perfluoroalkyl group such as trifluoromethyl or heptafluoropropyl. Suitably  $X$  represents the above groups having 1 to 30 carbon atoms, more preferably 8 to 20 linear carbon atoms. Most typically,  $X$  represents a 65 linear alkyl or alkoxy group of 12 to 18 carbon atoms such as dodecyl, dodecyloxy, pentadecyl, or octadecyl.

"n" represents 1, 2, or 3; if n is 2 or 3, then the substituents  $X$  may be the same or different.

$Z$  represents a hydrogen atom or a group which can be split off by the reaction of the coupler with an oxidized color developing agent, known in the photographic art as a "coupling-off group". The presence or absence of such groups determines the chemical equivalency of the coupler, i.e., whether it is a 2-equivalent or 4-equivalent coupler, and its particular identity can modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction, and the like.

Representative classes of such coupling-off groups include, for example, halogen, alkoxy, aryloxy, heterocyclyoxy, sulfonyloxy, acyloxy, acyl, heterocycl, sulfonamido, heterocyclthio, benzothiazolyl, phosphonyloxy, alkylthio, arylthio, and arylazo. These coupling-off groups are described in the art, for example, in U.S. Pat. Nos. 2,455,169; 3,227,551; 3,432,521; 3,467,563; 3,617,291; 3,880,661; 4,052,212; and 4,134,766; and in U.K. Patent Nos. and published applications 1,466,728; 1,531,927; 1,533,039; 2,066,755A, and 2,017,704A. Halogen, alkoxy and aryloxy groups are most suitable.

Examples of specific coupling-off groups are  $-\text{Cl}$ ,  $-\text{F}$ ,  $-\text{Br}$ ,  $-\text{SCN}$ ,  $-\text{OCH}_3$ ,  $-\text{OC}_6\text{H}_5$ ,  $-\text{OCH}_2\text{C}(=\text{O})$   $\text{NHCH}_2\text{CH}_2\text{OH}$ ,  $-\text{OCH}_2\text{C}(\text{O})\text{NHCH}_2\text{CH}_2\text{OCH}_3$ ,  $-\text{OCH}_2\text{C}(\text{O})\text{NHCH}_2\text{CH}_2\text{OC}(\text{O})\text{OCH}_3$ ,  $-\text{P}(\text{O})\text{(OC}_2\text{H}_5)_2$ ,  $-\text{SCH}_2\text{CH}_2\text{COOH}$ ,



23



24

-continued

C-2



C-3



C-4



C-5



C-1 50



**25**

-continued



5



25



40



55

**26**

-continued



**27**

-continued



C-14

**28**

-continued



C-18



C-15



C-19



C-16



C-20



C-17



C-21

29

-continued



C-22

5

10

15



623

25

30



40

15

66



C-25



-continued

C-26



C-27



C-28



C-29



**31**

-continued

C-30



5



C-31

20



C-32

25



C-33

30



C-34

35



C-35

40



C-36

45

**32**

-continued

C-34



5



C-31

20



C-32

30



C-33

40



C-34

50



C-35

60



C-36

65

**Magenta Image Couplers**

The magenta image coupler utilized in the invention may be any magenta imaging coupler known in the art. Suitable is a pyrazole of the following structure:



II

wherein R<sub>a</sub> and R<sub>b</sub> independently represent H or a substituent; X is hydrogen or a coupling-off group; and Z<sub>a</sub>, Z<sub>b</sub>, and Z<sub>c</sub> are independently a substituted methine group, =N—, =C—, or —NH—, provided that one of either the Z<sub>a</sub>—Z<sub>b</sub> bond or the Z<sub>b</sub>—Z<sub>c</sub> bond is a double bond and the other is a single bond, and when the Z<sub>b</sub>—Z<sub>c</sub> bond is a carbon-carbon double bond, it may form part of an aromatic ring, and at least one of Z<sub>a</sub>, Z<sub>b</sub>, and Z<sub>c</sub> represents a methine group connected to the group R<sub>b</sub>.

Preferred magenta couplers are 1H-pyrazolo[5,1-c]-1,2,4-triazole and 1H-pyrazolo[1,5-b]-1,2,4-triazole. Examples

**33**

of 1H-pyrazolo [5,1 -c]- 1,2,4-triazole couplers are described in U.K. Patent Nos. 1,247,493; 1,252,418; 1,398, 979; U.S. Pat. Nos. 4,443,536; 4,514,490; 4,540,654; 4,590, 153; 4,665,015; 4,822,730; 4,945,034; 5,017,465; and 5,023,170. Examples of 1H-pyrazolo [1,5-b]-1,2,4-triazoles can be found in European Patent applications 176,804; 177,765; U.S. Patent Nos. 4,659,652; 5,066,575; and 5,250, 400.

In particular, pyrazoloazole magenta couplers of general structures PZ-1 and PZ-2 are suitable:



PZ-1

**34**

-continued

PZ-2

wherein R<sub>a</sub>, R<sub>b</sub>, and X are as defined for formula (II).

Particularly preferred are the two-equivalent versions of magenta couplers PZ-1 and PZ-2 wherein X is not hydrogen. This is the case because of the advantageous drop in silver required to reach the desired density in the print element.

Other examples of suitable magenta couplers are those based on pyrazolones as described hereinafter.

Typical magenta couplers that may be used in the inventive photographic element are shown below.

M-1



M-2



M-3



M-4



-continued



M-5



M-6



M-7



M-8



M-9



The coupler identified as M-2 is useful because of its narrow absorption band.

55

#### Yellow Image Couplers

Couplers that form yellow dyes upon reaction with oxidized color developing agent and which are useful in elements of the invention are described in such representative patents and publications as: U.S. Pat. Nos. 2,875,057; 2,407, 210; 3,265,506; 2,298,443; 3,048,194; 3,447,928 and

“Farbkuppler-Eine Literature Ubersicht,” published in Agfa Mitteilungen, Band III, pp. 112–126 (1961). Such couplers are typically open chain ketomethylene compounds. Also preferred are yellow couplers such as described in, for example, European Patent Application Nos. 482,552; 510, 535; 524,540; 543,367; and U.S. Pat. No. 10 5,238,803.

60

Typical preferred yellow couplers are represented by the following formulas:



wherein  $R_1$ ,  $R_2$ ,  $R_3$ ,  $R_4$ ,  $Q_1$  and  $Q_2$  each represents a substituent;  $X$  is hydrogen or a coupling-off group;  $Y$  represents an aryl group or a heterocyclic group;  $Q_3$  represents an organic residue required to form a nitrogen-containing heterocyclic group together with the  $>N-$ ; and  $Q_4$  represents nonmetallic atoms necessary to from a 3- to 5-membered hydrocarbon ring or a 3- to 5-membered heterocyclic ring which contains at least one hetero atom selected from N, O, S, and P in the ring. Particularly preferred is when  $Q_1$  and  $Q_2$  each represents an alkyl group, an aryl group, or a heterocyclic group, and  $R_2$  represents an aryl or tertiary alkyl group. Preferred yellow couplers for use in elements of the invention are represented by YELLOW-4, wherein  $R_2$  represents a tertiary alkyl group,  $Y$  represents an aryl group, and  $X$  represents an aryloxy or N-heterocyclic coupling-off group.

The most preferred yellow couplers are represented by YELLOW-5, wherein  $R_2$  represents a tertiary alkyl group,  $R_3$  represents a halogen or an alkoxy substituent,  $R_4$  represents a substituent, and  $X$  represents a N-heterocyclic coupling-off group because of their good development and desirable color.

Even more preferred are yellow couplers are represented by YELLOW-5, wherein  $R_2$ ,  $R_3$  and  $R_4$  are as defined above, and  $X$  is represented by the following formula:



wherein  $Z$  is oxygen of nitrogen and  $R_5$  and  $R_6$  are substituents. Most preferred are yellow couplers wherein  $Z$  is oxygen and  $R_5$  and  $R_6$  are alkyl groups.

Representative substituents on such groups include alkyl, aryl, alkoxy, aryloxy, alkylthio, hydroxy, halogen, alkoxy carbonyl, arylox carbonyl, carboxy, acyl, acyloxy, amino, anilino, carbonamido (also known as acylamino), carbamoyl, alkylsulfonyl, arylsulfonyl, sulfonamido, and sulfamoyl groups wherein the substituents typically contain 1 to 40 carbon atoms. Such substituents can also be further substituted. Alternatively, the molecule can be made immobile by attachment to polymeric backbone.

Examples of the yellow couplers suitable for use in the invention are the acylacetanilide couplers, such as those having formula III:



wherein  $Z$  represents hydrogen or a coupling-off group bonded to the coupling site in each of the above formulae. In the above formulae, when  $R^{1a}$ ,  $R^{1b}$ ,  $R^{1d}$ , or  $R^{1f}$  contains a ballast or anti-diffusing group, it is selected so that the total number of carbon atoms is at least 8 and preferably at least 10.

$R^{1a}$  represents an aliphatic (including alicyclic) hydrocarbon group, and  $R^{1b}$  represents an aryl group.

The aliphatic- or alicyclic hydrocarbon group represented by  $R^{1a}$  typically has at most 22 carbon atoms, may be substituted or unsubstituted, and aliphatic hydrocarbon may be straight or branched. Preferred examples of the substituent for these groups represented by  $R^{1a}$  are an alkoxy group, an aryloxy group, an amino group, an acylamino group, and a halogen atom. These substituents may be further substituted with at least one of these substituents repeatedly. Useful examples of the groups as  $R^{1a}$  include an isopropyl group, an isobutyl group, a tert-butyl group, an isoamyl group, a tert-amyl group, a 1,1-dimethyl-butyl group, a 1,1-dimethylhexyl group, a 1,1-diethylhexyl group, a dodecyl group, a hexadecyl group, an octadecyl group, a cyclohexyl group, a 2-methoxyisopropyl group, a 2-phenoxyisopropyl group, a 2-p-tert-butylphenoxyisopropyl group, an a-aminoisopropyl group, an a-(diethylamino)isopropyl group, an a-(succinimido)isopropyl group, an a-(phthalimido)isopropyl group, an a-(benzenesulfonamido)isopropyl group, and the like.

As an aryl group, (especially a phenyl group),  $R^{1b}$  may be substituted. The aryl group (e.g., a phenyl group) may be substituted with substituent groups typically having not more than 32 carbon atoms such as an alkyl group, an alkenyl group, an alkoxy group, an alkoxy carbonyl group, an alkoxy carbonyl amino group, an aliphatic- or alicyclic-amido group, an alkylsulfamoyl group, an alkylsulfonamido group, an alkylureido group, an aralkyl group and an alkyl-substituted succinimido group. This phenyl group in the aralkyl group may be further substituted with groups such as an aryloxy group, an arylox carbonyl group, an aryl carbamoyl group, an arylamido group, an arylsulfamoyl group, an arylsulfonamido group, and an arylureido group.

The phenyl group represented by  $R_{1b}$  may be substituted with an amino group which may be further substituted with a lower alkyl group having from 1 to 6 carbon atoms, a hydroxyl group,  $-COOM$  and  $-SO_2M$  ( $M=H$ , an alkali metal atom,  $NH_4$ ), a nitro group, a cyano group, a thiocyanato group, or a halogen atom.

In a preferred embodiment, the phenyl group represented by  $R_{1b}$  is a phenyl group having in the position ortho to the

**39**

anilide nitrogen a halogen such as fluorine, chlorine or an alkoxy group such as methoxy, ethoxy, propoxy, butoxy. Alkoxy groups of less than 8 carbon atoms are preferred.

$R^{1b}$  may represent substituents resulting from condensation of a phenyl group with other rings, such as a naphthyl group, a quinolyl group, an isoquinolyl group, a chromanyl group, a coumaranyl group, and a tetrahydronaphthyl group.

**40**

These substituents may be further substituted repeatedly with at least one of above-described substituents for the phenyl group.

$R^{1d}$  and  $R^{1f}$  represent a hydrogen atom, or a substituent group (as defined hereafter in the passage directed to substituents).

Representative examples of yellow couplers useful in the present invention are as follows:

Y-1



Y-2



Y-3



Y-4



-continued



Y-5



Y-6



Y-7



Y-8



Y-9

-continued



Y-10



Y-11



Y-12



Y-13

Throughout this specification, unless otherwise specifically stated, substituent groups which may be substituted on molecules herein include any groups, whether substituted or unsubstituted, which do not destroy properties necessary for photographic utility. When the term "group" is applied to the identification of a substituent containing a substitutable hydrogen, it is intended to encompass not only the substituent's unsubstituted form, but also its form further substituted with any group or groups as herein mentioned. Suitably, the group may be halogen or may be bonded to the remainder of the molecule by an atom of carbon, silicon, oxygen, nitrogen, phosphorous, or sulfur. The substituent may be, for example, halogen, such as chlorine, bromine or fluorine; nitro; hydroxyl; cyano; carboxyl; or groups which may be further substituted, such as alkyl, including straight or branched chain alkyl, such as methyl, trifluoromethyl, ethyl, t-butyl, 3-(2,4-di-t-pentylphenoxy) propyl, and tetradecyl; alkenyl, such as ethylene, 2-butene; alkoxy, such as methoxy, ethoxy, propoxy, butoxy, 2-methoxyethoxy, sec-butoxy, hexyloxy, 2-ethylhexyloxy, tetradecyloxy, 2-(2,4-di-t-pentylphenoxy)ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolyloxy; carbonamido, such as acetamido, benzamido, butyramido, tetradecanamido, alpha-(2,4-di-t-pentyl-phenoxy)acetamido, alpha-(2,4-di-t-pentylphenoxy)butyramido, alpha-(3-pentadecylphenoxy)-hexanamido, alpha-(4-hydroxy-3-t-butylphenoxy)-tetradecanamido, 2-oxo-pyrrolidin-1-yl, 2-oxo-5-tetradecylpyrrolidin-1-yl, N-methyltetradecanamido, 30 N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, phenoxy carbonylamino, benzyloxycarbonylamino, hexadecyloxycarbonylamino, 2,4-di-t-butylphenoxy carbonylamino, phenylcarbonylamino, 2,5-(di-1-pentylphenyl)carbonylamino, p-dodecylphenylcarbonylamino, p-tolylcarbonylamino, N-methylureido, N,N-dimethylureido, N-methyl-N-dodecylureido, N-hexadecylureido, N,N-dioctadecylureido, 40 N,N-dioctyl-N'-ethylureido, N-phenylureido, N,N-diphenylureido, N-phenyl-N-p-tolylureido, N-(m-hexadecylphenyl)ureido, N,N-(2,5-di-t-pentylphenyl)-N'-ethylureido, and t-butylcarbonamido; sulfonamido, such as methylsulfonamido, benzenesulfonamido, 45 p-tolylsulfonamido, p-dodecylbenzenesulfonamido, N-methyltetradecylsulfonamido, N,N-dipropylsulfamoylamino, and hexadecylsulfonamido; sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecyloxy)propyl]sulfamoyl, 50 N-[4-(2,4-di-t-pentylphenoxy)butyl]sulfamoyl, N-methyl-N-tetradecylsulfamoyl, and N-dodecylsulfamoyl; carbamoyl, such as N-methylcarbamoyl, N,N-dibutylcarbamoyl, N-octadecylcarbamoyl, N-[4-(2,4-di-t-pentylphenoxy)butyl]carbamoyl, N-methyl-N-tetradecylcarbamoyl, and N,N-dioctylcarbamoyl; acyl, such as acetyl, (2,4-di-t-aminophenoxy)acetyl, phenoxy carbonyl, p-dodecyloxyphenoxy carbonyl methoxycarbonyl, 55 butoxycarbonyl, tetradecyloxycarbonyl, ethoxycarbonyl, benzyloxycarbonyl, 3-pentadecyloxycarbonyl, and dodecylloxycarbonyl; sulfonyl, such as methoxysulfonyl, octyloxysulfonyl, tetradecyloxysulfonyl, 2-ethylhexyloxysulfonyl, phenoxy sulfonyl, 2,4-di-t-pentylphenoxy sulfonyl, methylsulfonyl, octylsulfonyl, 2-ethylhexylsulfonyl, dodecylsulfonyl, hexadecylsulfonyl, phenylsulfonyl, 4-nonylphenylsulfonyl, and

p-tolylsulfonyl; sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl, hexadecylsulfinyl, phenylsulfinyl, 4-nonylphenylsulfinyl, and p-tolylsulfinyl; thio, such as ethylthio, octylthio, benzylthio, tetradecylthio, 2-(2,4-di-t-pentylphenoxy)ethythio, phenylthio, 2-butoxy-5-t-octylphenylthio, and p-tolylthio; acyloxy, such as acetoxy, benzyloxy, octadecanoyloxy, p-dodecylamidobenzoyloxy, N-phenylcarbamoyloxy, N-ethylcarbamoyloxy, and cyclohexylcarbonyloxy; amine, such as phenylanilino, 2-chloroanilino, diethylamine, dodecylamine; imino, such as 1 (N-phenylimido)ethyl, N-succinimido or 3-benzylhydantoinyl; phosphate, such as dimethylphosphate and ethylbutylphosphate; phosphite, such as diethyl and dihexylphosphite; a heterocyclic group, a heterocyclic oxy group or a heterocyclic thio group, each of which may be substituted and which contain a 3- to 7-membered heterocyclic ring composed of carbon atoms and at least one hetero atom selected from the group consisting of oxygen, nitrogen and sulfur, such as 2-furyl, 2-thienyl, 2-benzimidazolyloxy or 2-benzothiazolyl; quaternary ammonium, such as triethylammonium; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups, etc. Generally, the above groups and substituents thereof may include those having up to 48 carbon atoms, typically 1 to 36 carbon atoms and usually less than 24 carbon atoms, but greater numbers are possible depending on the particular substituents selected.

The materials of the invention can be used in any of the ways and in any of the combinations known in the art. Typically, the invention materials are incorporated in a silver halide emulsion and the emulsion coated as a layer on a support to form part of a photographic element. Alternatively, unless provided otherwise, they can be incorporated at a location adjacent to the silver halide emulsion layer where, during development, they will be in reactive association with development products such as oxidized color developing agent. Thus, as used herein, the term "associated" signifies that the compound is in the silver halide emulsion layer or in an adjacent location where, during processing, it is capable of reacting with silver halide development products.

Representative substituents on ballast groups include alkyl, aryl, alkoxy, aryloxy, alkylthio, hydroxy, halogen, alkoxy carbonyl, arylox carbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 42 carbon atoms. Such substituents can also be further substituted.

The color photographic elements of the invention are multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art.

If desired, the photographic element can be used in conjunction with an applied magnetic layer as described in *Research Disclosure*, November 1992, Item 34390 pub-

lished by Kenneth Mason Publications, Ltd., Dudley Annex, 12a North Street, Emsworth, Hampshire PO10 7DQ, ENGLAND, and as described in Hatsumi Kyoukai Koukai Gihou No. 94-6023, published Mar. 15, 1994, available from the Japanese Patent Office. When it is desired to employ the inventive materials in a small format film, *Research Disclosure*, June 1994, Item 36230, provides suitable embodiments.

In the following discussion of suitable materials for use in the emulsions and elements of this invention, reference will be made to *Research Disclosure*, September 1994, Item 36544, available as described above, which will be identified hereafter by the term "Research Disclosure". Sections hereafter referred to are Sections of the *Research Disclosure*.

Except as provided, the silver halide emulsion containing elements employed in this invention can be either negative-working or positive-working as indicated by the type of processing instructions (i.e., color negative, reversal, or direct positive processing) provided with the element. Suitable emulsions and their preparation, as well as methods of chemical and spectral sensitization, are described in Sections I-V. Various additives such as UV dyes, brighteners, antifoggants, stabilizers, light absorbing and scattering materials, and physical property modifying addenda such as hardeners, coating aids, plasticizers, lubricants and matting agents are described, for example, in Sections II and VI-VIII. Color materials are described in Sections X-XIII. Scan facilitating is described in Section XIV. Supports, exposure, development systems, and processing methods and agents are described in Sections XV to XX. Certain desirable photographic elements and processing steps, particularly those useful in conjunction with color reflective prints, are described in *Research Disclosure*, Item 37038, February 1995.

Couplers that form magenta dyes upon reaction with oxidized color developing agent are described in such representative patents and publications as: U.S. Pat. Nos. 2,311,082; 2,343,703; 2,369,489; 2,600,788; 2,908,573; 3,062,653; 3,152,896; 3,519,429; 3,758,309; 4,540,654; and "Farbkuppler-eine Literature Ubersicht," published in Agfa Mitteilungen, Band III, pp. 126-156 (1961). Preferably such couplers are pyrazolones, pyrazolotriazoles, or pyrazolobenimidazoles that form magenta dyes upon reaction with oxidized color developing agents.

Couplers that form yellow dyes upon reaction with oxidized color developing agent are described in such representative patents and publications as: U.S. Pat. Nos. 2,298,443; 2,407,210; 2,875,057; 3,048,194; 3,265,506; 3,447,928; 4,022,620; 4,443,536; and "Farbkuppler-eine Literature Ubersicht," published in Agfa Mitteilungen, Band III, pp. 112-126 (1961). Such couplers are typically open chain ketomethylene compounds.

Couplers that form colorless products upon reaction with oxidized color developing agent are described in such representative patents as U.K. Patent No. 861,138 and U.S. Pat. Nos. 3,632,345; 3,928,041; 3,958,993; and 3,961,959. Typically such couplers are cyclic carbonyl containing compounds that form colorless products on reaction with an oxidized color developing agent.

Couplers that form black dyes upon reaction with oxidized color developing agent are described in such representative patents as U.S. Pat. Nos. 1,939,231; 2,181,944; 2,333,106; and 4,126,461; German OLS No. 2,644,194 and German OILS No. 2,650,764. Typically, such couplers are resorcinols or m-aminophenols that form black or neutral products on reaction with oxidized color developing agent.

In addition to the foregoing, so-called "universal" or "washout" couplers may be employed. These couplers do

not contribute to image dye-formation. Thus, for example, a naphthol having an unsubstituted carbamoyl or one substituted with a low molecular weight substituent at the 2- or 3-position may be employed. Couplers of this type are described, for example, in U.S. Pat. Nos. 5,026,628; 5,151,343; and 5,234,800.

It may be useful to use a combination of couplers any of which may contain known ballasts or coupling-off groups such as those described in U.S. Pat. Nos. 4,301,235; 4,853,319; and 4,351,897. The coupler may contain solubilizing groups such as described in U.S. Pat. No. 4,482,629.

The invention materials may be used in association with materials that accelerate or otherwise modify the processing steps, e.g., of bleaching or fixing to improve the quality of the image. Bleach accelerator releasing couplers such as those described in EP 0 193,389; EP 0 301,477; and U.S. Pat. Nos. 4,163,669; 4,865,956; and 4,923,784 may be useful. Also contemplated is use of the compositions in association with nucleating agents, development accelerators or their precursors (UK Patent Nos. 2,097,140 and 2,131,188); electron transfer agents (U.S. Pat. Nos. 4,859,578 and 4,912,025); antifogging and anticolor-mixing agents such as derivatives of hydroquinones, aminophenols, amines, gallic acid; catechol; ascorbic acid; hydrazides; sulfonamidophenols; and non color-forming couplers.

The invention materials may also be used in combination with filter dye layers comprising colloidal silver sol or yellow, 'blue', cyan, and/or magenta filter dyes, either as oil-in-water dispersions, latex dispersions or as solid particle dispersions. Additionally, they may be used with "smearing" couplers (e.g. as described in U.S. Pat. No. 4,366,237; EP 96,570; U.S. Pat. Nos. 4,420,556; and 4,543,323.) Also, the compositions may be blocked or coated in protected form as described, for example, in Japanese Application 61/258,249 or U.S. Pat. No. 5,019,492.

The invention materials may further be used in combination with image-modifying compounds such as "Developer Inhibitor-Releasing" compounds (DIR's). DIR's useful in conjunction with the compositions of the invention are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346,899; 362,870; 365,252; 365,346; 373,382; 376,212; 377,463; 378,236; 384,670; 396,486; 401,612; and 401,613.

Such compounds are also disclosed in "Developer-Inhibitor-Releasing (DIR) Couplers for Color Photography," C. R. Barr, J. R. Thirtle and P. W. Vittum in Photographic Science and Engineering, Vol. 13, p. 174 (1969). Generally, the developer inhibitor-releasing (DIR) couplers include a coupler moiety and an inhibitor coupling-off moiety (IN). The inhibitor-releasing couplers may be of the time-delayed type (DIAR couplers) which also include a timing moiety or chemical switch which produces a delayed release of inhibitor. Examples of typical inhibitor moieties are: oxazoles, thiazoles, diazoles, triazoles, oxadiazoles, thiadiazoles, oxathiazoles, thiatriazoles, benzotriazoles, tetrazoles,

benzimidazoles, indazoles, isoindazoles, mercaptotetrazoles, selenotetrazoles, mercaptobenzothiazoles, selenobenzothiazoles, mercaptobenzoxazoles, selenobenzoxazoles, mercaptobenzimidazoles, selenobenzimidazoles, benzodiazoles, mercaptooxazoles, mercaptothiadiazoles, mercaptobenzothiazoles, mercaptotriazoles, mercaptooxadiazoles, mercaptodiazoles, mercaptoxathiazoles, tellurotetrazoles or benzisodiazoles. In a preferred embodiment, the inhibitor moiety or group is selected from the following formulas:



wherein  $R_I$  is selected from the group consisting of straight and branched alkyls of from 1 to about 8 carbon atoms, benzyl, phenyl, and alkoxy groups and such groups containing none, one or more than one such substituent;  $R_{II}$  is selected from  $R_I$  and  $-SR_I$ ;  $R_{III}$  is a straight or branched alkyl group of from 1 to about 5 carbon atoms and  $m$  is from 1 to 3; and  $R_{IV}$  is selected from the group consisting of hydrogen, halogens and alkoxy, phenyl and carbonamido groups,  $-COOR_V$  and  $-NHCOOR_V$  wherein  $R_V$  is selected from substituted and unsubstituted alkyl and aryl groups.

It is contemplated that the concepts of the present invention may be employed to obtain reflection color prints as described in *Research Disclosure*, November 1979, Item 18716, available from Kenneth Mason Publications, Ltd, Dudley Annex, 12a North Street, Emsworth, Hampshire PO 101 7DQ, England. Materials of the invention may be coated on pH adjusted support as described in U.S. Pat. No. 4,917,994; on a support with reduced oxygen permeability (EP 553,339); with epoxy solvents (EP 164,961); with nickel complex stabilizers (U.S. Pat. Nos. 4,346,165; 4,540,653 and 4,906,559, for example); with ballasted chelating agents such as those in U.S. Pat. No. 4,994,359 to reduce sensitivity to polyvalent cations such as calcium; and with stain reducing compounds such as described in U.S. Pat. No. 5,068,171. Other compounds useful in combination with the invention are disclosed in Japanese Published Applications described in Derwent Abstracts having accession numbers as follows: 90-072,629; 90-072,630; 90-072,631; 90-072,632; 90-072,633; 90-072,634; 90-077,822; 90-078,229; 90-078,230; 90-079,336; 90-079,337; 90-079,338; 90-079,690; 90-079,691; 90-080,487; 90-080,488; 90-080,489; 90-080,490; 90-080,491; 90-080,492; 90-080,494; 90-085,928; 90-086,669; 90-086,670; 90-087,360; 90-087,361; 90-087,362; 90-087,363; 90-087,364; 90-088,097; 90-093,662; 90-093,663; 90-093,664; 90-093,665; 90-093,666; 90-093,668; 90-094,055; 90-094,056; 90-103,409; 83-62,586; 83-09,959.

The emulsions can be spectrally sensitized with any of the dyes known to the photographic art, such as the polymethine dye class, which includes the cyanines, merocyanines, complex cyanines and merocyanines, oxonols, hemioxonols, 5 styryls, merostyryls and streptocyanines. In particular, it would be advantageous to use the low staining sensitizing dyes disclosed in U.S. Pat. Nos. 5,292,634 and 5,316,904 in conjunction with elements of the invention.

In addition, emulsions can be sensitized with mixtures of 10 two or more sensitizing dyes which form mixed dye aggregates on the surface of the emulsion grain. The use of mixed dye aggregates enables adjustment of the spectral sensitivity of the emulsion to any wavelength between the extremes of the wavelengths of peak sensitivities ( $\lambda$ -max) of the two or 15 more dyes. This practice is especially valuable if the two or more sensitizing dyes absorb in similar portions of the spectrum (i.e., blue, or green or red and not green plus red or blue plus red or green plus blue). Since the function of the spectral sensitizing dye is to modulate the information 20 recorded in the negative which is recorded as an image dye, positioning the peak spectral sensitivity at or near the  $\lambda$ -max of the image dye in the color negative produces the optimum preferred response.

In addition, emulsions of this invention may contain a 25 mixture of spectral sensitizing dyes which are substantially different in their light absorptive properties. For example, Hahm in U.S. Pat. No. 4,902,609 describes a method for broadening the effective exposure latitude of a color negative paper by adding a smaller amount of green spectral 30 sensitizing dye to a silver halide emulsion having predominately a red spectral sensitivity. Thus, when the red sensitized emulsion is exposed to green light, it has little, if any, response. However, when it is exposed to larger amounts of green light, a proportionate amount of cyan image dye will 35 be formed in addition to the magenta image dye, causing it to appear to have additional contrast and hence a broader exposure latitude.

Waki et al in U.S. Pat. No. 5,084,374 describes a silver halide color photographic material in which the red spectrally sensitized layer and the green spectrally sensitized 40 layers are both sensitized to blue light. Like Hahm, the second sensitizer is added in a smaller amount to the primary sensitizer. When these imaging layers are given a large enough exposure of the blue light exposure, they produce 45 yellow image dye to complement the primary exposure. This process of adding a second spectral sensitizing dye of different primary absorption is called false-sensitization.

Any silver halide combination can be used, such as silver 50 chloride, silver chlorobromide, silver chlorobromoiodide, silver bromide, silver bromoiodide, or silver chloroiodide. Due to the need for rapid processing of the color paper, silver chloride emulsions are preferred. In some instances, silver chloride emulsions containing small amounts of bromide, or iodide, or bromide and iodide are preferred, generally less than 2.0 mole percent of bromide less than 1.0 mole percent of iodide. Bromide or iodide addition when forming the emulsion may come from a soluble halide source such as potassium iodide or sodium bromide or an organic bromide or iodide or an inorganic insoluble halide such as silver bromide or silver iodide.

The shape of the silver halide emulsion grain can be 55 cubic, pseudo-cubic, octahedral, tetradecahedral or tabular. It is preferred that the 3-dimensional grains be monodisperse and that the grain size coefficient of variation of the 60 3-dimensional grains is less than 35% or, most preferably less than 25%. The emulsions may be precipitated in any suitable environment such as a ripening environment, or a

reducing environment. Specific references relating to the preparation of emulsions of differing halide ratios and morphologies are Evans U.S. Pat. No. 3,618,622; Atwell U.S. Pat. No. 4,269,927; Wey U.S. Pat. No. 4,414,306; Maskasky U.S. Pat. No. 4,400,463; Maskasky U.S. Pat. No. 4,713,323; Tufano et al U.S. Pat. No. 4,804,621; Takada et al U.S. Pat. No. 4,738,398; Nishikawa et al U.S. Pat. No. 4,952,491; Ishiguro et al U.S. Pat. No. 4,493,508; Hasebe et al U.S. Pat. No. 4,820,624; Maskasky U.S. Pat. No. 5,264,337; and Brust et al EP 534,395.

The combination of similarly spectrally sensitized emulsions can be in one or more layers, but the combination of emulsions having the same spectral sensitivity should be such that the resultant D vs. log-E curve and its corresponding instantaneous contrast curve should be such that the instantaneous contrast of the combination of similarly spectrally sensitized emulsions generally increases as a function of exposure.

Emulsion precipitation is conducted in the presence of silver ions, halide ions and in an aqueous dispersing medium including, at least during grain growth, a peptizer. Grain structure and properties can be selected by control of precipitation temperatures, pH and the relative proportions of silver and halide ions in the dispersing medium. To avoid fog, precipitation is customarily conducted on the halide side of the equivalence point (the point at which silver and halide ion activities are equal). Manipulations of these basic parameters are illustrated by the citations including emulsion precipitation descriptions and are further illustrated by Matsuzaka et al U.S. Pat. No. 4,497,895, Yagi et al U.S. Pat. No. 4,728,603, Sugimoto U.S. Pat. No. 4,755,456, Kishita et al U.S. Pat. No. 4,847,190, Joly et al U.S. Pat. No. 5,017,468, Wu U.S. Pat. No. 5,166,045, Shibayama et al EPO 0 328 042, and Kawai EPO 0 531 799.

Reducing agents present in the dispersing medium during precipitation can be employed to increase the sensitivity of the grains, as illustrated by Takada et al U.S. Pat. No. 5,061,614, Takada U.S. Pat. No. 5,079,138 and EPO 0 434 012, Inoue U.S. Pat. No. 5,185,241, Yamashita et al EPO 0 369 491, Ohashi et al EPO 0 371 338, Katsumi EPO 435 270 and 0 435 355 and Shibayama EPO 0 438 791. Chemically sensitized core grains can serve as hosts for the precipitation of shells, as illustrated by Porter et al U.S. Pat. Nos. 3,206,313 and 3,327,322, Evans U.S. Pat. No. 3,761,276, Atwell et al U.S. Pat. No. 4,035,185 and Evans et al U.S. Pat. No. 4,504,570.

Dopants (any grain occlusions other than silver and halide ions) can be employed to modify grain structure and properties. Periods 3-7 ions, including Group VIII metal ions (Fe, Co, Ni and platinum metals (pm) Ru, Rh, Pd, Re, Os, Ir and Pt), Mg, Al, Ca, Sc, Ti, V, Cr, Mn, Cu, Zn, Ga, As, Se, Sr, Y, Mo, Zr, Nb, Cd, In, Sn, Sb, Ba, La, W, Au, Hg, Ti, Pb, Bi, Ce and U can be introduced during precipitation. The dopants can be employed (a) to increase the sensitivity of either (a1) direct positive or (a2) negative working emulsions, (b) to reduce (b1) high or (b2) low intensity reciprocity failure, (c) to (c1) increase, (c2) decrease or (c3) reduce the variation of contrast, (d) to reduce pressure sensitivity, (e) to decrease dye desensitization, (f) to increase stability, (g) to reduce minimum density, (h) to increase maximum density, (i) to improve room light handling and (j) to enhance latent image formation in response to shorter wavelength (e.g., X-ray or gamma radiation) exposures. For some uses any polyvalent metal ion (pvmi) is effective. The selection of the host grain and the dopant, including its concentration and, for some uses, its location within the host grain and/or its valence can be varied to achieve aim

photographic properties, as illustrated by B. H. Carroll, "Iridium Sensitization: A Literature Review", Photographic Science and Engineering, Vol. 24, No. 6 Nov./Dec. 1980, pp. 265-267 (pm, Ir, a, b and d); Hochstetter U.S. Pat. No. 1,951,933 (Cu); De Witt U.S. Pat. No. 2,628,167 (Tl, a, c); Mueller et al U.S. Pat. No. 2,950,972 (Cd, j); Spence et al U.S. Pat. No. 3,687,676 and Gilman et al U.S. Pat. No. 3,761,267 (Pb, Sb, Bi, As, Au, Os, Ir, a); Ohkubo et al U.S. Pat. No. 3,890,154 (VIII, a); Iwaosa et al U.S. Pat. No. 3,901,711 (Cd, Zn, Co, Ni, Tl, U, T h, Ir, Sr, Pb, b1); Habu et al U.S. Pat. No. 4,173,483 (VIII, b1); Atwell U.S. Pat. No. 4,269,927 (Cd, Pb, Cu, Zn, a2); Weyde U.S. Pat. No. 4,413,055 (Cu, Co, Ce, a2); Akimura et al U.S. Pat. No. 4,452,882 (Rh, i); Menjo et al U.S. Pat. No. 4,477,561 (pm, f); Habu et al U.S. Pat. No. 4,581,327 (Rh, cl, f); Kobuta et al U.S. Pat. No. 4,643,965 (VIII, Cd, Pb, t, c2); Yamashita et al U.S. Pat. No. 4,806,462 (pvmi, a2, g); Grzeskowiak et al U.S. Pat. No. 4,4,828,962 (Ru+Ir, b1); Janusonis U.S. Pat. No. 4,835,093 (Re, al); Leubner et al U.S. Pat. No. 4,902,611 (Ir+4); Inoue et al U.S. Pat. No. 4,981,780 (Mn, Cu, Zn, Cd, Pb, Bi, In, Ti, Zr, La, Cr, Re, VIII, cl, g, h); Kim U.S. Pat. No. 4,997,751 (Ir, b2); Kuno U.S. Pat. No. 5,057,402 (Fe, b, f); Maekawa et al U.S. Pat. No. 5,134,060 (Ir, b, c3); Kawai et al U.S. Pat. No. 5,164,292 (Ir+Se, b); Asami U.S. Pat. Nos. 5,166,044 and 5,204,234 (Fe+Ir, a2 b, cl, c3); Wu U.S. Pat. No. 5,166,045 (Se, a2); Yoshida et al U.S. Pat. No. 5,229,263 (Ir+Fe/Re/Ru/Os, a2, b1); Marchetti et al U.S. Pat. Nos. 5,264,336 and 5,268,264 (Fe, g); Komarita et al EPO 0 244 184 (Ir, Cd, Pb, Cu, Zn, Rh, Pd, Pt, Ti, Fe, d); Miyoshi et al EPO 0 488 737 and 0 488 601 (Ir+VIII/Sc/Ti/V/Cr/Mn/Y/Zr/Nb/Mo/La/Ta/W/Re, a2, b, g); Ihama et al EPO 0 368 304 (Pd, a2, g); Tashiro EPO 0 405 938 (Ir, a2, b); Murakami et al EPO 0 509 674 (VIII, Cr, Zn, Mo, Cd, W, Re, Au, a2, b, g) and Budz WO 93/02390 (Au, g); Ohkubo et al U.S. Pat. No. 3,672,901 (Fe, a2, ol); Yamasue et al U.S. Pat. No. 3,901,713 (Ir+Rh, f); and Miyoshi et al EPO 0 488 737.

When dopant metals are present during precipitation in the form of coordination complexes, particularly tetra- and hexa-coordination complexes, both the metal ion and the coordination ligands can be occluded within the grains. Coordination ligands, such as halo, aquo, cyano, cyanate, fulminate, thiocyanate, selenocyanate, nitrosyl, thionitrosyl, oxo, carbonyl and ethylenediamine tetraacetic acid (EDTA) ligands have been disclosed and, in some instances, observed to modify emulsion properties, as illustrated by Grzeskowiak U.S. Pat. No. 4,847,191, McDugle et al U.S. Pat. Nos. 4,933,272, 4,981,781, and 5,037,732; Marchetti et al U.S. Pat. No. 4,937,180; Keevert et al U.S. Pat. No. 4,945,035, Hayashi U.S. Pat. No. 5,112,732, Murakami et al EPO 0 509 674, Ohya et al EPO 0 513 738, Janusonis WO 91/10166, Beavers WO 92/16876, Pietsch et al German DD 298,320, and Olm et al U.S. Pat. No. 5,360,712.

Oligomeric coordination complexes can also be employed to modify grain properties, as illustrated by Evans et al U.S. Pat. No. 5,024,931.

Dopants can be added in conjunction with addenda, antifoggants, dye, and stabilizers either during precipitation of the grains or post precipitation, possibly with halide ion addition. These methods may result in dopant deposits near or in a slightly subsurface fashion, possibly with modified emulsion effects, as illustrated by Ihama et al U.S. Pat. No. 4,693,965 (Ir, a2); Shiba et al U.S. Pat. No. 3,790,390 (Group VIII, a2, b1); Habu et al U.S. Pat. No. 4,147,542 (Group VIII, a2, b1); Hasebe et al EPO 0 273 430 (Ir, Rh, Pt); Ohshima et al EPO 0 312 999 (Ir, f); and Ogawa U.S. Statutory Invention Registration H760 (Ir, Au, Hg, Tl, Cu, Pb, Pt, Pd, Rh, b, f).

Desensitizing or contrast increasing ions or complexes are typically dopants which function to trap photogenerated holes or electrons by introducing additional energy levels deep within the bandgap of the host material. Examples include, but are not limited to, simple salts and complexes of Groups 8–10 transition metals (e.g., rhodium, iridium, cobalt, ruthenium, and osmium), and transition metal complexes containing nitrosyl or thionitrosyl ligands as described by McDugle et al U.S. Pat. No. 4,933,272. Specific examples include  $K_3RhCl_6$ ,  $(NH_4)_2Rh(Cl_5)H_2O$ ,  $K_2IrCl_6$ ,  $K_3IrCl_6$ ,  $K_2IrBr_6$ ,  $K_2RuCl_6$ ,  $K_2Ru(NO)Br_5$ ,  $K_2Ru(NS)Br_5$ ,  $K_2OsCl_6$ ,  $Cs_2Os(NO)Cl_5$ , and  $K_2Os(NS)Cl_5$ . Amine, oxalate, and organic ligand complexes of these or other metals as disclosed in Olm et al U.S. Pat. No. 5,360,712 are also specifically contemplated.

Shallow electron trapping ions or complexes are dopants which introduce additional net positive charge on a lattice site of the host grain, and which also fail to introduce an additional empty or partially occupied energy level deep within the bandgap of the host grain. For the case of a six coordinate transition metal dopant complex, substitution into the host grain involves omission from the crystal structure of a silver ion and six adjacent halide ions (collectively referred to as the seven vacancy ions). The seven vacancy ions exhibit a net charge of -5. A six coordinate dopant complex with a net charge more positive than -5 will introduce a net positive charge onto the local lattice site and can function as a shallow electron trap. The presence of additional positive charge acts as a scattering center through the Coulomb force, thereby altering the kinetics of latent image formation.

Based on electronic structure, common shallow electron trapping ions or complexes can be classified as metal ions or complexes which have (i) a filled valence shell or (ii) a low spin, half-filled d shell with no low-lying empty or partially filled orbitals based on the ligand or the metal due to a large crystal field energy provided by the ligands. Classic examples of class (i) type dopants are divalent metal complex of Group II, e.g.,  $Mg(2+)$ ,  $Pb(2+)$ ,  $Cd(2+)$ ,  $Zn(2+)$ ,  $Hg(2+)$ , and  $Tl(3+)$ . Some type (ii) dopants include Group VIII complex with strong crystal field ligands such as cyanide and thiocyanate. Examples include, but are not limited to, iron complexes illustrated by Ohkubo U.S. Pat. No. 3,672,901; and rhenium, ruthenium, and osmium complexes disclosed by Keevert U.S. Pat. No. 4,945,035; and iridium and platinum complexes disclosed by Ohshima et al U.S. Pat. No. 5,252,456. Preferred complexes are ammonium and alkali metal salts of low valent cyanide complexes such as  $K_4Fe(CN)_6$ ,  $K_4Ru(CN)_6$ ,  $K_4Os(CN)_6$ ,  $K_2Pt(CN)_4$ , and  $K_3Ir(CN)_6$ . Higher oxidation state complexes of this type, such as  $K_3Fe(CN)_6$  and  $K_3Ru(CN)_6$ , can also possess shallow electron trapping characteristics, particularly when any partially filled electronic states which might reside within the bandgap of the host grain exhibit limited interaction with photocharge carriers.

Emulsion addenda that absorb to grain surfaces, such as antifoggants, stabilizers and dyes can also be added to the emulsions during precipitation. Precipitation in the presence of spectral sensitizing dyes is illustrated by locker U.S. Pat. No. 4,183,756, Locker et al U.S. Pat. No. 4,225,666, Ihama et al U.S. Pat. Nos. 4,683,193 and 4,828,972, Takagi et al U.S. Pat. No. 4,912,017, Ishiguro et al U.S. Pat. No. 4,983,508, Nakayama et al U.S. Pat. No. 4,996,140, Steiger U.S. Pat. No. 5,077,190, Brugger et al U.S. Pat. No. 5,141,845, Metoki et al U.S. Pat. No. 5,153,116, Asami et al EPO 0 287 100 and Tadaaki et al EPO 0 301 508. Non-dye addenda are illustrated by Klotzer et al U.S. Pat. No. 4,705,747, Ogi et

al U.S. Pat. No. 4,868,102, Ohya et al U.S. Pat. No. 5,015,563, Bahnmuller et al U.S. Pat. No. 5,045,444, Maeka et al U.S. Pat. No. 5,070,008, and Vandenabeele et al EPO 0 392 092.

Chemical sensitization of the materials in this invention is accomplished by any of a variety of known chemical sensitizers. The emulsions described herein may or may not have other addenda such as sensitizing dyes, supersensitizers, emulsion ripeners, gelatin or halide conversion restrainers present before, during or after the addition of chemical sensitization.

The use of sulfur, sulfur plus gold or gold only sensitizations are very effective sensitizers. Typical gold sensitizers are chloroaurates, aurous dithiosulfate, aqueous colloidal gold sulfide or gold (aurous bis(1,4,5-trimethyl-1,2,4-triazolium-3-thiolate) tetrafluoroborate. Sulfur sensitizers may include thiosulfate, thiocyanate or N, N'-carbobethoxybis(N-methylcyclycine).

The addition of one or more antifoggants as stain reducing agents is also common in silver halide systems. Tetrazaindenes, such as 4-hydroxy-6-methyl-(1,3,3a,7)-tetrazaindene, are commonly used as stabilizers. Also useful are mercaptotetrazoles such as 1-phenyl-5-mercaptotetrazole or acetamido-1-phenyl-5-mercaptotetrazole. Arylthiosulfonates, such as tolylthiosulfonate or arylsulfonates such as tolylthiosulfonate or esters thereof are also useful.

Useful in this invention are tabular grain silver halide emulsions. Specifically contemplated tabular grain emulsions are those in which greater than 50 percent of the total projected area of the emulsion grains are accounted for by tabular grains having a thickness of less than  $0.3 \mu m$  ( $0.5 \mu m$  for blue sensitive emulsion) and an average tabularity (T) of greater than 25 (preferably greater than 100), where the term "tabularity" is employed in its art recognized usage as

$$T = ECD/t^2$$

where

ECD is the average equivalent circular diameter of the tabular grains in micrometers and

t is the average thickness in micrometers of the tabular grains.

The average useful ECD of photographic emulsions can range up to about  $10 \mu m$ , although in practice emulsion ECD's seldom exceed about  $4 \mu m$ . Since both photographic speed and granularity increase with increasing ECD's, it is generally preferred to employ the smallest tabular grain ECD's compatible with achieving aim speed requirements.

Emulsion tabularity increases markedly with reductions in tabular grain thickness. It is generally preferred that aim tabular grain projected areas be satisfied by thin ( $t < 0.2 \mu m$ ) tabular grains. To achieve the lowest levels of granularity it is preferred that aim tabular grain projected areas be satisfied with ultrathin ( $t < 0.06 \mu m$ ) tabular grains. Tabular grain thicknesses typically range down to about  $0.02 \mu m$ . However, still lower tabular grain thicknesses are contemplated. For example, Daubendick et al U.S. Pat. No. 4,672,027 reports a 3 mole percent iodide tabular grain silver bromoiodide emulsion having a grain thickness of  $0.017 \mu m$ . Ultrathin tabular grain high chloride emulsions are disclosed by Maskasky U.S. Pat. No. 5,217,858.

As noted above tabular grains of less than the specified thickness account for at least 50 percent of the total grain projected area of the emulsion. To maximize the advantages of high tabularity, it is generally preferred that tabular grains satisfying the stated thickness criterion account for the

highest conveniently attainable percentage of the total grain projected area of the emulsion. For example, in preferred emulsions, tabular grains satisfying the stated thickness criteria above account for at least 70 percent of the total grain projected area. In the highest performance tabular grain emulsions, tabular grains satisfying the thickness criteria above account for at least 90 percent of total grain projected area.

The emulsions can be surface-sensitive emulsions, i.e., emulsions that form latent images primarily on the surfaces of the silver halide grains, or the emulsions can form internal latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent.

Photographic elements can be exposed to actinic radiation, typically in the visible region of the spectrum, to form a latent image and can then be processed to form a visible dye image. Processing to form a visible dye image includes the step of contacting the element with a color developing agent to reduce developable silver halide and oxidize the color developing agent. Oxidized color developing agent in turn reacts with the coupler to yield a dye.

To prevent halation during exposure, an antihalation layer needs to be provided between the bottom most light sensitive layer on either side of the transparent support. The antihalation layer acts as a photon trap, absorbing photons of light, which was not part of the latent image formation process after exposure. This layer prevents light from being scattered throughout the photographic element, where it could potentially expose silver halide grains not inline with the exposing beam of incident exposure light. Eliminating the light that is not part of the latent image forming process eliminates halation and increases image sharpness. This is especially important when a scanning exposing device is employed on integral lenticular materials, since the lines of image information are very narrow, typically  $5\mu$  to  $10\mu$  in diameter. If the consecutive adjacent lines of image information differ significantly in intensity and which subsequently result in significantly different amount of image density, if the element is un-sharp, the lines will broaden unnecessarily and merge in such a way that the distinct separate images will appear undistinguished from each other. Thus an image scene which is predominantly "dark" which is arranged adjacent to an image scene which is predominately "light" will visually blur together in the eyes of the observer and reduce the apparent quality of the image.

Antihalation layers are common in most color negative films such as Kodak Advantix™ film and also are found in some color print films such as Kodak Vision Color Print Film™ or Kodak Duraclear RA Display Material™. Antihalation materials are incorporated to absorb light not absorbed as part of the imaging process. This material is typically 'gray' in color and absorbs light of all color. A variety of materials have been suggested to fill this requirement. Finely dispersed carbon black is used in some products and is known in the trade as 'rem-jet'. It must be removed prior to the chemical development step via a pre-bath and as such must be coated on the side of the support opposite the imaging layers as it cannot be solubilized during the processing cycles. Finely divided elemental silver is also widely used in many color negative films. This material is known as 'gray gel' and is easily removed in the

chemical development process during the bleaching and fixing steps. In some products, mixtures of water soluble cyan, magenta, and yellow dyes are coated in a separate layer (usually on the side of the support opposite the emulsion layers). If these water soluble dyes are coated on the same side of the support as the emulsions, they diffuse into the emulsion layers after the coating operation and retard the photographic speed of the photographic element. Since these dye are aqueous soluble, they are conveniently removed during processing via diffusion or reaction with alkali or sulfite in the color developer.

To overcome this tendency, solid particle dispersions of these dyes have been developed. The dyes in these formulations are insoluble under all but alkaline conditions so that they remain in the layer in which they are coated, but can be removed by hydrolysis or ionization during the chemical development step of the photographic process.

With negative-working silver halide, the processing step described above provides a negative image. The described elements can be processed in the known Kodak RA-4 color process as described the British Journal of Photography Annual of 1988, pp. 198-199. To provide a positive (or reversal) image, the color development step can be preceded by development with a non-chromogenic developing agent to develop exposed silver halide, but not form dye, and followed by uniformly fogging the element to render unexposed silver halide developable. Such reversal emulsions are typically sold with instructions to process using a color reversal process such as E-6. Alternatively, a direct positive emulsion can be employed to obtain a positive image.

Preferred color developing agents are p-phenylenediamines such as:

4-amino-N,N-diethylaniline hydrochloride,  
4-amino-3-methyl-N,N-diethylaniline hydrochloride,  
4-amino-3-methyl-N-ethyl-N-(2-methanesulfonamidoethyl)aniline sesquisulfate hydrate,  
4-amino-3-methyl-N-ethyl-N-(2-hydroxyethyl)aniline sulfate,  
4-amino-3-(2-methanesulfonamido-ethyl)-N,N-diethylaniline hydrochloride and  
4-amino-N-ethyl-N-(2-methoxyethyl)-m-toluidine di-p-toluene sulfonic acid.

Development is usually followed by the conventional steps of bleaching, fixing, or bleach-fixing, to remove silver or silver halide, washing, and drying.

A direct-view photographic element is defined as one which yields a color image that is designed to be viewed directly (1) by reflected light, such as a photographic paper print, (2) by transmitted light, such as a display transparency, or (3) by projection, such as a color slide or a motion picture print. These direct-view elements may be exposed and processed in a variety of ways. For example, paper prints, display transparencies, and motion picture prints are typically produced by optically printing an image from a color negative onto the direct-viewing element and processing through an appropriate negative-working photographic process to give a positive color image. Color slides may be produced in a similar manner but are more typically produced by exposing the film directly in a camera and processing through a reversal color process or a direct positive process to give a positive color image. The image may also be produced by alternative processes such as digital printing.

Each of these types of photographic elements has its own particular requirements for dye hue, but in general, they all require cyan dyes that whose absorption bands are less deeply absorbing (that is, shifted away from the red end of

the spectrum) than color negative films. This is because dyes in direct viewing elements are selected to have the best appearance when viewed by human eyes, whereas the dyes in color negative materials designed for optical printing are designed to best match the spectral sensitivities of the print materials.

The following examples illustrate the practice of this invention. They are not intended to be exhaustive of all possible variations of the invention. Parts and percentages are by weight unless otherwise indicated. The following examples are representative of materials that could be adhered to translucent polymer base to form display members of the invention.

## EXAMPLES

## Photographic Examples 1 to 7

Dispersions of example couplers were emulsified by methods well known to the art, and were coated on the face side of a doubly extruded polyethylene coated color paper support or transparent polymeric support as appropriate for the example, using conventional coating techniques. The gelatin layers were hardened with bis (vinylsulfonyl methyl) ether at 2.4% of the total gelatin. The preparation and composition of the individual layers and their components is given as follows:

## Dispersion Formulations

## Dispersions Such as CD Were Formulated as Follows

The oil phase of the dispersion formula is composed of a mixture of:

|                                |         |
|--------------------------------|---------|
| Coupler C-1                    | 100.0 g |
| Di-n-butylphthalate            | 100.0 g |
| Tinuvin 328™                   | 64.3 g  |
| 2-(2-butoxyethoxy)ethylacetate | 8.2 g   |

The aqueous phase of the dispersion is composed of a mixture of:

|                        |          |
|------------------------|----------|
| Gelatin                | 120.0 g  |
| Alkanol XC™ surfactant | 12.0 g   |
| Water                  | 1574.0 g |

## Dispersions Such as MD Were Formulated as Follows

The oil phase of the dispersion formula is composed of a mixture of:

|                                |         |
|--------------------------------|---------|
| Coupler M-2                    | 100.0 g |
| Oleyl alcohol                  | 105.0 g |
| Di-n-undecyl phthalate         | 54.0 g  |
| 2-(2-butoxyethoxy)ethylacetate | 10.0 g  |
| ST-21                          | 19.3 g  |
| ST-22                          | 131.8 g |

## Dispersions Such as YD Were Formulated as Follows

The oil phase of the dispersion formula is composed of a mixture of:

|                                |         |
|--------------------------------|---------|
| Coupler Y-5                    | 100.0 g |
| Tri-butyl-citrate              | 52.6 g  |
| 2-(2-butoxyethoxy)ethylacetate | 4.0 g   |
| ST-23                          | 29.2 g  |

## Dispersions Such as KD-1 Were Formulated as Follows

The oil phase of the dispersion formula is composed of a mixture of:

|                                |        |
|--------------------------------|--------|
| Coupler C-1                    | 50.0 g |
| Coupler M-1                    | 37.1 g |
| Coupler Y-13                   | 65.6 g |
| Di-n-butyl phthalate           | 62.6 g |
| 2-(2-butoxyethoxy)ethylacetate | 78.5 g |

## Dispersions Such as KD-2 Were Formulated as Follows

The oil phase of the dispersion formula is composed of a mixture of:

|                        |         |
|------------------------|---------|
| Coupler K-73           | 100.0 g |
| N,N-di-butyl lauramide | 200.0 g |

## Dispersinsch Procedure

- 1) The materials used in the oil phase are combined and heated to 125° C. with stirring, until dissolution occurs.
- 2) The hot oil phase is quickly added to the a queous phase which has been pre-heated to 70° C.
- 3) The mixture is then passed through a colloid mix, collected, then chilled until the dispersion is set.

## Emulsion Formulations

Silver chloride emulsions were chemically and spectrally sensitized as is described below.

Blue Sensitive Emulsion (BEM-1, prepared as described in U.S. Pat. No. 5,252,451, column 8, lines 55–68): A high chloride silver halide emulsion was precipitated by adding approximately equimolar silver nitrate and sodium chloride solutions into a well-stirred reactor containing gelatin peptizer and thioether ripener.  $\text{Cs}_2\text{Os}(\text{NO})\text{Cl}_5$  (136  $\mu\text{g}/\text{Ag-M}$ ) and  $\text{K}_2\text{IrCl}_5$  (5-methylthiazole) (72  $\mu\text{g}/\text{Ag-M}$ ), dopants were added during the silver halide grain formation for most of the precipitation. At 90% of the grain volume, precipitation was halted and a quantity of potassium iodide was added, equivalent to 0.2 M % of the total amount of silver. After addition, the precipitation was completed with the addition of additional silver nitrate and sodium chloride and subsequently followed by a shelling without dopant. The resultant emulsion contained cubic shaped grains of 0.60  $\mu\text{m}$  in edge length. This emulsion was optimally sensitized by the addition of a colloidal suspension of aurous sulfide (18.4 mg/Ag-M) and heat ramped up to 60° C. during which time blue sensitizing dye BSD-4, (388 mg/Ag-M), 1-(3-acetamidophenyl)-5-mercaptotetrazole (93 mg/Ag-M) and potassium bromide (0.5 M %) were added. In addition,

59

iridium dopant  $K_2IrCl_6$  (7.4  $\mu\text{g}/\text{Ag-M}$ ) was added during the sensitization process.

Blue Sensitive Emulsion (BEM-2, prepared as described in U.S. Pat. No. 5,252,451, column 8, lines 55-68): A high chloride silver halide emulsion was precipitated by adding approximately equimolar silver nitrate and sodium chloride solutions into a well-stirred reactor containing gelatin peptizer and thioether ripener.  $Cs_2Os(NO)Cl_5$  (136  $\mu\text{g}/\text{Ag-M}$ ) and  $K_2IrCl_5(5\text{-methylthiazole})$  (72  $\mu\text{g}/\text{Ag-M}$ ), dopants were added during the silver halide grain formation for most of the precipitation. At 90% of the grain volume, precipitation was halted and a quantity of potassium iodide was added, equivalent to 0.2 M % of the total amount of silver. After addition, the precipitation was completed with the addition of additional silver nitrate and sodium chloride and subsequently followed by a shelling without dopant. The resultant emulsion contained cubic shaped grains of 0.60  $\mu\text{m}$  in edge length. This emulsion was optimally sensitized by the addition of a colloidal suspension of aurous sulfide (18.4 mg/Ag-M) and heat ramped up to 60° C. during which time blue sensitizing dye BSD-2, (414 mg/Ag-M), 1-(3-acetamidophenyl)-5-mercaptopentetrazole (93 mg/Ag-M) and potassium bromide (0.5 M %) were added. In addition, iridium dopant  $K_2IrCl_6$  (7.4  $\mu\text{g}/\text{Ag-M}$ ) was added during the sensitization process.

Green Sensitive Emulsion (GEM-1): A high chloride silver halide emulsion was precipitated by adding approximately equimolar silver nitrate and sodium chloride solutions into a well-stirred reactor containing gelatin peptizer and thioether ripener.  $Cs_2Os(NO)Cl_5$  (1.36  $\mu\text{g}/\text{Ag-M}$ ) dopant and  $K_2IrCl_5(5\text{-methylthiazole})$  (0.54 mg/Ag-M) dopant was added during the silver halide grain formation for most of the precipitation, followed by a shelling without dopant. The resultant emulsion contained cubic shaped grains of 0.30  $\mu\text{m}$  in edge length. This emulsion was optimally sensitized by addition of a colloidal suspension of aurous sulfide (12.3 mg/Ag-M), heat digestion, followed by the addition of silver bromide (0.8 M %), green sensitizing dye, GSD-1 (427 mg/Ag-M), and 1-(3-acetamidophenyl)-5-mercaptopentetrazole (96 mg/Ag-M).

Red Sensitive Emulsion (REM-1): A high chloride silver halide emulsion was precipitated by adding approximately equimolar silver nitrate and sodium chloride solutions into a well-stirred reactor containing gelatin peptizer and thioether ripener. The resultant emulsion contained cubic shaped grains of 0.40  $\mu\text{m}$  in edge length. In addition, ruthenium hexacyanide dopant (at 16.5 mg/Ag-M) and  $K_2IrCl_5(5\text{-methylthiazole})$  dopant (at 0.99 mg/Ag-M) was added during the precipitation process. This emulsion was optimally sensitized by the addition of a colloidal suspension of aurous sulfide (60 mg/Ag-M) followed by a heat ramp to 65° C. for 45 minutes, and further additions of 1-(3-acetamidophenyl)-5-mercaptopentetrazole (295 mg/Ag-M), iridium dopant,  $K_2IrCl_6$  (149  $\mu\text{g}/\text{Ag-M}$ ), potassium bromide, (0.5 Ag-M %), and red sensitizing dye RSD-I (7.1 mg/Ag-M).

Red Sensitive Emulsion (Red EM-2): A high chloride silver halide emulsion was precipitated by adding approximately equimolar silver nitrate and sodium chloride solutions into a well-stirred reactor containing gelatin peptizer and thioether ripener. The resultant emulsion contained cubic shaped grains of 0.40  $\mu\text{m}$  in edge length. In addition,

60

ruthenium hexacyanide dopant (at 16.5 mg/Ag-M) and  $K_2IrCl_5(5\text{-methylthiazole})$  dopant (0.99 mg/Ag-M) was added during the precipitation process. This emulsion was optimally sensitized by the addition of a colloidal suspension of aurous sulfide (60 mg/Ag-M) followed by a heat ramp to 65° C. for 45 minutes, and further additions of 1-(3-acetamidophenyl)-5-mercaptopentetrazole (295 mg/Ag-M), iridium dopant  $K_2IrCl_6$  (149  $\mu\text{g}/\text{Ag-M}$ ), potassium bromide (0.5 Ag-M %), and sensitizing dye GSD-2 (8.9 mg/Ag-M).

Infrared Sensitive Emulsion (FSEM-1): A high chloride silver halide emulsion was precipitated by adding approximately equimolar silver nitrate and sodium chloride solutions into a well-stirred reactor containing gelatin peptizer and thioether ripener. The resultant emulsion contained cubic shaped grains of 0.40  $\mu\text{m}$  in edge length. In addition, ruthenium hexacyanide dopant (at 16.5 mg/Ag-M) and  $K_2IrCl_5(5\text{-methylthiazole})$  dopant (at 0.99 mg/Ag-M) was added during the precipitation process. This emulsion was optimally sensitized by the addition of a colloidal suspension of aurous sulfide (60. mg/Ag-M) followed by a heat ramp to 65° C. for 45 minutes, followed by further additions of antifoggant, 1-(3-acetamidophenyl)-5-mercaptopentetrazole (295. mg/Ag-M), iridium dopant ( $K_2IrCl_6$  at 149.  $\mu\text{g}/\text{Ag-M}$ ), potassium bromide (0.5 Ag-M %), DYE-5 (300 mg/Ag-M), infrared sensitizing dye IRSD-1 (33.0 mg/Ag-M) and finally, after the emulsion was cooled to 40° C., DYE-4 (10.76 mg/M<sup>2</sup>).

Infrared Sensitive Emulsion (FSEM-2): A high chloride silver halide emulsion was precipitated by adding approximately equimolar silver nitrate and sodium chloride solutions into a well-stirred reactor containing gelatin peptizer and thioether ripener. The resultant emulsion contained cubic shaped grains of 0.40  $\mu\text{m}$  in edge length. In addition, ruthenium hexacyanide dopant (at 16.5 mg/Ag-M) and  $K_2IrCl_5(5\text{-methylthiazole})$  dopant (at 0.99 mg/Ag-M) was added during the precipitation process. This emulsion was optimally sensitized by the addition of a colloidal suspension of aurous sulfide (60. mg/Ag-M) followed by a heat ramp to 65° C. for 45 minutes, followed by further additions of antifoggant, 1-(3-acetamidophenyl)-5-mercaptopentetrazole (295. mg/Ag-M), iridium dopant  $K_2IrCl_6$  (149.  $\mu\text{g}/\text{Ag-M}$ ), potassium bromide (0.5 Ag-M %), DYE-5 (300 mg/Ag-M), infrared sensitizing dye IRSD-2 (33.0 mg/Ag-M) and finally, after the emulsion was cooled to 40° C., DYE-4 (10.76 mg/M<sup>2</sup>).

Infrared Sensitive Emulsion (FSEM-3): A high chloride silver halide emulsion was precipitated by adding, approximately equimolar silver nitrate and sodium chloride solutions into a well-stirred reactor containing gelatin peptizer and thioether ripener. The resultant emulsion contained cubic shaped grains of 0.40  $\mu\text{m}$  in edge length. In addition, ruthenium hexacyanide dopant (16.5 mg/Ag-M) and  $K_2IrCl_5(5\text{-methylthiazole})$  dopant (0.99 mg/Ag-M) was added during the precipitation process. This emulsion was optimally sensitized by the addition of a colloidal suspension of aurous sulfide (60. mg/Ag-M) followed by a heat ramp to 65° C. for 45 minutes, followed by further additions of antifoggant, 1-(3-acetamidophenyl)-5-mercaptopentetrazole (295. mg/Ag-M), iridium dopant  $K_2IrCl_6$  (149.  $\mu\text{g}/\text{Ag-M}$ ), potassium bromide (0.5 Ag-M %), DYE-5 (300 mg/Ag-M), infrared

sensitizing dye IRSD-3 (33.0 mg/Ag-M) and finally, after the emulsion was cooled to 40° C., DYE-4 (10.76 mg/M<sup>2</sup>).

Infrared Sensitive Emulsion (FSEM-4): A high chloride silver halide emulsion was precipitated by adding approximately equimolar silver nitrate and sodium chloride solutions into a well-stirred reactor containing gelatin peptizer and thioether ripener. The resultant emulsion contained cubic shaped grains of 0.40  $\mu$ m in edge length. In addition, ruthenium hexacyanide dopant (at 16.5 mg/Ag-M) and K<sub>2</sub>IrCl<sub>5</sub>(5-methylthiazole) dopant (0.99 mg/Ag-M) was added during the precipitation process. This emulsion was optimally sensitized by the addition of a colloidal suspension of aurous sulfide (60. mg/Ag-M) followed by a heat ramp to 65° C. for 45 minutes, followed by further additions of antifoggant, 1-(3-acetamidophenyl)-5-mercaptopotetrazole (295. mg/Ag-M), iridium dopant K<sub>2</sub>IrCl<sub>6</sub> (149.  $\mu$ g/Ag-M), potassium bromide (0.5 Ag-M %), DYE-5 (300 mg/Ag-M), infrared sensitizing dye IRSD-4 (33.0 mg/Ag-M) and finally, after the emulsion was cooled to 40° C., DYE-4 (10.76 mg/M<sup>2</sup>).

After the coatings were prepared, they were exposed via a digital printer whose output devices were co-optimized to align with the spectral sensitivities of the elements described below. After exposing, the elements were processed in the standard Kodak Ektacolor™ RA4 Color Paper development process which is described below:

TABLE 1

| Kodak Ektacolor™ RA-4 Color Developer |                 |
|---------------------------------------|-----------------|
| Chemical                              | Grams/Liter     |
| Triethanol amine                      | 12.41           |
| Phorwite REU™                         | 2.30            |
| Lithium polystyrene sulfonate (30%)   | 0.30            |
| N,N-diethylhydroxylamine (85%)        | 5.40            |
| Lithium sulfate                       | 2.70            |
| Kodak color developer CD-3            | 5.00            |
| DEQUEST 2010™ (60%)                   | 1.16            |
| Potassium carbonate                   | 21.16           |
| Potassium bicarbonate                 | 2.79            |
| Potassium chloride                    | 1.60            |
| Potassium bromide                     | 0.007           |
| Water                                 | to make 1 liter |

pH @ 26.7° C. is 10.04 +/- 0.05

TABLE 2

| Kodak Ektacolor™ RA-4 Bleach-Fix |                 |
|----------------------------------|-----------------|
| Chemical                         | Grams/Liter     |
| Ammonium thiosulfate (56.5%)     | 127.40          |
| Sodium metabisulfite             | 10.00           |
| Glacial acetic acid              | 10.20           |
| Ammonium ferric EDTA (44%)       | 110.40          |
| Water                            | to make 1 liter |

pH @ 26.7° C. is 5.5 +/- 0.10

TABLE 3

| Kodak Ektacolor™ RA-4 Color Paper Process |                |
|-------------------------------------------|----------------|
| Process Step                              | Time (seconds) |
| Color Development                         | 45 or 81       |
| Bleach-fix                                | 45 or 81       |

TABLE 3-continued

| Kodak Ektacolor™ RA-4 Color Paper Process |                |     |
|-------------------------------------------|----------------|-----|
| Process Step                              | Time (seconds) |     |
| Wash                                      | 90 or 162      | Dry |

Processing the exposed paper samples is performed with the developer and bleach-fix temperatures adjusted to 35° C. Washing is performed with tap water at 32.2° C.

The following table gives the spectral sensitivities obtained with the combinations of spectral sensitizing dyes and emulsions provided above.

TABLE 4

| Spectral Sensitivities of the Photographic Element |             |                 |                           |
|----------------------------------------------------|-------------|-----------------|---------------------------|
| Color Record                                       | Emulsion    | Sensitizing Dye | Peak Spectral Sensitivity |
| Blue                                               | BEM-2       | BSD-4           | 473 nm                    |
| Green                                              | GEM-1       | GSD-1           | 550 nm                    |
| Red                                                | REM-1       | RSD-1           | 695 nm                    |
| 4 <sup>th</sup> Sensitive                          | BEM-1       | BSD-2           | 425 nm                    |
| 5 <sup>th</sup> Sensitive                          | REM-2       | GSD-2           | 625 nm                    |
| 6 <sup>th</sup> Sensitive                          | FSEM-1 to 4 | IRSD-1 to 4     | 750 to 800 nm             |

#### Reference and 4-Colorant Duplitzed Photographic Elements 1 to 7

The following table describes the combinations of layers, emulsions and coupler dispersions that make up the control or reference 3-color element and the inventive 4-color duplitzed elements. The first column of the table provides a reference code for an element combination. The second and third columns describe the layer orders of each of the different spectrally sensitized color records. The second column, titled 'Face Side', gives the colorant layer order starting with the layer furthest from the support. The third column, titled 'Reverse Side', describes the colorant used on the reverse side of the support, opposite the other color records. The fourth to the seventh columns describe the combination of emulsion and dispersion used in each layer and which were described in detail above.

The first two rows of the table provide the general compositions of two reference multilayer elements that are not duplitzed. Reference element-1 shows the conventional and historic layer orders for conventional color papers. Reference element-2 provides an alternate combination of emulsions and dispersions. This combination of emulsions and dispersions results in an element that is false sensitized, in that the colorant produced by the layer is not complementary to the wavelength of light used to expose the layer. A design such as this requires that the element be printed using a digital exposing device due to the nature of color negative films.

TABLE 5

| General Composition of the Reference and 4 Colorant Elements |                   |         |                                                    |          |          |             |  |
|--------------------------------------------------------------|-------------------|---------|----------------------------------------------------|----------|----------|-------------|--|
| Reference                                                    | Sensitized Layers |         | Identification of Emulsion and Coupler Dispersions |          |          |             |  |
|                                                              | Face and 4-Color  | Reverse | CE/CD                                              | ME/MD    | YE/YD    | KE/KD       |  |
| Examples                                                     | Side              | Side    | CE/CD                                              | ME/MD    | YE/YD    | KE/KD       |  |
| Reference-1                                                  | CMY               | none    | REM-1/CD                                           | GEM-1/MD | BEM-1/YD | N/A         |  |
| Reference-2                                                  | CMY               | none    | GEM-1/CD                                           | BEM-1/MD | REM-1/YD | N/A         |  |
| 1-31-1                                                       | CMY               | K       | REM-1/CD                                           | GEM-1/MD | BEM-1/YD | FSEM-1/KD-1 |  |
| 2-31-2                                                       | CYK               | M       | REM-1/CD                                           | GEM-1/MD | BEM-1/YD | FSEM-2/KD-1 |  |
| 3-31-3                                                       | MYK               | C       | REM-1/CD                                           | GEM-1/MD | BEM-1/YD | FSEM-3/KD-1 |  |
| 4-31-4                                                       | CMK               | Y       | REM-1/CD                                           | GEM-1/MD | BEM-1/YD | FSEM-4/KD-1 |  |
| 5-22-1                                                       | CK                | MY      | REM-1/CD                                           | GEM-1/MD | BEM-1/YD | REM-2/KD-2  |  |
| 6-22-2                                                       | CY                | MK      | REM-1/CD                                           | GEM-1/MD | BEM-1/YD | BEM-2/KD-2  |  |
| 7-22-3                                                       | CM                | YK      | REM-1/CD                                           | GEM-1/MD | BEM-1/YD | BEM-2/KD-2  |  |

N/A is not applicable

20

## Specific Composition of the Elements

The tables below contain the detailed composition of selected elements. The specific combination of the other examples cited can be ascertained from the table above and the element below.

TABLE 6

| Reference Multilayer Element - 1 |                                                 |                           |
|----------------------------------|-------------------------------------------------|---------------------------|
| Layer/Function                   | Material                                        | Coverage g/m <sup>2</sup> |
| Protective Overcoat              | Gelatin                                         | 0.645                     |
|                                  | Dow Corning DC200™                              | 0.0202                    |
|                                  | Ludox AM™                                       | 0.1614                    |
|                                  | Di-t-octyl hydroquinone                         | 0.013                     |
|                                  | Di-n-butyl phthalate                            | 0.039                     |
|                                  | Alkanol XC™                                     | 0.009                     |
|                                  | FT-248                                          | 0.004                     |
| UV-Light Absorber-2              | Gelatin                                         | 0.624                     |
|                                  | Tinuvin 328™                                    | 0.156                     |
|                                  | Tinuvin 326™                                    | 0.027                     |
|                                  | Di-t-octyl hydroquinone                         | 0.0485                    |
|                                  | Cyclohexane-dimethanol-bis-2-ethylhexanoic acid | 0.18                      |
| Red Light Sensitive Layer C      | Di-n-butyl phthalate                            | 0.18                      |
|                                  | Gelatin                                         | 1.356                     |
|                                  | Red Sensitive Silver REM-1                      | 0.194                     |
|                                  | Coupler C-1 or C-2                              | 0.381                     |
|                                  | Di-n-butyl phthalate                            | 0.381                     |
|                                  | Tinuvin 328™                                    | 0.245                     |
|                                  | 2-(2-butoxyethoxy)ethyl acetate                 | 0.0312                    |
|                                  | Di-t-octyl hydroquinone                         | 0.0035                    |
|                                  | Dye-3                                           | 0.0665                    |
| UV-Light Absorber-1              | Gelatin                                         | 0.624                     |
|                                  | Tinuvin 328™                                    | 0.156                     |
|                                  | Tinuvin 326™                                    | 0.027                     |
|                                  | Di-t-octyl hydroquinone                         | 0.0485                    |
|                                  | Cyclohexane-dimethanol-bis-2-ethylhexanoic acid | 0.18                      |
| Green Light Sensitive Layer M    | Di-n-butyl phthalate                            | 0.18                      |
|                                  | Gelatin                                         | 1.421                     |
|                                  | Green Sensitive Silver GEM-1                    | 0.0785                    |
|                                  | Coupler M-2                                     | 0.237                     |
|                                  | Oleyl alcohol                                   | 0.0846                    |
|                                  | Di-undecyl phthalate                            | 0.0362                    |
|                                  | ST-21                                           | 0.064                     |
|                                  | ST-22                                           | 0.604                     |
|                                  | 1-Phenyl-5-mercaptopurine                       | 0.0001                    |
|                                  | Dye-2                                           | 0.0602                    |
| Interlayer                       | Gelatin                                         | 0.753                     |
|                                  | Di-t-octyl hydroquinone                         | 0.108                     |

TABLE 6-continued

| Reference Multilayer Element - 1 |                                               |                           |
|----------------------------------|-----------------------------------------------|---------------------------|
| Layer/Function                   | Material                                      | Coverage g/m <sup>2</sup> |
| 30                               | Di-n-butyl phthalate                          | 0.308                     |
|                                  | Di-sodium 4,5 Di-hydroxy-m-benzenedisulfonate | 0.0129                    |
|                                  | SF-1 (Alkanol XC™)                            | 0.0495                    |
|                                  | Irganox 1076™                                 | 0.0323                    |
| 35                               | Blue Light Sensitive Layer Y                  |                           |
|                                  | Gelatin                                       | 1.312                     |
|                                  | Blue Sensitive Silver BEM-1                   | 0.227                     |
|                                  | Coupler Y-3 or                                | 0.414                     |
|                                  | Y5                                            | 0.414                     |
|                                  | ST-23                                         | 0.186                     |
|                                  | Tri-butyl citrate                             | 0.0001                    |
|                                  | 1-Phenyl-5-mercaptopurine                     | 0.009                     |
|                                  | Dye-1                                         |                           |
| 40                               | Support                                       |                           |
|                                  | Resin Coated Color Paper Support or           |                           |
|                                  | Transparent Polymeric Support                 |                           |

TABLE 7

| Inventive Multilayer Element 1-31-1 |                                                 |                           |
|-------------------------------------|-------------------------------------------------|---------------------------|
| Layer/Function                      | Material                                        | Coverage g/m <sup>2</sup> |
| 50                                  | Protective Overcoat                             |                           |
|                                     | Gelatin                                         | 0.645                     |
|                                     | Dow Coming DC200™                               | 0.0202                    |
|                                     | Ludox AM™                                       | 0.1614                    |
|                                     | Di-t-octyl hydroquinone                         | 0.013                     |
|                                     | Di-n-butyl phthalate                            | 0.039                     |
|                                     | Alkanol XC™                                     | 0.009                     |
|                                     | FT-248                                          | 0.004                     |
| 55                                  | UV-Light Absorber-2                             |                           |
|                                     | Gelatin                                         | 0.624                     |
|                                     | Tinuvin 328™                                    | 0.156                     |
|                                     | Tinuvin 326™                                    | 0.027                     |
|                                     | Di-t-octyl hydroquinone                         | 0.0485                    |
|                                     | Cyclohexane-dimethanol-bis-2-ethylhexanoic acid | 0.18                      |
| 60                                  | Layer C Red Light Sensitive                     |                           |
|                                     | Di-n-butyl phthalate                            | 0.18                      |
|                                     | Gelatin                                         | 1.356                     |
|                                     | Red Sensitive Silver REM-1                      | 0.194                     |
|                                     | Coupler C-1 or C-2                              | 0.381                     |
|                                     | Di-n-butyl phthalate                            | 0.381                     |
|                                     | Tinuvin 328™                                    | 0.245                     |
|                                     | 2-(2-butoxyethoxy)ethyl acetate                 | 0.0312                    |
| 65                                  | Dye-3                                           | 0.0665                    |

TABLE 7-continued

| Inventive Multilayer Element 1-31-1 |                                                                      |                           |
|-------------------------------------|----------------------------------------------------------------------|---------------------------|
| Layer/Function                      | Material                                                             | Coverage g/m <sup>2</sup> |
| UV-Light Absorber-1                 | Gelatin                                                              | 0.624                     |
|                                     | Tinuvin 328™                                                         | 0.156                     |
|                                     | Tinuvin 326™                                                         | 0.027                     |
|                                     | Di-t-octyl hydroquinone                                              | 0.0485                    |
|                                     | Cyclohexane-dimethanol-bis-2-ethylhexanoic acid                      | 0.18                      |
|                                     | Di-n-butyl phthalate                                                 | 0.18                      |
|                                     | Gelatin                                                              | 1.421                     |
|                                     | Green Sensitive Silver GEM-1                                         | 0.0785                    |
|                                     | Coupler M-2                                                          | 0.237                     |
|                                     | Oleyl alcohol                                                        | 0.0846                    |
| Green Light Sensitive Layer M       | Di-undecyl phthalate                                                 | 0.0362                    |
|                                     | ST-21                                                                | 0.064                     |
|                                     | ST-22                                                                | 0.604                     |
|                                     | 1-Phenyl-5-mercaptopotetrazole                                       | 0.0001                    |
|                                     | Dye-2                                                                | 0.0602                    |
|                                     | Gelatin                                                              | 0.753                     |
|                                     | Di-t-octyl hydroquinone                                              | 0.108                     |
|                                     | Di-n-butyl phthalate                                                 | 0.308                     |
|                                     | Di-sodium 4,5 Di-hydroxy-m-benzenedi-sulfonate                       | 0.0129                    |
|                                     | SF-1 (Alkanol XC™)                                                   | 0.0495                    |
| Blue Light Sensitive Layer Y        | Irganox 1076™                                                        | 0.0323                    |
|                                     | Gelatin                                                              | 1.312                     |
|                                     | Blue Sensitive Silver BEM-1                                          | 0.227                     |
|                                     | Coupler Y-3 or Y5                                                    | 0.414                     |
|                                     | ST-23                                                                | 0.414                     |
|                                     | Tri-butyl citrate                                                    | 0.0001                    |
|                                     | 1-Phenyl-5-mercaptopotetrazole                                       | 0.009                     |
|                                     | Dye-1                                                                |                           |
|                                     | 2 to 7 mil Transparent Polymeric Support with Sub-coat on both sides |                           |
|                                     | IR Light Sensitive Layer                                             |                           |
| Antihalation Layer                  | Gelatin                                                              | 1.076                     |
|                                     | Infrared Sensitive Silver FSEM-1                                     | 0.560                     |
|                                     | Coupler K73                                                          | 0.270                     |
|                                     | N,N-diethyl lauramide                                                | 0.54                      |
|                                     | 2-(2-butoxyethoxy)ethyl acetate                                      | 0.0129                    |
|                                     | Gelatin                                                              | 1.29                      |
|                                     | Silver                                                               | 0.151                     |
|                                     | Versa TL-502™                                                        | 0.0311                    |
|                                     | Di-t-octyl hydroquinone                                              | 0.118                     |
|                                     | Di-n-butyl phthalate                                                 | 0.359                     |
| Protective Overcoat                 | Gelatin                                                              | 0.645                     |
|                                     | Dow Corning DC200™                                                   | 0.0202                    |
|                                     | Ludox AM™                                                            | 0.1614                    |
|                                     | Di-t-octyl hydroquinone                                              | 0.013                     |
|                                     | Di-n-butyl phthalate                                                 | 0.039                     |
|                                     | Alkanol XC™                                                          | 0.009                     |
|                                     | FT-248                                                               | 0.004                     |

TABLE 8

Inventive Multilayer Element 7-22-3

| Inventive Multilayer Element 7-22-3 |                         |                           |
|-------------------------------------|-------------------------|---------------------------|
| Layer/Function                      | Material                | Coverage g/m <sup>2</sup> |
| Protective Overcoat                 | Gelatin                 | 0.645                     |
|                                     | Dow Corning DC200™      | 0.0202                    |
|                                     | Ludox AM™               | 0.1614                    |
|                                     | Di-t-octyl hydroquinone | 0.013                     |
|                                     | Di-n-butyl phthalate    | 0.039                     |
|                                     | Alkanol XC™             | 0.009                     |
|                                     | FT-248                  | 0.004                     |
|                                     | Gelatin                 | 0.624                     |

TABLE 8-continued

| Inventive Multilayer Element 7-22-3 |                             |                                                                            |
|-------------------------------------|-----------------------------|----------------------------------------------------------------------------|
| Layer/Function                      | Material                    | Coverage g/m <sup>2</sup>                                                  |
| 5                                   | Absorber-2                  | Tinuvin 328™                                                               |
|                                     |                             | Tinuvin 326™                                                               |
|                                     |                             | Di-t-octyl hydroquinone                                                    |
|                                     |                             | Cyclohexane-dimethanol-bis-2-ethylhexanoic acid                            |
|                                     |                             | Di-n-butyl phthalate                                                       |
|                                     |                             | Gelatin                                                                    |
|                                     |                             | Red Sensitive Silver REM-1                                                 |
|                                     |                             | Coupler C-1 or C-2                                                         |
|                                     |                             | Di-n-butyl phthalate                                                       |
|                                     |                             | Tinuvin 328™                                                               |
| 10                                  | Layer C                     | 2-(2-butoxyethoxy)ethyl acetate                                            |
|                                     |                             | Di-t-octyl hydroquinone                                                    |
|                                     |                             | Dye-3                                                                      |
|                                     |                             | Gelatin                                                                    |
|                                     |                             | Tinuvin 328™                                                               |
|                                     |                             | 2-(2-butoxyethoxy)ethyl acetate                                            |
|                                     |                             | Di-t-octyl hydroquinone                                                    |
|                                     |                             | Dye-3                                                                      |
|                                     |                             | Gelatin                                                                    |
|                                     |                             | Tinuvin 326™                                                               |
| 15                                  | Layer M                     | Di-t-octyl hydroquinone                                                    |
|                                     |                             | Cyclohexane-dimethanol-bis-2-ethylhexanoic acid                            |
|                                     |                             | Di-n-butyl phthalate                                                       |
|                                     |                             | Gelatin                                                                    |
|                                     |                             | Red Sensitive Silver REM-1                                                 |
|                                     |                             | Coupler C-1 or C-2                                                         |
|                                     |                             | Di-n-butyl phthalate                                                       |
|                                     |                             | Tinuvin 328™                                                               |
|                                     |                             | 2-(2-butoxyethoxy)ethyl acetate                                            |
|                                     |                             | Di-t-octyl hydroquinone                                                    |
| 20                                  | UV-Light Absorber-1         | Dye-3                                                                      |
|                                     |                             | Gelatin                                                                    |
|                                     |                             | Tinuvin 328™                                                               |
|                                     |                             | 2-(2-butoxyethoxy)ethyl acetate                                            |
|                                     |                             | Di-t-octyl hydroquinone                                                    |
|                                     |                             | Cyclohexane-dimethanol-bis-2-ethylhexanoic acid                            |
|                                     |                             | Di-n-butyl phthalate                                                       |
|                                     |                             | Gelatin                                                                    |
|                                     |                             | Tinuvin 326™                                                               |
|                                     |                             | Di-t-octyl hydroquinone                                                    |
| 25                                  | Green Light Sensitive Layer | Cyclohexane-dimethanol-bis-2-ethylhexanoic acid                            |
|                                     |                             | Di-n-butyl phthalate                                                       |
|                                     |                             | Gelatin                                                                    |
|                                     |                             | Green Sensitive Silver GEM-1                                               |
|                                     |                             | Coupler M-2                                                                |
|                                     |                             | Oleyl alcohol                                                              |
|                                     |                             | Di-undecyl phthalate                                                       |
|                                     |                             | ST-21                                                                      |
|                                     |                             | ST-22                                                                      |
|                                     |                             | 1-Phenyl-5-mercaptopotetrazole                                             |
| 30                                  | Support                     | Dye-2                                                                      |
|                                     |                             | 2 to 9 mil thick Transparent Polymeric Support with Sub-coat on both sides |
|                                     |                             | Gelatin                                                                    |
|                                     |                             | BIue Sensitive Silver BEM-1                                                |
|                                     |                             | Coupler Y-3 or Y5                                                          |
|                                     |                             | ST-23                                                                      |
|                                     |                             | Tri-butyl citrate                                                          |
|                                     |                             | 1-Phenyl-5-mercaptopotetrazole                                             |
|                                     |                             | Dye-1                                                                      |
|                                     |                             | 2 to 9 mil thick Transparent Polymeric Support with Sub-coat on both sides |
| 35                                  | Blue Light Sensitive Layer  | Gelatin                                                                    |
|                                     |                             | BIue Sensitive Silver BEM-1                                                |
|                                     |                             | Coupler Y-3 or Y5                                                          |
|                                     |                             | ST-23                                                                      |
|                                     |                             | Tri-butyl citrate                                                          |
|                                     |                             | 1-Phenyl-5-mercaptopotetrazole                                             |
|                                     |                             | Dye-1                                                                      |
|                                     |                             | 2 to 9 mil thick Transparent Polymeric Support with Sub-coat on both sides |
|                                     |                             | Gelatin                                                                    |
|                                     |                             | BIue Sensitive Silver BEM-1                                                |
| 40                                  | Interlayer                  | Coupler Y-3 or Y5                                                          |
|                                     |                             | ST-23                                                                      |
|                                     |                             | Tri-butyl citrate                                                          |
|                                     |                             | 1-Phenyl-5-mercaptopotetrazole                                             |
|                                     |                             | Dye-1                                                                      |
|                                     |                             | Gelatin                                                                    |
|                                     |                             | Di-t-octyl hydroquinone                                                    |
|                                     |                             | Di-n-butyl phthalate                                                       |
|                                     |                             | Di-sodium 4,5 Di-hydroxy-m-benzenedi-sulfonate                             |
|                                     |                             | Alkanol XC™                                                                |
| 45                                  | Antihalation Layer          | Irganox 1076™                                                              |
|                                     |                             | Gelatin                                                                    |
|                                     |                             | Blue Sensitive Silver BEM-2                                                |
|                                     |                             | Coupler C-1                                                                |
|                                     |                             | Coupler M-1                                                                |
|                                     |                             | Coupler Y-13                                                               |
|                                     |                             | Di-n-butyl phthalate                                                       |
|                                     |                             | Gelatin                                                                    |
|                                     |                             | Silver                                                                     |
|                                     |                             | Versa TL-502™                                                              |
| 50                                  | Antihalation Layer          | Di-t-octyl hydroquinone                                                    |
|                                     |                             | Di-n-butyl phthalate                                                       |
|                                     |                             | Gelatin                                                                    |
|                                     |                             | Silver                                                                     |
|                                     |                             | Versa TL-502™                                                              |
|                                     |                             | Di-t-octyl hydroquinone                                                    |
|                                     |                             | Di-n-butyl phthalate                                                       |
|                                     |                             | Gelatin                                                                    |
|                                     |                             | Dow Corning DC200™                                                         |
|                                     |                             | Ludox AM™                                                                  |
| 55                                  | Protective Overcoat         | Di-t-octyl hydroquinone                                                    |
|                                     |                             | Di-n-butyl phthalate                                                       |
|                                     |                             | Gelatin                                                                    |
|                                     |                             | Dow Corning DC200™                                                         |
|                                     |                             | Ludox AM™                                                                  |
|                                     |                             | Di-t-octyl hydroquinone                                                    |
|                                     |                             | Di-n-butyl phthalate                                                       |
|                                     |                             | Alkanol XC™                                                                |
|                                     |                             | FT-248                                                                     |

## Examples 8 to 22

The following table describes the combinations of layers, emulsions, and coupler dispersions that make up the inventive 5-color duplitzied elements. The interpretation of the table is similar to that given in the examples above.

TABLE 9

5 Colorant-Duplitized Photographic Elements

| Sensitized Layers |      |         |                                                    |          |          |             |           |
|-------------------|------|---------|----------------------------------------------------|----------|----------|-------------|-----------|
| 5-Color           | Face | Reverse | Identification of Emulsion and Coupler Dispersions |          |          |             |           |
| Examples          | Side | Side    | CE/CD                                              | ME/MD    | YE/YD    | KE/KD       | XE/XD     |
| 8-41-1            | CMYK | X       | REM-1/CD                                           | GEM-1/MD | BEM-1/YD | FSEM-1/KD-1 | BEM-2/XD  |
| 9-41-2            | CMYX | K       | REM-1/CD                                           | GEM-1/MD | BEM-1/YD | FSEM-2/KD-2 | REM-2/XD  |
| 10-41-3           | CMXK | Y       | REM-1/CD                                           | GEM-1/MD | BEM-1/YD | FSEM-3/KD-1 | FSEM-1/XD |
| 11-41-4           | CYXK | M       | REM-1/CD                                           | GEM-1/MD | BEM-1/YD | BEM-2/KD-1  | FSEM-1/XD |
| 12-41-5           | MYXK | C       | REM-1/CD                                           | GEM-1/MD | BEM-1/YD | REM-2/KD-1  | FSEM-1/XD |
| 13-32-1           | CMY  | XK      | REM-1/CD                                           | GEM-1/MD | BEM-1/YD | FSEM-1/KD-2 | BEM-2/XD  |
| 14-32-2           | CMX  | YK      | REM-1/CD                                           | GEM-1/MD | BEM-1/YD | FSEM-2/KD-2 | REM-2/XD  |
| 15-32-3           | CMK  | XY      | REM-1/CD                                           | GEM-1/MD | BEM-1/YD | FSEM-3/KD-1 | BEM-2/XD  |
| 16-32-4           | CYK  | MX      | REM-1/CD                                           | GEM-1/MD | BEM-1/YD | FSEM-4/KD-1 | REM-2/XD  |
| 17-32-5           | CYX  | MK      | REM-1/CD                                           | GEM-1/MD | BEM-1/YD | BEM-2/KD-2  | FSEM-1/XD |
| 18-32-6           | CXK  | MY      | REM-1/CD                                           | GEM-1/MD | BEM-1/YD | REM-2/KD-1  | FSEM-1/XD |
| 19-32-7           | YXK  | CM      | REM-1/CD                                           | GEM-1/MD | BEM-1/YD | FSEM-1/KD-1 | REM-2/XD  |
| 20-32-8           | MYX  | CK      | REM-1/CD                                           | GEM-1/MD | BEM-1/YD | FSEM-2/KD-2 | BEM-2/XD  |
| 21-32-9           | MYK  | CX      | REM-1/CD                                           | GEM-1/MD | BEM-1/YD | FSEM-3/KD-1 | BEM-2/XD  |
| 22-32-10          | MKX  | CY      | REM-1/CD                                           | GEM-1/MD | BEM-1/YD | FSEM-4/KD-1 | REM-2/XD  |

25

TABLE 10

TABLE 10-continued

| Inventive Multilayer Element 8-41-1 |                                                 |                           | Inventive Multilayer Element 8-41-1 |                                                |                                                                            |
|-------------------------------------|-------------------------------------------------|---------------------------|-------------------------------------|------------------------------------------------|----------------------------------------------------------------------------|
| Layer/Function                      | Material                                        | Coverage g/m <sup>2</sup> | 30                                  | Layer/Function                                 | Coverage g/m <sup>2</sup>                                                  |
| Protective Overcoat                 | Gelatin                                         | 0.645                     | 35                                  | sulfonate                                      |                                                                            |
|                                     | Dow Corning DC200™                              | 0.0202                    |                                     | Alkanol XC™                                    | 0.0495                                                                     |
|                                     | Ludox AM™                                       | 0.1614                    |                                     | Irganox 1076™                                  | 0.0323                                                                     |
|                                     | Di-t-octyl hydroquinone                         | 0.013                     |                                     | Blue Light                                     |                                                                            |
|                                     | Di-n-butyl phthalate                            | 0.039                     |                                     | Gelatin                                        | 1.312                                                                      |
|                                     | Alkanol XC™                                     | 0.009                     |                                     | Blue Sensitive Silver BEM-1                    | 0.227                                                                      |
|                                     | FT-248                                          | 0.004                     |                                     | Coupler Y-3 or                                 | 0.414                                                                      |
|                                     | Gelatin                                         | 0.624                     |                                     | Y5                                             | 0.414                                                                      |
|                                     | Tinuvin 328™                                    | 0.156                     |                                     | ST-23                                          | 0.186                                                                      |
|                                     | Tinuvin 326™                                    | 0.027                     |                                     | Tri-butyl citrate                              | 0.0001                                                                     |
| UV-Light Absorber-2                 | Di-t-octyl hydroquinone                         | 0.0485                    | 40                                  | 1-Phenyl-5-mercaptopotetrazole                 | 0.009                                                                      |
|                                     | Cyclohexane-dimethanol-bis-2-ethylhexanoic acid | 0.18                      |                                     | Dye-1                                          |                                                                            |
|                                     | Di-n-butyl phthalate                            | 0.18                      |                                     | Gelatin                                        | 0.753                                                                      |
|                                     | Gelatin                                         | 1.356                     |                                     | Di-t-octyl hydroquinone                        | 0.108                                                                      |
|                                     | Red Sensitive Silver REM-1                      | 0.194                     |                                     | Di-n-butyl phthalate                           | 0.308                                                                      |
|                                     | Coupler C-1 or C-2                              | 0.381                     |                                     | Di-sodium 4,5 Di-hydroxy-m-benzenedi-sulfonate | 0.0129                                                                     |
|                                     | Di-n-butyl phthalate                            | 0.237                     |                                     | Alkanol XC™                                    | 0.0495                                                                     |
|                                     | Tinuvin 328™                                    | 0.381                     |                                     | Irganox 1076™                                  | 0.0323                                                                     |
|                                     | 2-(2-butoxyethoxy)ethyl acetate                 | 0.245                     |                                     | IR Light                                       |                                                                            |
|                                     | Di-t-octyl hydroquinone                         | 0.0312                    |                                     | Gelatin                                        | 1.076                                                                      |
| Layer C Red Light Sensitive         | Dye-3                                           | 0.0035                    |                                     | Sensitive Layer                                | Infrared Sensitive Silver FSEM-1                                           |
|                                     | Gelatin                                         | 0.0665                    |                                     | Layer K                                        | 0.560                                                                      |
|                                     | Tinuvin 328™                                    | 0.624                     |                                     | Coupler K73                                    | 0.270                                                                      |
|                                     | Tinuvin 326™                                    | 0.156                     |                                     | N,N-diethyl lauramide                          | 0.54                                                                       |
|                                     | Di-t-octyl hydroquinone                         | 0.027                     |                                     | 2-(2-butoxyethoxy)ethyl acetate                | 0.0129                                                                     |
|                                     | Cyclohexane-dimethanol-bis-2-ethylhexanoic acid | 0.0485                    |                                     | 50 Support                                     | 2 to 9 mil thick Transparent Polymeric Support with Sub-coat on both sides |
|                                     | Di-n-butyl phthalate                            | 0.18                      |                                     | Layer X                                        | Gelatin                                                                    |
|                                     | Gelatin                                         | 1.421                     |                                     | 5th Light                                      | Blue Sensitive Silver BEM-2                                                |
|                                     | Green Sensitive Silver GEM-1                    | 0.0785                    |                                     | Sensitive Layer                                | Coupler IB-1                                                               |
|                                     | Coupler M-2                                     | 0.237                     |                                     | Antihalation Layer                             | Di-n-butyl phthalate                                                       |
| UV-Light Absorber-1                 | Oleyl alcohol                                   | 0.0846                    |                                     | Gelatin                                        | 1.29                                                                       |
|                                     | Di-undecyl phthalate                            | 0.0362                    |                                     | Silver                                         | 0.151                                                                      |
|                                     | ST-21                                           | 0.064                     |                                     | 60                                             | Versa TL-502™                                                              |
|                                     | ST-22                                           | 0.604                     |                                     | Di-t-octyl hydroquinone                        | 0.118                                                                      |
|                                     | 1-Phenyl-5-mercaptopotetrazole                  | 0.0001                    |                                     | Di-n-butyl phthalate                           | 0.359                                                                      |
|                                     | Dye-2                                           | 0.0602                    |                                     | Gelatin                                        | 0.645                                                                      |
|                                     | Gelatin                                         | 0.753                     |                                     | Overcoat                                       | Dow Corning DC200™                                                         |
|                                     | Di-t-octyl hydroquinone                         | 0.108                     |                                     | Ludox AM™                                      | 0.1614                                                                     |
|                                     | Di-n-butyl phthalate                            | 0.308                     |                                     | 65                                             | Di-t-octyl hydroquinone                                                    |
|                                     | Di-sodium 4,5 Di-hydroxy-m-benzenedi-sulfonate  | 0.0129                    |                                     | Di-n-butyl phthalate                           | 0.039                                                                      |

TABLE 10-continued

| Inventive Multilayer Element 8-41-1 |             |                              |
|-------------------------------------|-------------|------------------------------|
| Layer/Function                      | Material    | Coverage<br>g/m <sup>2</sup> |
|                                     | Alkanol XC™ | 0.009                        |
|                                     | FT-248      | 0.004                        |

TABLE 11

| Inventive Multilayer Element 14-32-2 |                                                 |                           |
|--------------------------------------|-------------------------------------------------|---------------------------|
| Layer/Function                       | Material                                        | Coverage g/m <sup>2</sup> |
| Protective Overcoat                  | Gelatin                                         | 0.645                     |
|                                      | Dow Corning DC200™                              | 0.0202                    |
|                                      | Ludox AM™                                       | 0.1614                    |
|                                      | Di-t-octyl hydroquinone                         | 0.013                     |
|                                      | Di-n-butyl phthalate                            | 0.039                     |
|                                      | Alkanol XC™                                     | 0.009                     |
|                                      | FT-248                                          | 0.004                     |
|                                      | Gelatin                                         | 0.624                     |
| UV-Light Absorber-2                  | Tinuvin 328™                                    | 0.156                     |
|                                      | Tinuvin 326™                                    | 0.027                     |
|                                      | Di-t-octyl hydroquinone                         | 0.0485                    |
|                                      | Cyclohexane-dimethanol-bis-2-ethylhexanoic acid | 0.18                      |
|                                      | Di-n-butyl phthalate                            | 0.18                      |
| Layer C<br>Red Light Sensitive       | Gelatin                                         | 1.356                     |
|                                      | Red Sensitive Silver REM-1                      | 0.194                     |
|                                      | Coupler C-1 or                                  | 0.381                     |
|                                      | C-2                                             | 0.237                     |
|                                      | Di-n-butyl phthalate                            | 0.381                     |
|                                      | Tinuvin 328™                                    | 0.245                     |
|                                      | 2-(2-butoxyethoxy)ethyl acetate                 | 0.0312                    |
|                                      | Di-t-octyl hydroquinone                         | 0.0035                    |
| UV-Light Absorber-1                  | Dye-3                                           | 0.0665                    |
|                                      | Gelatin                                         | 0.624                     |
|                                      | Tinuvin 328™                                    | 0.156                     |
|                                      | Tinuvin 326™                                    | 0.027                     |
|                                      | Di-t-octyl hydroquinone                         | 0.0485                    |
| Green Light Sensitive Layer M        | Cyclohexane-dimethanol-bis-2-ethylhexanoic acid | 0.18                      |
|                                      | Di-n-butyl phthalate                            | 0.18                      |
|                                      | Gelatin                                         | 1.421                     |
|                                      | Green Sensitive Silver GEM-1                    | 0.0785                    |
|                                      | Coupler M-2                                     | 0.237                     |
| Interlayer                           | Oleyl alcohol                                   | 0.0846                    |
|                                      | Di-undecyl phthalate                            | 0.0362                    |
|                                      | ST-21                                           | 0.064                     |
|                                      | ST-22                                           | 0.604                     |
|                                      | 1-Phenyl-5-mercaptotetrazole                    | 0.0001                    |
|                                      | Dye-2                                           | 0.0602                    |
|                                      | Gelatin                                         | 0.753                     |
|                                      | Di-t-octyl hydroquinone                         | 0.108                     |
|                                      | Di-n-butyl phthalate                            | 0.308                     |
|                                      | Di-sodium 4,5 Di-hydroxy-m-benzenedi-sulfonate  | 0.0129                    |
| Alkanol XC™                          | Alkanol XC™                                     | 0.0495                    |
|                                      | Irganox 1076™                                   | 0.0323                    |

TABLE 11-continued

Inventive Multilayer Element 14-32-2

|                                 | Layer/Function                 | Material                                                                   | Coverage g/m <sup>2</sup> |
|---------------------------------|--------------------------------|----------------------------------------------------------------------------|---------------------------|
| 5                               | Layer X                        | Gelatin                                                                    | 1.421                     |
| 5 <sup>th</sup> Light Sensitive | Light Sensitive Layer          | Red Sensitive Silver REM-2 Coupler IR-7                                    | 0.0785 0.237              |
| 10                              | Layer                          | Oleyl alcohol                                                              | 0.0846                    |
|                                 |                                | Di-undecyl phthalate                                                       | 0.0362                    |
|                                 |                                | ST-21                                                                      | 0.064                     |
|                                 |                                | ST-22                                                                      | 0.604                     |
|                                 |                                | 1-Phenyl-5-mercaptopentetrazole                                            | 0.0001                    |
|                                 |                                | Dye-2                                                                      | 0.0602                    |
| 15                              | Support                        | 2 to 9 mil thick Transparent Polymeric Support with Sub-coat on both sides |                           |
|                                 | Blue Light Sensitive           | Gelatin                                                                    | 1.312                     |
|                                 | Layer Y                        | Blue Sensitive Silver BEM-1 Coupler Y-3 or                                 | 0.227 0.414               |
|                                 |                                | Y5                                                                         | 0.414                     |
| 20                              |                                | ST-23                                                                      | 0.186                     |
|                                 |                                | Tri-butyl citrate                                                          | 0.0001                    |
|                                 |                                | 1-Phenyl-5-mercaptopentetrazole                                            | 0.009                     |
|                                 |                                | Dye-1                                                                      |                           |
|                                 | Interlayer                     | Gelatin                                                                    | 0.753                     |
|                                 |                                | Di-t-octyl hydroquinone                                                    | 0.108                     |
|                                 |                                | Di-n-butyl phthalate                                                       | 0.308                     |
| 25                              |                                | Di-sodium 4,5 Di-hydroxy-m-benzenedi-sulfonate                             | 0.0129                    |
|                                 |                                | Alkanol XC™                                                                | 0.0495                    |
|                                 | Infrared Light Sensitive Layer | Irganox 1076™                                                              | 0.0323                    |
| 30                              | Layer K                        | Gelatin                                                                    | 1.076                     |
|                                 |                                | Infrared Sensitive Silver FSEM-2                                           | 0.350                     |
|                                 |                                | Coupler C-1                                                                | 0.19                      |
|                                 |                                | Coupler M-1                                                                | 0.14                      |
|                                 |                                | Coupler Y-13                                                               | 0.25                      |
|                                 |                                | Di-n-butyl phthalate                                                       | 0.240                     |
|                                 | Antihalation Layer             | Gelatin                                                                    | 1.29                      |
|                                 |                                | Silver                                                                     | 0.151                     |
| 35                              |                                | Versa TL-502™                                                              | 0.0311                    |
|                                 |                                | Di-t-octyl hydroquinone                                                    | 0.118                     |
|                                 |                                | Di-n-butyl phthalate                                                       | 0.359                     |
|                                 |                                | 1,4-Cyclohexylenedimethylene bis(2-ethylhexanoate)                         | 0.0717                    |
|                                 | Protective Overcoat            | Gelatin                                                                    | 0.645                     |
| 40                              |                                | Dow Corning DC200™                                                         | 0.0202                    |
|                                 |                                | Ludox AM™                                                                  | 0.1614                    |
|                                 |                                | Di-t-octyl hydroquinone                                                    | 0.013                     |
|                                 |                                | Di-n-butyl phthalate                                                       | 0.039                     |
|                                 |                                | Alkanol XC™                                                                | 0.009                     |
|                                 |                                | FT-248                                                                     | 0.004                     |

### Examples 23 to 3

The following table describes the combinations of layers, emulsions, and coupler dispersions that make up the inventive 6-color duplitzited elements. The interpretation of the table is similar to that given in the examples above.

TABLE 12

## 6 Colorant Duplitized Photographic Elements

## Sensitized Layers

| 6-Color Examples |       | Face Side | Reverse Side | Identification of Emulsion and Coupler Dispersions |              |              |                |              |               |
|------------------|-------|-----------|--------------|----------------------------------------------------|--------------|--------------|----------------|--------------|---------------|
|                  |       |           |              | CE/CD                                              | ME/MD        | YE/YD        | KE/KD          | XE/XD        | ZE/ZD         |
| 23-51-1          | CMYKX | Z         |              | REM-1/<br>CD                                       | GEM-1/<br>MD | BEM-1/<br>YD | REM-2/<br>KD-1 | BEM-2/<br>XD | FSEM-1/<br>ZD |

TABLE 12-continued

6 Colorant Duplitzed Photographic Elements

| 6-Color Examples | Face Side | Reverse Side | Identification of Emulsion and Coupler Dispersions |              |              |                |              |               |
|------------------|-----------|--------------|----------------------------------------------------|--------------|--------------|----------------|--------------|---------------|
|                  |           |              | CE/CD                                              | ME/MD        | YE/YD        | KE/KD          | XE/XD        | ZE/ZD         |
| 24-51-2          | CMYKZ     | X            | REM-1/<br>CD                                       | GEM-1/<br>MD | BEM-1/<br>YD | REM-2/<br>KD-1 | BEM-2/<br>XD | FSEM4/<br>ZD  |
| 25-51-3          | CMYXZ     | K            | REM-1/<br>CD                                       | GEM-1/<br>MD | BEM-1/<br>YD | REM-2/<br>KD-2 | REM-2/<br>XD | FSEM-2/<br>ZD |
| 26-51-4          | CMKXZ     | Y            | REM-1/<br>CD                                       | GEM-1/<br>MD | BEM-1/<br>YD | REM-2/<br>KD-1 | REM-2/<br>XD | FSEM-3/<br>ZD |
| 27-51-5          | CYKXZ     | M            | REM-1/<br>CD                                       | GEM-1/<br>MD | BEM-1/<br>YD | REM-2/<br>KD-1 | REM-2/<br>XD | FSEM-4/<br>ZD |
| 28-51-6          | MYXK      | C            | REM-1/<br>CD                                       | GEM-1/<br>MD | BEM-1/<br>YD | REM-2/<br>KD-1 | REM-2/<br>XD | FSEM-2/<br>ZD |
| 29-42-1          | CMYK      | XZ           | REM-1/<br>CD                                       | GEM-1/<br>MD | BEM-1/<br>YD | REM-2/<br>KD-1 | REM-2/<br>XD | FSEM-3/<br>ZD |
| 30-42-2          | CMYX      | KZ           | REM-1/<br>CD                                       | GEM-1/<br>MD | BEM-1/<br>YD | REM-2/<br>KD-2 | REM-2/<br>XD | FSEM-4/<br>ZD |
| 31-42-3          | CMKZ      | YZ           | REM-1/<br>CD                                       | GEM-1/<br>MD | BEM-1/<br>YD | REM-2/<br>KD-1 | REM-2/<br>XD | FSEM-1/<br>ZD |
| 32-42-4          | CYKX      | MZ           | REM-1/<br>CD                                       | GEM-1/<br>MD | BEM-1/<br>YD | REM-2/<br>KD-1 | REM-2/<br>XD | FSEM-2/<br>ZD |
| 33-42-5          | MYKX      | CZ           | REM-1/<br>CD                                       | GEM-1/<br>MD | BEM-1/<br>YD | REM-2/<br>KD-J | REM-2/<br>XD | FSEM-3/<br>ZD |
| 34-42-6          | CMYZ      | KX           | REM-1/<br>CD                                       | GEM-1/<br>MD | BEM-1/<br>YD | REM-2/<br>KD-2 | REM-2/<br>XD | FSEM4/<br>ZD  |
| 35-42-7          | CMKZ      | YX           | REM-1/<br>CD                                       | GEM-1/<br>MD | BEM-1/<br>YD | REM-2/<br>KD-1 | REM-2/<br>XD | FSEM-3/<br>ZD |
| 36-42-8          | CYKZ      | MX           | REM-1/<br>CD                                       | GEM-1/<br>MD | BEM-1/<br>YD | REM-2/<br>KD-1 | REM-2/<br>XD | FSEM-2/<br>ZD |
| 37-42-9          | MYKZ      | CX           | REM-1/<br>CD                                       | GEM-1/<br>MD | BEM-1/<br>YD | REM-2/<br>KD-1 | REM-2/<br>XD | FSEM-1/<br>ZD |
| 38-42-10         | CMXZ      | YK           | REM-1/<br>CD                                       | GEM-1/<br>MD | BEM-1/<br>YD | REM-2/<br>KD-2 | REM-2/<br>XD | FSEM-2/<br>ZD |
| 39-42-11         | CYXZ      | MK           | REM-1/<br>CD                                       | GEM-1/<br>MD | BEM-1/<br>YD | REM-2/<br>KD-2 | REM-2/<br>XD | FSEM-4/<br>ZD |
| 40-42-12         | MYXZ      | CK           | REM-1/<br>CD                                       | GEM-1/<br>MD | BEM-1/<br>YD | REM-2/<br>KD-2 | REM-2/<br>XD | FSEM-1/<br>ZD |
| 41-42-13         | CKXY      | MY           | REM-1/<br>CD                                       | GEM-1/<br>MD | BEM-1/<br>YD | REM-2/<br>KD-1 | REM-2/<br>XD | FSEM-1/<br>ZD |
| 42-42-14         | MKXY      | CY           | REM-1/<br>CD                                       | GEM-1/<br>MD | BEM-1/<br>YD | REM-2/<br>KD-1 | REM-2/<br>XD | FSEM-4/<br>ZD |
| 43-42-15         | YKXZ      | CM           | REM-1/<br>CD                                       | GEM-1/<br>MD | BEM-1/<br>YD | REM-2/<br>KD-1 | REM-2/<br>XD | FSEM-3/<br>ZD |
| 44-33-1          | CMY       | KXZ          | REM-1/<br>CD                                       | GEM-1/<br>MD | BEM-1/<br>YD | REM-2/<br>KD-2 | REM-2/<br>XD | FSEM-2/<br>ZD |
| 45-33-2          | CMK       | YXZ          | REM-1/<br>CD                                       | GEM-1/<br>MD | BEM-1/<br>YD | REM-2/<br>KD-1 | REM-2/<br>XD | FSEM-1/<br>ZD |
| 46-33-3          | CYK       | MXZ          | REM-1/<br>CD                                       | GEM-1/<br>MD | BEM-1/<br>YD | REM-2/<br>KD-1 | REM-2/<br>XD | FSEM4/<br>ZD  |
| 47-33-4          | MYK       | CXZ          | REM-1/<br>CD                                       | GEM-1/<br>MD | BEM-1/<br>YD | REM-2/<br>KD-1 | REM-2/<br>XD | FSEM-4/<br>ZD |
| 48-33-5          | CMX       | KYZ          | REM-1/<br>CD                                       | GEM-1/<br>MD | BEM-1/<br>YD | REM-2/<br>KD-1 | REM-2/<br>XD | FSEM4/<br>ZD  |
| 49-33-6          | CKX       | MYZ          | REM-1/<br>CD                                       | GEM-1/<br>MD | BEM-1/<br>YD | REM-2/<br>KD-1 | REM-2/<br>XD | FSEM-4/<br>ZD |
| 50-33-7          | MKX       | CYZ          | REM-1/<br>CD                                       | GEM-1/<br>MD | BEM-1/<br>YD | REM-2/<br>KD-1 | REM-2/<br>XD | FSEM-3/<br>ZD |
| 51-33-8          | CYX       | KMZ          | REM-1/<br>CD                                       | GEM-1/<br>MD | BEM-1/<br>YD | REM-2/<br>KD-1 | REM-2/<br>XD | FSEM-3/<br>ZD |
| 52-33-9          | YKX       | CMZ          | REM-1/<br>CD                                       | GEM-1/<br>MD | BEM-1/<br>YD | REM-2/<br>KD-1 | REM-2/<br>XD | FSEM-3/<br>ZD |
| 53-33-10         | CMX       | KCZ          | REM-1/<br>CD                                       | GEM-1/<br>MD | BEM-1/<br>YD | REM-2/<br>KD-1 | REM-2/<br>XD | FSEM4/<br>ZD  |

TABLE 13

| Inventive Multilayer Element 25-51-3 |                                                 |                           |
|--------------------------------------|-------------------------------------------------|---------------------------|
| Layer/Function                       | Material                                        | Coverage g/m <sup>2</sup> |
| Protective Overcoat                  | Gelatin                                         | 0.645                     |
|                                      | Dow Corning DC200™                              | 0.0202                    |
|                                      | Ludox AM™                                       | 0.1614                    |
|                                      | Di-t-octyl hydroquinone                         | 0.013                     |
|                                      | Di-n-butyl phthalate                            | 0.039                     |
|                                      | Alkanol XC™                                     | 0.009                     |
|                                      | FT-248                                          | 0.004                     |
|                                      | Gelatin                                         | 0.624                     |
|                                      | Tinuvin 328™                                    | 0.156                     |
|                                      | Tinuvin 326™                                    | 0.027                     |
| UV-Light Absorber-2                  | Di-t-octyl hydroquinone                         | 0.0485                    |
|                                      | Cyclohexane-dimethanol-bis-2-ethylhexanoic acid | 0.18                      |
|                                      | Di-n-butyl phthalate                            | 0.18                      |
|                                      | Gelatin                                         | 1.356                     |
|                                      | Red Sensitive Silver REM-1                      | 0.194                     |
|                                      | Coupler C-1 or C-2                              | 0.381                     |
|                                      | Di-n-butyl phthalate                            | 0.381                     |
|                                      | Tinuvin 328™                                    | 0.245                     |
|                                      | 2-(2-butoxyethoxy)ethyl acetate                 | 0.0312                    |
|                                      | Di-t-octyl hydroquinone                         | 0.0035                    |
| Layer C Red Light Sensitive          | Dye-3                                           | 0.0665                    |
|                                      | Gelatin                                         | 0.624                     |
|                                      | Tinuvin 328™                                    | 0.156                     |
|                                      | Tinuvin 326™                                    | 0.027                     |
|                                      | Di-t-octyl hydroquinone                         | 0.0485                    |
|                                      | Cyclohexane-dimethanol-bis-2-ethylhexanoic acid | 0.18                      |
|                                      | Di-n-butyl phthalate                            | 0.18                      |
|                                      | Gelatin                                         | 1.421                     |
|                                      | Green Sensitive Silver GEM-1                    | 0.0785                    |
|                                      | Coupler M-2                                     | 0.237                     |
| Green Light Sensitive Layer M        | Oleyl alcohol                                   | 0.0846                    |
|                                      | Di-undecyl phthalate                            | 0.0362                    |
|                                      | ST-21                                           | 0.064                     |
|                                      | ST-22                                           | 0.604                     |
|                                      | 1-Phenyl-5-mercaptopotetrazole                  | 0.0001                    |
|                                      | Dye-2                                           | 0.0602                    |
|                                      | Gelatin                                         | 0.753                     |
|                                      | Di-t-octyl hydroquinone                         | 0.108                     |
|                                      | Di-n-butyl phthalate                            | 0.308                     |
|                                      | Di-sodium 4,5 Di-hydroxy-m-benzenedi-sulfonate  | 0.0129                    |
| Blue Light Sensitive Layer Y         | Alkanol XC™                                     | 0.0495                    |
|                                      | Irganox 1076™                                   | 0.0323                    |
|                                      | Gelatin                                         | 1.312                     |
|                                      | Blue Sensitive Silver BEM-1                     | 0.227                     |
|                                      | Coupler Y-3 or Y5                               | 0.414                     |
|                                      | ST-23                                           | 0.186                     |
|                                      | Tri-butyl citrate                               | 0.0001                    |
|                                      | 1-Phenyl-5-mercaptopotetrazole                  | 0.009                     |
|                                      | Dye-1                                           | 0.0001                    |
|                                      | Gelatin                                         | 0.753                     |
| Interlayer                           | Di-t-octyl hydroquinone                         | 0.108                     |
|                                      | Di-n-butyl phthalate                            | 0.308                     |
|                                      | Di-sodium 4,5 Di-hydroxy-m-benzenedi-sulfonate  | 0.0129                    |
|                                      | Alkanol XC™                                     | 0.0495                    |
|                                      | Irganox 1076™                                   | 0.0323                    |
|                                      | Gelatin                                         | 1.421                     |
|                                      | Red Sensitive Silver REM-2                      | 0.0785                    |
|                                      | Coupler IR-7                                    | 0.237                     |
|                                      | Oleyl alcohol                                   | 0.0846                    |
|                                      | Di-undecyl phthalate                            | 0.0362                    |
| Layer X 4th Light Sensitive Layer    | ST-21                                           | 0.064                     |
|                                      | ST-22                                           | 0.604                     |
|                                      | 1-Phenyl-5-mercaptopotetrazole                  | 0.0001                    |
|                                      | Dye-2                                           | 0.0602                    |
|                                      | Gelatin                                         | 0.753                     |
|                                      | Di-t-octyl hydroquinone                         | 0.108                     |
|                                      | Di-n-butyl phthalate                            | 0.308                     |
|                                      | Di-sodium 4,5 Di-hydroxy-m-benzenedi-sulfonate  | 0.0129                    |
|                                      | Alkanol XC™                                     | 0.0495                    |
|                                      | Irganox 1076™                                   | 0.0323                    |
| Interlayer                           | Gelatin                                         | 1.421                     |
|                                      | Red Sensitive Silver REM-2                      | 0.0785                    |
|                                      | Coupler IR-7                                    | 0.237                     |
|                                      | Oleyl alcohol                                   | 0.0846                    |
|                                      | Di-undecyl phthalate                            | 0.0362                    |
|                                      | ST-21                                           | 0.064                     |
|                                      | ST-22                                           | 0.604                     |
|                                      | 1-Phenyl-5-mercaptopotetrazole                  | 0.0001                    |
|                                      | Dye-2                                           | 0.0602                    |
|                                      | Gelatin                                         | 0.753                     |

TABLE 13-continued

| Inventive Multilayer Element 25-51-3  |                                                    |                                                                            |
|---------------------------------------|----------------------------------------------------|----------------------------------------------------------------------------|
| Layer/Function                        | Material                                           | Coverage g/m <sup>2</sup>                                                  |
| 5                                     | sulfonate                                          |                                                                            |
|                                       | Alkanol XC™                                        | 0.0495                                                                     |
|                                       | Irganox 1076™                                      | 0.0323                                                                     |
|                                       | Gelatin                                            | 1.356                                                                      |
|                                       | Infrared Sensitive Silver FSEM-2                   | 0.194                                                                      |
|                                       | Coupler IB-1                                       | 0.381                                                                      |
|                                       | Di-n-butyl phthalate                               | 0.381                                                                      |
|                                       | Tinuvin 328™                                       | 0.245                                                                      |
|                                       | 2-(2-butoxyethoxy)ethyl acetate                    | 0.0312                                                                     |
|                                       | Di-t-octyl hydroquinone                            | 0.0035                                                                     |
| 10                                    | Dye-3                                              | 0.0665                                                                     |
|                                       | Support                                            | 2 to 9 mil thick Transparent Polymeric Support with Sub-coat on both sides |
|                                       | Gelatin                                            | 1.076                                                                      |
|                                       | Blue Sensitive Silver BEM-2                        | 0.350                                                                      |
|                                       | Coupler C-1                                        | 0.19                                                                       |
|                                       | Coupler M-1                                        | 0.14                                                                       |
|                                       | Coupler Y-13                                       | 0.25                                                                       |
|                                       | Di-n-butyl phthalate                               | 0.240                                                                      |
|                                       | Gelatin                                            | 1.29                                                                       |
|                                       | Silver                                             | 0.151                                                                      |
| 15                                    | Versa TL-502™                                      | 0.0311                                                                     |
|                                       | Di-t-octyl hydroquinone                            | 0.118                                                                      |
|                                       | Di-n-butyl phthalate                               | 0.359                                                                      |
|                                       | 1,4-Cyclohexylenedimethylene bis(2-ethylhexanoate) | 0.0717                                                                     |
|                                       | Gelatin                                            | 0.645                                                                      |
|                                       | Dow Corning DC200™                                 | 0.0202                                                                     |
|                                       | Ludox AM™                                          | 0.1614                                                                     |
|                                       | Di-t-octyl hydroquinone                            | 0.013                                                                      |
|                                       | Di-n-butyl phthalate                               | 0.039                                                                      |
|                                       | Alkanol XC™                                        | 0.009                                                                      |
| 20                                    | FT-248                                             | 0.004                                                                      |
|                                       | Gelatin                                            | 0.645                                                                      |
|                                       | Dow Corning DC200™                                 | 0.0202                                                                     |
|                                       | Ludox AM™                                          | 0.1614                                                                     |
|                                       | Di-t-octyl hydroquinone                            | 0.013                                                                      |
|                                       | Di-n-butyl phthalate                               | 0.039                                                                      |
|                                       | Alkanol XC™                                        | 0.009                                                                      |
|                                       | FT-248                                             | 0.004                                                                      |
|                                       | Gelatin                                            | 0.645                                                                      |
|                                       | Dow Corning DC200™                                 | 0.0202                                                                     |
| 25                                    | Ludox AM™                                          | 0.1614                                                                     |
|                                       | Di-t-octyl hydroquinone                            | 0.013                                                                      |
|                                       | Di-n-butyl phthalate                               | 0.039                                                                      |
|                                       | Alkanol XC™                                        | 0.009                                                                      |
|                                       | FT-248                                             | 0.004                                                                      |
|                                       | Gelatin                                            | 0.645                                                                      |
|                                       | Dow Corning DC200™                                 | 0.0202                                                                     |
|                                       | Ludox AM™                                          | 0.1614                                                                     |
|                                       | Di-t-octyl hydroquinone                            | 0.013                                                                      |
|                                       | Di-n-butyl phthalate                               | 0.039                                                                      |
| 30                                    | Alkanol XC™                                        | 0.009                                                                      |
|                                       | FT-248                                             | 0.004                                                                      |
|                                       | Gelatin                                            | 0.645                                                                      |
|                                       | Dow Corning DC200™                                 | 0.0202                                                                     |
|                                       | Ludox AM™                                          | 0.1614                                                                     |
|                                       | Di-t-octyl hydroquinone                            | 0.013                                                                      |
|                                       | Di-n-butyl phthalate                               | 0.039                                                                      |
|                                       | Alkanol XC™                                        | 0.009                                                                      |
|                                       | FT-248                                             | 0.004                                                                      |
|                                       | Gelatin                                            | 0.645                                                                      |
| TABLE 14                              |                                                    |                                                                            |
| Inventive Multilayer Element 38-42-10 |                                                    |                                                                            |
| Layer/Function                        | Material                                           | Coverage g/m <sup>2</sup>                                                  |
| 40                                    | Gelatin                                            | 0.645                                                                      |
|                                       | Dow Corning DC200™                                 | 0.0202                                                                     |
|                                       | Ludox AM™                                          | 0.1614                                                                     |
|                                       | Di-t-octyl hydroquinone                            | 0.013                                                                      |
|                                       | Di-n-butyl phthalate                               | 0.039                                                                      |
|                                       | Alkanol XC™                                        | 0.009                                                                      |
|                                       | FT-248                                             | 0.004                                                                      |
|                                       | Gelatin                                            | 0.624                                                                      |
|                                       | Tinuvin 328™                                       | 0.156                                                                      |
|                                       | Tinuvin 326™                                       | 0.027                                                                      |
| 45                                    | Di-t-octyl hydroquinone                            | 0.0485                                                                     |
|                                       | Cyclohexane-dimethanol-bis-2-ethylhexanoic acid    | 0.18                                                                       |
|                                       | Di-n-butyl phthalate                               | 0.18                                                                       |
|                                       | Gelatin                                            | 1.356                                                                      |
|                                       | Red Sensitive Silver REM-1                         | 0.194                                                                      |
|                                       | Coupler C-1 or C-2                                 | 0.381                                                                      |
|                                       | Di-n-butyl phthalate                               | 0.245                                                                      |
|                                       | Tinuvin 328™                                       | 0.245                                                                      |
|                                       | 2-(2-butoxyethoxy)ethyl acetate                    | 0.0312                                                                     |
|                                       | Di-t-octyl hydroquinone                            | 0.0035                                                                     |
| 50                                    | Di-n-butyl phthalate                               | 0.0665                                                                     |
|                                       | Gelatin                                            | 0.624                                                                      |
|                                       | Tinuvin 328™                                       | 0.156                                                                      |
|                                       | Tinuvin 326™                                       | 0.027                                                                      |
|                                       | Di-t-octyl hydroquinone                            | 0.0485                                                                     |
|                                       | Cyclohexane-dimethanol-bis-2-ethylhexanoic acid    | 0.18                                                                       |
|                                       | Di-n-butyl phthalate                               | 0.18                                                                       |
|                                       | Gelatin                                            | 1.356                                                                      |
|                                       | Red Sensitive Silver REM-1                         | 0.194                                                                      |
|                                       | Coupler C-1 or C-2                                 | 0.381                                                                      |
| 55                                    | Di-n-butyl phthalate                               | 0.245                                                                      |
|                                       | Tinuvin 328™                                       | 0.245                                                                      |
|                                       | 2-(2-butoxyethoxy)ethyl acetate                    | 0.0312                                                                     |
|                                       | Di-t-octyl hydroquinone                            | 0.0035                                                                     |
|                                       | Dye-3                                              | 0.0665                                                                     |
|                                       | Gelatin                                            | 0.624                                                                      |
|                                       | Tinuvin 328™                                       | 0.156                                                                      |
|                                       | Tinuvin 326™                                       | 0.027                                                                      |
|                                       | Di-t-octyl hydroquinone                            | 0.0485                                                                     |
|                                       | Cyclohexane-dimethanol-bis-2-ethylhexanoic acid    | 0.18                                                                       |
| 60                                    | Di-n-butyl phthalate                               | 0.18                                                                       |
|                                       | Gelatin                                            | 1.356                                                                      |
|                                       | Red Sensitive Silver REM-1                         | 0.194                                                                      |
|                                       | Coupler C-1 or C-2                                 | 0.381                                                                      |
|                                       | Di-n-butyl phthalate                               | 0.245                                                                      |
|                                       | Tinuvin 328™                                       | 0.245                                                                      |
|                                       | 2-(2-butoxyethoxy)ethyl acetate                    | 0.0312                                                                     |
|                                       | Di-t-octyl hydroquinone                            | 0.0035                                                                     |
|                                       | Dye-3                                              | 0.0665                                                                     |
|                                       | Gelatin                                            | 0.624                                                                      |
| 65                                    | Tinuvin 328™                                       | 0.156                                                                      |
|                                       | Tinuvin 326™                                       | 0.027                                                                      |
|                                       | Di-t-octyl hydroquinone                            | 0.0485                                                                     |
|                                       | Cyclohexane-dimethanol-bis-2-ethylhexanoic acid    | 0.18                                                                       |
|                                       | Di-n-butyl phthalate                               | 0.18                                                                       |
|                                       | Gelatin                                            | 1.356                                                                      |
|                                       | Red Sensitive Silver REM-1                         | 0.194                                                                      |
|                                       | Coupler C-1 or C-2                                 | 0.381                                                                      |
|                                       | Di-n-butyl phthalate                               | 0.245                                                                      |
|                                       | Tinuvin 328™                                       | 0.245                                                                      |

TABLE 14

TABLE 14-continued

| Inventive Multilayer Element 38-42-10 |                                                     |                                                                            |
|---------------------------------------|-----------------------------------------------------|----------------------------------------------------------------------------|
| Layer/Function                        | Material                                            | Coverage g/m <sup>2</sup>                                                  |
| Green Light Sensitive Layer M         | Gelatin                                             | 1.421                                                                      |
|                                       | Green Sensitive Silver GEM-1                        | 0.0785                                                                     |
|                                       | Coupler M-2                                         | 0.237                                                                      |
|                                       | Oleyl alcohol                                       | 0.0846                                                                     |
|                                       | Di-undecyl phthalate                                | 0.0362                                                                     |
|                                       | ST-21                                               | 0.064                                                                      |
|                                       | ST-22                                               | 0.604                                                                      |
|                                       | 1-Phenyl-5-mercaptotetrazole                        | 0.0001                                                                     |
|                                       | Dye-2                                               | 0.0602                                                                     |
|                                       | Gelatin                                             | 0.753                                                                      |
| Interlayer                            | Di-t-octyl hydroquinone                             | 0.108                                                                      |
|                                       | Di-n-butyl phthalate                                | 0.308                                                                      |
|                                       | Di-sodium 4,5 Di-hydroxy-m-benzenedi-sulfonate      | 0.0129                                                                     |
|                                       | Alkanol XC™                                         | 0.0495                                                                     |
|                                       | Irganox 1076™                                       | 0.0323                                                                     |
|                                       | Gelatin                                             | 1.421                                                                      |
|                                       | Red Sensitive Silver REM-2                          | 0.0785                                                                     |
|                                       | Coupler IR-7                                        | 0.237                                                                      |
|                                       | Oleyl alcohol                                       | 0.0846                                                                     |
|                                       | Di-undecyl phthalate                                | 0.0362                                                                     |
| Layer X 3rd Light Sensitive Layer     | ST-21                                               | 0.064                                                                      |
|                                       | ST-22                                               | 0.604                                                                      |
|                                       | 1-Phenyl-5-mercaptotetrazole                        | 0.0001                                                                     |
|                                       | Dye-2                                               | 0.0602                                                                     |
|                                       | Gelatin                                             | 0.753                                                                      |
|                                       | Di-t-octyl hydroquinone                             | 0.108                                                                      |
|                                       | Di-n-butyl phthalate                                | 0.308                                                                      |
|                                       | Di-sodium 4,5 Di-hydroxy-m-benzenedi-sulfonate      | 0.0129                                                                     |
|                                       | Alkanol XC™                                         | 0.0495                                                                     |
|                                       | Irganox 1076™                                       | 0.0323                                                                     |
| Layer Z 4th Light Sensitive Layer     | Gelatin                                             | 1.356                                                                      |
|                                       | Infrared Sensitive Silver FSEM-2                    | 0.194                                                                      |
|                                       | Coupler IB-1                                        | 0.381                                                                      |
|                                       | Di-n-butyl phthalate                                | 0.381                                                                      |
|                                       | Tinuvin 328™                                        | 0.245                                                                      |
|                                       | 2-(2-butoxyethoxy)ethyl acetate                     | 0.0312                                                                     |
|                                       | Di-t-octyl hydroquinone                             | 0.0035                                                                     |
|                                       | Dye-3                                               | 0.0665                                                                     |
|                                       | Support                                             | 2 to 9 mil thick Transparent Polymeric Support with Sub-coat on both sides |
|                                       | Gelatin                                             | 1.312                                                                      |
| Blue Light Sensitive Layer Y          | Blue Sensitive Silver BEM-1                         | 0.227                                                                      |
|                                       | Coupler Y-3 or                                      | 0.414                                                                      |
|                                       | Y5                                                  | 0.414                                                                      |
|                                       | ST-23                                               | 0.186                                                                      |
|                                       | Tri-butyl citrate                                   | 0.0001                                                                     |
|                                       | 1-Phenyl-5-mercaptotetrazole                        | 0.009                                                                      |
|                                       | Dye-1                                               |                                                                            |
|                                       | Gelatin                                             | 0.753                                                                      |
|                                       | Di-t-octyl hydroquinone                             | 0.108                                                                      |
|                                       | Di-n-butyl phthalate                                | 0.308                                                                      |
| Interlayer                            | Di-sodium 4,5 Di-hydroxy-m-benzenedi-sulfonate      | 0.0129                                                                     |
|                                       | Alkanol XC™                                         | 0.0495                                                                     |
|                                       | Irganox 1076™                                       | 0.0323                                                                     |
|                                       | Gelatin                                             | 1.076                                                                      |
|                                       | Blue Sensitive Silver BEM-2                         | 0.350                                                                      |
|                                       | Coupler C-1                                         | 0.19                                                                       |
|                                       | Coupler M-1                                         | 0.14                                                                       |
|                                       | Coupler Y-13                                        | 0.25                                                                       |
|                                       | Di-n-butyl phthalate                                | 0.240                                                                      |
|                                       | Gelatin                                             | 1.29                                                                       |
| Antihalation Layer                    | Silver                                              | 0.151                                                                      |
|                                       | Versa TL-502™                                       | 0.0311                                                                     |
|                                       | Di-t-octyl hydroquinone                             | 0.118                                                                      |
|                                       | Di-n-butyl phthalate                                | 0.359                                                                      |
|                                       | 1,4-Cyclohexylenedimethylene bis (2-ethylhexanoate) | 0.0717                                                                     |
|                                       | Gelatin                                             | 0.645                                                                      |
|                                       | Dow Corning DC200™                                  | 0.0202                                                                     |
|                                       | Ludox AM™                                           | 0.1614                                                                     |
|                                       | Di-t-octyl hydroquinone                             | 0.013                                                                      |

TABLE 14-continued

| Inventive Multilayer Element 38-42-10 |                                                 |                                                                            |
|---------------------------------------|-------------------------------------------------|----------------------------------------------------------------------------|
| Layer/Function                        | Material                                        | Coverage g/m <sup>2</sup>                                                  |
| 5                                     | Di-n-butyl phthalate                            | 0.039                                                                      |
|                                       | Alkanol XC™                                     | 0.009                                                                      |
|                                       | FT-248                                          | 0.004                                                                      |
|                                       | Gelatin                                         | 0.645                                                                      |
|                                       | Dow Corning DC200™                              | 0.0202                                                                     |
|                                       | Ludox AM™                                       | 0.1614                                                                     |
|                                       | Di-t-octyl hydroquinone                         | 0.013                                                                      |
|                                       | Di-n-butyl phthalate                            | 0.039                                                                      |
|                                       | Alkanol XC™                                     | 0.009                                                                      |
|                                       | FT-248                                          | 0.004                                                                      |
| TABLE 15                              |                                                 |                                                                            |
| Inventive Multilayer Element 44-33-1  |                                                 |                                                                            |
| Layer/Function                        | Material                                        | Coverage g/m <sup>2</sup>                                                  |
| 15                                    | Gelatin                                         | 0.624                                                                      |
|                                       | Tinuvin 328™                                    | 0.156                                                                      |
|                                       | Tinuvin 326™                                    | 0.027                                                                      |
|                                       | Di-t-octyl hydroquinone                         | 0.0485                                                                     |
|                                       | Cyclohexane-dimethanol-bis-2-ethylhexanoic acid | 0.18                                                                       |
|                                       | Di-n-butyl phthalate                            | 0.18                                                                       |
|                                       | Gelatin                                         | 1.356                                                                      |
|                                       | Red Sensitive Silver REM-1                      | 0.194                                                                      |
|                                       | Coupler C-1 or                                  | 0.381                                                                      |
|                                       | C-2                                             | 0.237                                                                      |
| 20                                    | Di-n-butyl phthalate                            | 0.381                                                                      |
|                                       | Tinuvin 328™                                    | 0.245                                                                      |
|                                       | 2-(2-butoxyethoxy)ethyl acetate                 | 0.0312                                                                     |
|                                       | Di-t-octyl hydroquinone                         | 0.0035                                                                     |
|                                       | Dye-3                                           | 0.0665                                                                     |
|                                       | Gelatin                                         | 0.624                                                                      |
|                                       | Tinuvin 328™                                    | 0.156                                                                      |
|                                       | Tinuvin 326™                                    | 0.027                                                                      |
|                                       | Di-t-octyl hydroquinone                         | 0.0485                                                                     |
|                                       | Cyclohexane-dimethanol-bis-2-ethylhexanoic acid | 0.18                                                                       |
| 30                                    | Layer C                                         |                                                                            |
|                                       | Red Light Sensitive                             |                                                                            |
|                                       | Gelatin                                         | 1.356                                                                      |
|                                       | Red Sensitive Silver REM-1                      | 0.194                                                                      |
|                                       | Coupler C-1 or                                  | 0.381                                                                      |
|                                       | C-2                                             | 0.237                                                                      |
|                                       | Di-n-butyl phthalate                            | 0.381                                                                      |
|                                       | Tinuvin 328™                                    | 0.245                                                                      |
|                                       | 2-(2-butoxyethoxy)ethyl acetate                 | 0.0312                                                                     |
|                                       | Di-t-octyl hydroquinone                         | 0.0035                                                                     |
| 35                                    | UV-Light Absorber-2                             |                                                                            |
|                                       | Dye-3                                           | 0.0665                                                                     |
|                                       | Gelatin                                         | 0.624                                                                      |
|                                       | Tinuvin 328™                                    | 0.156                                                                      |
|                                       | Tinuvin 326™                                    | 0.027                                                                      |
|                                       | Di-t-octyl hydroquinone                         | 0.0485                                                                     |
|                                       | Cyclohexane-dimethanol-bis-2-ethylhexanoic acid | 0.18                                                                       |
|                                       | Di-n-butyl phthalate                            | 0.18                                                                       |
|                                       | Gelatin                                         | 1.356                                                                      |
|                                       | Red Sensitive Silver REM-1                      | 0.194                                                                      |
| 40                                    | Layer M                                         |                                                                            |
|                                       | Red Light Sensitive                             |                                                                            |
|                                       | Gelatin                                         | 1.356                                                                      |
|                                       | Red Sensitive Silver REM-1                      | 0.194                                                                      |
|                                       | Coupler C-1 or                                  | 0.381                                                                      |
|                                       | C-2                                             | 0.237                                                                      |
|                                       | Di-n-butyl phthalate                            | 0.381                                                                      |
|                                       | Tinuvin 328™                                    | 0.245                                                                      |
|                                       | 2-(2-butoxyethoxy)ethyl acetate                 | 0.0312                                                                     |
|                                       | Di-t-octyl hydroquinone                         | 0.0035                                                                     |
| 45                                    | UV-Light Absorber-1                             |                                                                            |
|                                       | Dye-3                                           | 0.0665                                                                     |
|                                       | Gelatin                                         | 0.624                                                                      |
|                                       | Tinuvin 328™                                    | 0.156                                                                      |
|                                       | Tinuvin 326™                                    | 0.027                                                                      |
|                                       | Di-t-octyl hydroquinone                         | 0.0485                                                                     |
|                                       | Cyclohexane-dimethanol-bis-2-ethylhexanoic acid | 0.18                                                                       |
|                                       | Di-n-butyl phthalate                            | 0.18                                                                       |
|                                       | Gelatin                                         | 1.421                                                                      |
|                                       | Green Sensitive Silver GEM-1                    | 0.0785                                                                     |
| 50                                    | Layer Y                                         |                                                                            |
|                                       | Green Light Sensitive                           |                                                                            |
|                                       | Gelatin                                         | 1.421                                                                      |
|                                       | Green Sensitive Silver GEM-1                    | 0.0785                                                                     |
|                                       | Coupler M-2                                     | 0.237                                                                      |
|                                       | Oleyl alcohol                                   | 0.0846                                                                     |
|                                       | Di-undecyl phthalate                            | 0.0362                                                                     |
|                                       | ST-21                                           | 0.064                                                                      |
|                                       | ST-22                                           | 0.604                                                                      |
|                                       | 1-Phenyl-5-mercaptotetrazole                    | 0.0001                                                                     |
| 55                                    | Interlayer                                      |                                                                            |
|                                       | Dye-2                                           | 0.0602                                                                     |
|                                       | Gelatin                                         | 0.753                                                                      |
|                                       | Di-t-octyl hydroquinone                         | 0.108                                                                      |
|                                       | Di-n-butyl phthalate                            | 0.308                                                                      |
|                                       | Di-sodium 4,5 Di-hydroxy-m-benzenedi-sulfonate  | 0.0129                                                                     |
|                                       | Alkanol XC™                                     | 0.0495                                                                     |
|                                       | Irganox 1076™                                   | 0.0323                                                                     |
|                                       | Gelatin                                         | 1.076                                                                      |
|                                       | Blue Sensitive Silver BEM-2                     | 0.350                                                                      |
| 60                                    | Blue Light Sensitive                            |                                                                            |
|                                       | Gelatin                                         | 1.312                                                                      |
|                                       | Blue Sensitive Silver BEM-1                     | 0.227                                                                      |
|                                       | Coupler Y-3 or                                  | 0.414                                                                      |
|                                       | Y5                                              | 0.414                                                                      |
|                                       | ST-23                                           | 0.186                                                                      |
|                                       | Tri-butyl citrate                               | 0.0001                                                                     |
|                                       | 1-Phenyl-5-mercaptotetrazole                    | 0.009                                                                      |
|                                       | Dye-1                                           |                                                                            |
|                                       | Support                                         | 2 to 9 mil thick Transparent Polymeric Support with Sub-coat on both sides |
| 65                                    | Layer Y                                         |                                                                            |
|                                       | Gelatin                                         | 1.312                                                                      |
|                                       | Blue Sensitive Silver BEM-1                     | 0.227                                                                      |
|                                       | Coupler Y-3 or                                  | 0.414                                                                      |
|                                       | Y5                                              | 0.414                                                                      |
|                                       | ST-23                                           | 0.186                                                                      |
|                                       | Tri-butyl citrate                               | 0.0001                                                                     |
|                                       | 1-Phenyl-5-mercaptotetrazole                    | 0.009                                                                      |
|                                       | Dye-1                                           |                                                                            |
|                                       | Support                                         | 2 to 9 mil thick Transparent Polymeric Support with Sub-coat on both sides |
| 65                                    | Blue Light Sensitive                            |                                                                            |
|                                       | Gelatin                                         | 1.312                                                                      |
|                                       | Blue Sensitive Silver BEM-2                     | 0.350                                                                      |
|                                       | Coupler C-1                                     | 0.19                                                                       |
| 65                                    | Layer K                                         |                                                                            |
|                                       | Gelatin                                         | 0.414                                                                      |
|                                       | ST-23                                           | 0.186                                                                      |
|                                       | Tri-butyl citrate                               | 0.0001                                                                     |

TABLE 15-continued

Inventive Multilayer Element 44-33-1

| Layer/Function  | Material                                       | Coverage<br>g/m <sup>2</sup> |
|-----------------|------------------------------------------------|------------------------------|
| Interlayer      | Coupler Y-13                                   | 0.25                         |
|                 | Di-n-butyl phthalate                           | 0.240                        |
|                 | Gelatin                                        | 0.753                        |
|                 | Di-t-octyl hydroquinone                        | 0.108                        |
|                 | Di-n-butyl phthalate                           | 0.308                        |
|                 | Di-sodium 4,5 Di-hydroxy-m-benzenedi-sulfonate | 0.0129                       |
| Layer X         | Alkanol XC™                                    | 0.0495                       |
|                 | Irganox 1076™                                  | 0.0323                       |
| 4th Light       | Gelatin                                        | 1.421                        |
| Sensitive Layer | Red Sensitive Silver REM-2                     | 0.0785                       |
| Interlayer      | Coupler IR-7                                   | 0.237                        |
|                 | Oleyl alcohol                                  | 0.0846                       |
|                 | Di-undecyl phthalate                           | 0.0362                       |
|                 | ST-21                                          | 0.064                        |
|                 | ST-22                                          | 0.604                        |
|                 | 1-Phenyl-5-mercaptotetrazole                   | 0.0001                       |
|                 | Dye-2                                          | 0.0602                       |
|                 | Gelatin                                        | 0.753                        |
|                 | Di-t-octyl hydroquinone                        | 0.108                        |
|                 | Di-n-butyl phthalate                           | 0.308                        |
| Interlayer      | Di-sodium 4,5 Di-hydroxy-m-benzenedi-sulfonate | 0.0129                       |
|                 | Alkanol XC™                                    | 0.0495                       |
|                 | Irganox 1076™                                  | 0.0323                       |

TABLE 15-continued

Inventive Multilayer Element 44-33-1

| Layer/Function            | Material                                               | Coverage<br>g/m <sup>2</sup> |
|---------------------------|--------------------------------------------------------|------------------------------|
| Layer Z                   | Gelatin                                                | 1.356                        |
| 5th Light Sensitive Layer | Infrared Sensitive Silver FSEM-2                       | 0.194                        |
| Sensitive Layer           | Coupler IB-1                                           | 0.381                        |
|                           | Di-n-butyl phthalate                                   | 0.381                        |
|                           | Tinuvin 328™                                           | 0.245                        |
|                           | 2-(2-butoxyethoxy)ethyl acetate                        | 0.0312                       |
|                           | Di-t-octyl hydroquinone                                | 0.0035                       |
|                           | Dye-3                                                  | 0.0665                       |
| Antihalation Layer        | Gelatin                                                | 1.29                         |
|                           | Silver                                                 | 0.151                        |
|                           | Versa TL-502™                                          | 0.0311                       |
|                           | Di-t-octyl hydroquinone                                | 0.118                        |
|                           | Di-n-butyl phthalate                                   | 0.359                        |
|                           | 1,4-Cyclohexylenedimethylene bis<br>(2-ethylhexanoate) | 0.0717                       |
| Protective                | Gelatin                                                | 0.645                        |
| Overcoat                  | Dow Corning DC200™                                     | 0.0202                       |
|                           | Ludox AM™                                              | 0.1614                       |
|                           | Di-t-octyl hydroquinone                                | 0.013                        |
|                           | Di-n-butyl phthalate                                   | 0.039                        |
|                           | Alkanol XC™                                            | 0.009                        |
|                           | FT-248                                                 | 0.004                        |

C.1



6-3



-continued

M-1



M-2



Y-3



Y-5



BSD-2



-continued

BSD-4



DYE-1



DYE-2



DYE-3



DYE-4



-continued

DYE-5



GSD-1



GSD-2



IRSD-1



IRSD-2



IRSD-3



-continued



IRSD-4



RSD-1



ST-6



ST-8



ST-16



ST-21

-continued



ST-23



ST-22



SF-1



512



UV 1



JIV 3



UV-2

The invention has been described in detail with particular reference to certain preferred embodiments thereof, but it will be understood that variations and modifications can be effected within the spirit and scope of the invention.

What is claimed is:

- What is claimed is:

and photosensitive silver halide containing layers on the face side of said sheet, wherein said at least three photosensitive forming coupler and photosensitive silver halide containing layers comprise a cyan dye forming layer comprising a cyan dye forming coupler in combination with a red sensitized photosensitive emulsion, a yellow dye forming layer comprising a yellow dye forming coupler in combination with a

blue light sensitive photosensitive emulsion, a magenta dye forming layer comprising a magenta dye forming coupler and a green light sensitive photosensitive emulsion, and on the backside of said translucent polymer sheet at least one dye forming coupler and photosensitive silver halide containing layer that forms at least one dye that is spectrally distinct from the dyes on the face side of said translucent sheet.

2. The imaging element of claim 1 wherein said spectrally distinct dye is black.

3. The imaging element of claim 1 wherein said spectrally distinct dye is red, wherein said red has a CIELAB hue angle,  $h_{ab}$ , from not less than 355 to not more than 75 degrees.

4. The imaging element of claim 1 wherein said spectrally distinct dye is blue, wherein said blue has a CIELAB hue angle,  $h_{ab}$ , from 225 to 310 degrees.

5. The imaging element of claim 1 wherein said spectrally distinct at least one dye comprises red dye and blue dye, wherein said blue has a CIELAB hue angle,  $h_{ab}$ , from 225 to 310 degrees and wherein said red has a CIELAB hue angle,  $h_{ab}$ , from not less than 355 to not more than 75 degrees.

6. The imaging element of claim 1 wherein said translucent polymer sheet comprises polyester.

7. The imaging element of claim 1 wherein said translucent polymer sheet comprises at least one sheet of oriented polyolefin polymer.

8. The imaging element of claim 1 further comprising a photosensitive layer adhesion promoting layer contacting each side of translucent polymer sheet.

9. The imaging element of claim 1 wherein said translucent polymer sheet comprises UV radiation absorbing material.

10. The imaging element of claim 1 further comprising a tone enhancing layer comprising between 200 and 10,000 mg/m<sup>2</sup> of titanium dioxide on the backside of said translucent polymer sheet.

11. The imaging element of claim 1 further comprising an antihalation layer comprising gray silver or solid particle dye dispersion on the backside of said translucent sheet.

12. A method of forming an image comprising providing an imaging element comprising a translucent polymer sheet, and at least three photosensitive dye forming coupler and photosensitive silver halide containing layers on the face side of said sheet, wherein said at least three photosensitive forming coupler and photosensitive silver halide containing layers comprise a cyan dye forming layer comprising a cyan dye forming coupler in combination with a red sensitized photosensitive emulsion, a yellow dye forming layer comprising a yellow dye forming coupler in combination with a blue light sensitive photosensitive emulsion, a magenta dye forming layer comprising a magenta dye forming coupler and a green light sensitive photosensitive emulsion, and on the backside of said translucent polymer sheet at least one dye forming coupler and photosensitive silver halide containing layer that forms at least one dye that is spectrally distinct from the dyes on the face side of said translucent sheet, image wise exposing said imaging element by actinic radiation, and developing an image.

13. The method of claim 12 further comprising applying an environmental protective layer to at least one surface of the developed image.

14. The method of claim 12 wherein said actinic radiation comprises collimated beams.

15. The method of claim 12 wherein said developed image is placed in a transmission light frame.

16. The method of claim 12 wherein said element further comprises a tone enhancing layer comprising between 200 and 10,000 mg/m<sup>2</sup> of titanium dioxide on the backside of said translucent polymer sheet.

17. The method of claim 12 wherein said element further comprises an antihalation layer comprising gray silver or solid particle dye dispersion on the backside of said translucent sheet.

\* \* \* \* \*